



US005098611A

**United States Patent** [19]

Honda et al.

[11] Patent Number: **5,098,611**[45] Date of Patent: **Mar. 24, 1992**

[54] **ELECTRICAL RESISTORS, ELECTRICAL RESISTOR PASTE AND METHOD FOR MAKING THE SAME**

[75] Inventors: **Toshimitsu Honda; Tadahiko Yamada; Kazuji Onikata; Shoichi Tosaka**, all of Gumma, Japan

[73] Assignee: **Taiyo Yuden Co., Ltd.**, Tokyo, Japan

[21] Appl. No.: **457,291**

[22] Filed: **Dec. 26, 1989**

**Related U.S. Application Data**

[62] Division of Ser. No. 138,439, Dec. 28, 1987.

**Foreign Application Priority Data**

Feb. 28, 1987 [JP] Japan ..... 62-45615  
Feb. 28, 1987 [JP] Japan ..... 62-45619  
Apr. 30, 1987 [JP] Japan ..... 62-104415  
Apr. 30, 1987 [JP] Japan ..... 62-104416

[51] Int. Cl.<sup>5</sup> ..... **H01B 1/06**

[52] U.S. Cl. ..... **252/518; 252/520; 252/521; 338/20**

[58] Field of Search ..... **252/518, 520; 338/20, 338/22, 308; 427/216, 217, 126.1, 126.2; 138/439; 264/61, 60; 419/61, 64, 65; 420/429**

[56] **References Cited**

**U.S. PATENT DOCUMENTS**

4,891,158 1/1990 Hatu ..... 252/518  
4,940,849 7/1990 Monis et al. ..... 252/518

Primary Examiner—Josephine Barr

Attorney, Agent, or Firm—Birch, Stewart, Kolasch & Birch

[57] **ABSTRACT**

A fixed chip resistor or a thick-film electrical resistor provided in circuit boards and the like and, an electrical resistor obtained by sintering in a non-oxidizing atmosphere, resistance pastes for producing an electrical resistor and a method for making such resistors. The aforesaid objects are achieved by the provision of an electrical resistor obtained using at least one molybdate belonging to the following groups (A) and (G) and glass,

- (A) Molybdates of alkaline earth metals,
- (B) Molybdate of zinc,
- (C) Molybdate of elements, Y, La, Ce, Pr, Nd, Sm, Eu, Gd, Tb, Dy, Ho, Er, Tm, Yb and Lu, and complex molybdates of two or more of said elements,
- (D) Molybdates of aluminum
- (E) Molybdates of elements zirconium and hafnium, and complex molybdates thereof,
- (F) Molybdates of elements niobium and tantalum, and complex molybdates thereof, and
- (G) Molybdates of manganese.

**18 Claims, 5 Drawing Sheets**



FIG. 1



FIG. 2



**FIG. 3****FIG. 4****FIG. 5**

## FIG. 6

## X-RAY DIFFRACTION PATTERN

- PEAKS INHERENT IN  $\text{MgMoO}_4$
- PEAK INHERENT IN  $\text{CaF}_2$



## X-RAY DIFFRACTION PATTERN

**FIG. 7**



X 900,000

FIG. 8



X 900000

**ELECTRICAL RESISTORS, ELECTRICAL  
RESISTOR PASTE AND METHOD FOR MAKING  
THE SAME**

This application is a divisional of copending application Ser. No. 07/138,439 filed on Dec. 28, 1987.

**BACKGROUND OF THE INVENTION**

1. Field of the Invention

The present invention relates to a fixed chip resistor or a thick-film type electrical resistor provided in circuit boards and the like and, more particularly, to an electrical resistor capable of being obtained by sintering in a non-oxidizing atmosphere. The present invention also relates to a method for making such resistors.

2. Statement of the Prior Art

Electrical circuits of electronic equipment are generally constructed by mounting various electrical elements such as resistors, capacitors, diodes and transistors to circuit boards. With miniaturization of electronic equipment, however, much use has been made of circuit boards capable of increasing the density of such mounted electrical elements.

The resistors mounted to such circuit board include a thick-film resistor formed by printing and firing a paste of a resistor material directly onto a circuit, a fixed chip resistor made by forming such a thick-film resistor across a pair of electrode terminals of a rectangular ceramic chip, and the like.

Hitherto, such a thick-film resistor has generally been formed on a circuit board in the following manner. A paste of a conductor material such as Ag or Ag-Pd is applied and fired on the surface of an alumina substrate obtained by sintering at, e.g., about 1500° C. Afterwards, a paste containing, e.g., RuO<sub>2</sub> as the main material of the resistor is applied on that surface by means of screen printing, etc., followed by firing at 750° to 850° C. and, if required, adjustment of a resistance value by means of laser trimming, etc.

However, recent heavy demands for reductions in the weight, thickness, size and cost of electronic equipment, etc. have led to intensive studies for reducing in the size and cost of circuit boards.

Referring to concrete measures to meet the former size reduction, multilayered circuit boards deserve the first mention, and formed resistors the second mention. Known examples of multilayered circuit boards include a multilayered circuitry board obtained by laminating ceramic green sheets, each having a paste of a conductor material such as Ag or Ag-Pd printed thereon, and simultaneously sintering them at 800° to 1100° C. in the air, while known examples of the formed resistor include a multilayered with a formed resistor, obtained by printing a paste of a RuO<sub>2</sub> base resistor material on a ceramic green sheet having said paste of a conductive material printed thereon, laminating such sheets, and then simultaneously sintering them.

Referring to concrete measures to achieve the latter cost reduction, multilayered circuitry boards have been put to practical use, and are obtained by using conductive materials based on inexpensive base metals such as Ni or Cu in place of those based on noble metals such as Ag or Ag-Pd, and sintering them simultaneously with green ceramic at 800° to 1100° C. in a neutral or reducing atmosphere to avoid any increase in resistance due to their oxidation, such as a nitrogen gas or a hydrogen-containing nitrogen gas. As disclosed in Japanese Patent

Laid-Open (Kokai) Publication No. 56-153702 in particular, there are also known thick-film resistors, etc. which are obtained by applying a resistor material comprising MoSi<sub>2</sub>-TaSi<sub>2</sub> and glass on an alumina substrate including a copper (Cu) conductor, followed by a heat treatment.

Where it is intended to simultaneously reduce the size and cost of circuit boards, the RuO<sub>2</sub> base resistor material undergoes a reducing reaction, when it is sintered simultaneously with green ceramic in a nitrogen gas or hydrogen-containing nitrogen atmosphere, and it does not provide any resistor.

Simultaneous sintering of the resistor material comprising MoSi<sub>2</sub>-TaSi<sub>2</sub> and glass and the green ceramic sheet in a non-oxidizing atmosphere also offers the problems that the substrate may warp due to a difference in the dislocation shrinkage curve, or may tend to swell easily due to the gas generated by the decomposing reaction of MoSi<sub>2</sub>-TaSi<sub>2</sub>. To solve such problems, it is known by way of example to use a resistor material comprising MoSi<sub>2</sub>-salts of metal fluorides (e.g., calcium fluoride) and glass, as disclosed in Japanese Patent Laid-Open (Kokai) Publication No. 60-198703. In this example, such warping or swelling of the substrate as mentioned above is not found.

However, when allowed to stand alone in a relative humidity of 95% for 1000 hours, the thick-film resistor obtained by applying such a resistor material comprising MoSi<sub>2</sub>-metal fluorides and glass on a green ceramic sheet and simultaneously sintering them shows a 5 to 10% increase in the resistance value and, hence, cannot perform its own resistor function.

Further, the conventional electrical resistors as mentioned above have posed some problem, when used as the resistor element for a circuit needing precise work, since it is impossible to decrease the temperature dependence coefficient of their resistance value to 1000 ppm/°C. or lower.

**SUMMARY OF THE INVENTION**

A first object of the present invention is to provide an electrical resistor which can be used as a fixed chip resistor or for general circuit boards, and can also be laminated with a conductive material of a base metal and formed in a multilayered substrate.

A second object of the present invention is to provide an electrical resistor, the resistance value of which is stabilized.

A third object of the present invention is to provide an electrical resistor, in which the temperature coefficient of resistance value can be decreased.

A fourth object of the present invention is to provide an electrical resistor having excellent properties, which can be obtained even by sintering a resistor material in a reducing atmosphere.

A fifth object of the present invention is to provide an electrical resistor which can meet the reductions in both the size and cost of circuit substrates.

A sixth object of the present invention is to provide a method for making said electrical resistors, which can realize the performance thereof and further improve the properties thereof.

According to the present invention, the aforesaid objects are achieved by the provision of an electrical resistor obtained using at least one molybdate selected from the group consisting of (A) to (G) with or without a fluoride of an alkaline earth metal, and an electrical

resistor paste obtained using the aforesaid components with or without a carbonate of an alkaline earth metal:

- (A) Molybdates of alkaline earth metals,
- (B) Molybdate of zinc,
- (C) Molybdates of elements Y, La, Ce, Pr, Nd, Sm, Eu, Tb, Dy, Ho, Er, Tm, Yb and Lu, and complex molybdates of two or more of said elements,
- (D) Molybdate of aluminium
- (E) Molybdates of elements zirconium and hafnium, and complex molybdates thereof, and
- (G) Molybdates of manganese.

According to the present invention, there is also provided a method for making electrical resistors which have their properties improved by using a heat-treated resistor material, and an electrical resistor of the particulate structure obtained by the growth of acicular particles from bulk particles so as to improve its properties.

#### BRIEF DESCRIPTION OF THE DRAWINGS

The aforesaid and other objects and features of the present invention will become apparent from the following detailed description with reference to the accompanying drawings, which are given for the purpose of illustration alone, and in which:

FIG. 1 is a schematical view showing the structure of the electrical resistor according to the present invention;

FIG. 2 is a view of one embodiment of the production of the electrical resistor according to the present invention, in which a resistive film and a conductive are applied on a substrate, and are being formed into a multilayered structure, prior to sintering;

FIG. 3 is a sectional view of that sintered body taken on line III—III;

FIG. 4 is a sectional view of a sintered body of a multilayered structure obtained using a conventional resistor material;

FIG. 5 is a view further illustrating that sintered body which is evolving gas;

FIG. 6 is an X-ray diffraction pattern, where the corresponding molybdate is detected from the electrical resistor of Sample No. 1 according to the example of the present invention;

FIG. 7 is a TEM 900,000 times enlargement photograph showing the structure of the electrical resistor, and

FIG. 8 is a TEM 900,000 times enlargement photograph showing the structure of the electrical resistor obtained by using the resistor material without the fluoride and the carbonate in the resistor material in FIG. 7.

#### DETAILED DESCRIPTION OF THE INVENTION

As illustrated as an example in FIG. 1, the electrical resistor according to the present invention is of the structure wherein spherical particles b and acicular particles c are dispersed throughout glass a. In this example, the acicular particles are deposited to the spherical particles, or are allowed to be present in the vicinity thereof. A current may pass through such a structure formed by contacting particles or particles in the vicinity thereof. For instance, such a structure may be formed by the sintering treatment of bulk particles of a resistor material, thereby growing the products formed on the surfaces thereof in the acicular form.

As such a resistor body material, at least one molybdate group selected from the group consisting of (A) to (G) may be used. For example, mentioned are the following molybdates are representative of the invention.

##### (A) Molybdates of Alkaline Earth Metals

Preferable molybdates to this end are expressed in terms of the following general formulae:



wherein Me is the alkaline earth metal. For example, the following groups may be mentioned: e.g.,  $\text{MgMoO}_4$ ,  $\text{CaMoO}_4$ ,  $\text{SrMoO}_4$ ,  $\text{BaMoO}_4$ ,  $\text{BaMo}_2\text{O}_7$ ,  $\text{BaMo}_4\text{O}_{13}$ ,  $\text{BaMo}_7\text{O}_{24}$ ,  $\text{BaMo}_3\text{O}_{10}$ ,  $\text{Ca}_3\text{MoO}_8$ ,  $\text{Sr}_3\text{MoO}_6$ ,  $\text{Ba}_3\text{MoO}_6$ ,  $\text{Ba}_2\text{MoO}_5$ ,  $\text{Mg}_2\text{Mo}_3\text{O}_{11}$  and the like.

The following complex molybdates are also exemplified.



##### (B) Molybdates of Zinc

For instance,  $\text{ZnMoO}_4$ ,  $\text{ZnMo}_2\text{O}_7$ ,  $\text{Zn}_3\text{Mo}_2\text{O}_9$  are mentioned.

##### (C) Molybdates of Elements Y, La, Ce, Pr, Nd, Sm, Eu, Gd, Tb, Dy, Ho, Er, Tm, Yb and Lu and Complex Molybdates of Two or More of Said Elements

Examples of such molybdates are tabulated in the following table.

| Molybdates of Various Elements and Complex Molybdates thereof |                                      |                                       |                           |                                       |                                          |
|---------------------------------------------------------------|--------------------------------------|---------------------------------------|---------------------------|---------------------------------------|------------------------------------------|
| $\text{Y}_6\text{MoO}_{12}$                                   | $\text{Y}_2\text{Mo}_3\text{O}_{12}$ | $\text{La}_6\text{MoO}_{12}$          | $\text{La}_2\text{MoO}_6$ | $\text{Y}_2\text{MoO}_5$              | $\text{Y}_4\text{MoO}_9$                 |
|                                                               |                                      |                                       |                           | $\text{La}_2\text{Mo}_2\text{O}_9$    | $\text{La}_3\text{Mo}_2\text{O}_{10}$    |
|                                                               |                                      |                                       |                           | $\text{La}_4\text{MoO}_9$             | $\text{La}_2\text{Mo}_4\text{O}_{15}$    |
|                                                               |                                      |                                       |                           | $\text{CeMo}_2\text{O}_8$             | $\text{Ce}_2\text{Mo}_3\text{O}_{13}$    |
| $\text{Ce}_6\text{MoO}_{12}$                                  | $\text{Pr}_6\text{MoO}_{12}$         | $\text{Pr}_2\text{Mo}_3\text{O}_{12}$ | $\text{Pr}_2\text{MoO}_6$ |                                       |                                          |
|                                                               |                                      |                                       |                           | $\text{Nd}_2\text{MoO}_6$             | $\text{Nd}_5\text{Mo}_3\text{O}_{16}$    |
|                                                               |                                      |                                       |                           | $\text{Sm}_2\text{MoO}_6$             | $\text{Sm}_2\text{Mo}_2\text{O}_7$       |
|                                                               |                                      |                                       |                           | $\text{Sm}_2\text{Mo}_2\text{O}_7$    | $\text{Sm}_{18}\text{Mo}_4\text{O}_{39}$ |
|                                                               |                                      |                                       |                           | $\text{Eu}_2\text{MoO}_6$             | $\text{Eu}_2\text{Mo}_2\text{O}_7$       |
|                                                               |                                      |                                       |                           | $\text{Eu}_2\text{MoO}_4$             |                                          |
|                                                               |                                      |                                       |                           | $\text{Gd}_2\text{MoO}_6$             | $\text{Gd}_2\text{Mo}_4\text{O}_{15}$    |
|                                                               |                                      |                                       |                           | $\text{Gd}_2\text{Mo}_6\text{O}_{21}$ |                                          |
|                                                               |                                      |                                       |                           | $\text{Tb}_2\text{MoO}_6$             | $\text{Tb}_2\text{Mo}_2\text{O}_9$       |
|                                                               |                                      |                                       |                           | $\text{Tb}_2\text{Mo}_6\text{O}_6$    |                                          |
|                                                               |                                      |                                       |                           | $\text{Dy}_2\text{MoO}_6$             |                                          |
|                                                               |                                      |                                       |                           | $\text{Ho}_2\text{MoO}_6$             | $\text{Ho}_{10}\text{Mo}_2\text{O}_{21}$ |
|                                                               |                                      |                                       |                           | $\text{Er}_2\text{MoO}_6$             |                                          |
|                                                               |                                      |                                       |                           | $\text{Tm}_2\text{MoO}_6$             |                                          |

-continued

| Molybdates of Various Elements and Complex Molybdates thereof          |                                                                                                    |  |                                                |
|------------------------------------------------------------------------|----------------------------------------------------------------------------------------------------|--|------------------------------------------------|
| Yb <sub>6</sub> MoO <sub>12</sub><br>Lu <sub>6</sub> MoO <sub>12</sub> | Yb <sub>2</sub> Mo <sub>4</sub> O <sub>15</sub><br>Lu <sub>2</sub> Mo <sub>3</sub> O <sub>12</sub> |  | Lu <sub>2</sub> Mo <sub>2</sub> O <sub>9</sub> |

The following complex molybdates of two or more elements are also mentioned.

(Y<sub>x</sub>Ce<sub>y</sub>)MoO<sub>12</sub>, provided that x+y=6,  
(Pr<sub>x</sub>Ey<sub>y</sub>)MoO<sub>12</sub>, provided that x+y=6,  
(Gd<sub>x</sub>Dy<sub>y</sub>)MoO<sub>12</sub>, provided that x+y=6,  
(Ho<sub>x</sub>Tm<sub>y</sub>Yb<sub>z</sub>)MoO<sub>12</sub>, provided that x+y+z=6.

(D) Molybdates of Aluminium

For instance, Al<sub>2</sub>Mo<sub>3</sub>O<sub>12</sub> is mentioned.

(E) Molybdates of Elements Zirconium and Hafnium, and Molybdates of Said Elements

For instance, ZrMo<sub>2</sub>O<sub>3</sub>, HfMo<sub>2</sub>O<sub>8</sub> and (Zr<sub>x</sub>Hf<sub>y</sub>)Mo<sub>2</sub>O<sub>3</sub>, provided that x+y=1, are mentioned.

(F) Molybdates of Elements Niobium and Tantalum

For instance, Nb<sub>2</sub>Mo<sub>3</sub>O<sub>14</sub>, Ta<sub>2</sub>Mo<sub>3</sub>O<sub>14</sub> and (Nb<sub>x</sub>Ta<sub>y</sub>)Mo<sub>3</sub>O<sub>14</sub>, provided that x+y=1, are mentioned.

(G) Molybdates of Manganese

For instance, MnMoO<sub>4</sub> is mentioned.

For use, at least one molybdate is selected from at least one molybdate group selected from the groups (A) to (G). When plural molybdates are selected from said at least one molybdate group, however, the single molybdates and/or complex molybdates of elements may be used.

The molybdates belonging to the aforesaid respective groups can be synthesized by the heat treatment of the oxides of the respective elements and molybdenum oxide (MoO<sub>3</sub>), but may be synthesized by the heat treatment of their precursors. For instance, the molybdates of alkaline earth metals may also be synthesized by mixing substances which provide the precursors of the respective oxides of alkaline earth metals with molybdenum oxide (MoO<sub>3</sub>) or its precursor in the predetermined molar ratio and heat-treating the resulting mixture. As an example, calcium carbonate (CaCO<sub>3</sub>) or calcium hydroxide [Ca(OH)<sub>2</sub>] which is, for instance, the precursor of CaO is mixed with molybdenum oxide (MoO<sub>3</sub>) or its precursor, for instance, molybdcic acid (H<sub>2</sub>MoO<sub>4</sub>) in the predetermined molar ratio, and the mixture is heat-treated. The heat-treatment conditions in this case are 600° to 1000° C. and 1 to 3 hours.

In the present invention, glass is preferably used. As such glass, use may be made of glass generally known in the art. Although the present invention is not limited to glass having a specific composition, it is to be noted that oxides such as Pb<sub>3</sub>O<sub>4</sub>, Bi<sub>2</sub>O<sub>3</sub>, SnO<sub>2</sub> and CdO may be reduced to metals which are likely to change the resistance value of resistors, when resistor materials containing them are sintered in a non-oxidizing atmosphere. Accordingly, where such a phenomenon is unpreferred, it is preferred that the glass used should not contain such oxides.

Preferable as the glass components are SiO<sub>2</sub>, B<sub>2</sub>O<sub>3</sub>, ZnO, CaO, SrO, ZrO<sub>2</sub> and the like. It is preferred that the compositional ratio of such oxides are:

SiO<sub>2</sub>: 12 to 33% by weight

B<sub>2</sub>O<sub>3</sub>: 20 to 35% by weight

ZnO or SrO: 13 to 33% by weight

CaO: 10 to 25% by weight

ZrO<sub>2</sub>: 15 to 45% by weight.

To make glass from the compositions of such oxides, the respective oxides are weighed and mixed together in the aforesaid compositional ratio. The mixture is charged in a crucible, in which it is molten at a temperature of 1200° to 1500° C. Thereafter, the melt is poured in, e.g., water for rapid cooling, and the thus obtained coarse glass powders are pulverized to the desired particle size (of, e.g., 10 µm or less) by a pulverizer such as a ball mill or vibration mill to obtain glass powders.

The precursors of the respective oxides may wholly or partly be used and molten into glass. For instance, CaO (calcium oxide) and B<sub>2</sub>O<sub>3</sub> (boron oxide) are obtained by the heat treatment of CaCO<sub>3</sub> (calcium carbonate) and boric acid (H<sub>3</sub>BO<sub>3</sub>), respectively. Hence, CaCO<sub>3</sub> and H<sub>2</sub>BO<sub>3</sub> may be used in place of the whole or a part of CaO and B<sub>2</sub>O<sub>3</sub>. The same also holds for other componential oxides.

25 The fluorides of alkaline earth metals used in the present invention are expressed in terms of the general formula:



wherein Me' is the metal. As Me', use is made of alkaline earth metals, i.e., Mg, Ca, Sr and Ba. The respective salts of these metals may preferably be used alone or in admixture. In the present invention, however, the fluorides of other metals may also be used in addition to those of alkaline earth metals.

The molybdates of the elements belonging to said element groups and the glass powders obtained in the aforesaid manner are mixed together with or without the fluorides of alkaline earth metals, etc., and the mixtures may be used directly as resistor materials. In view of the resistance temperature properties of resistors, however, it is preferred to heat-treat and pulverize such mixtures and sinter the thus pulverized bodies as the resistor materials. The temperature for this heat treatment is preferably 800° to 1200° C. At a temperature departing from such a temperature range, the resistance value of the resulting resistors are apt to be influenced by delicate variations in the compositional ratio, which 50 are caused by the operational conditions for the respective steps of processing the resistor materials into the electrical resistors. As a consequence, it is difficult to stably obtain the desired resistance value.

The heat treatment is desirously effected in a non-oxidizing atmosphere. To this end, use is preferably made of nitrogen gas or other inert gas, which may or may not contain hydrogen gas.

To prepare a fixed chip resistor or a resistor for thick-film resistors from the thus obtained resistor material powders, the powders are applied on, e.g., a ceramic green sheet, and the resulting product is sintered. In this case, for instance, the aforesaid molybdate forming the resistor body is preferably used in the form of bulk particles such as spherical, oval or polygonal particles.

65 This is because it is preferable to allow the original matrixes of the acicular particles to remain in the process of the growth of the acicular particles during sintering. In order to form such a resistor body material

into bulk particles, a binder such as glass may also be used.

For the purpose of applying such a resistor material comprising a molybdate and e.g., glass, a vehicle is mixed with the powders of such a resistor material so as to enable, e.g., screen printing. Prepared in this case, however, is a coating liquid to which a carbonate of an alkaline earth metal is added.

Such a carbonate may be expressed in terms of the general formula:



wherein  $\text{Me}''$  is preferably but not exclusively the alkaline earth metal such as Mg, Ca, Sr and Ba. However, carbonates of other metals may be used.

Although varying dependent upon the type and combination of the molybdates of the elements selected from the groups (A) to (G) as already referred to, the compositional ratio of the respective components of the resistor materials should preferably be within the following range, when one or plural molybdates are selected from the same group.

| Group                             | Preferred Composition in weight % |        |        |        |        |        |        |
|-----------------------------------|-----------------------------------|--------|--------|--------|--------|--------|--------|
|                                   | A                                 | B      | C      | D      | E      | F      | G      |
| Molybdate                         | 40-95                             | 65-95  | 60-95  | 45-95  | 50-95  | 55-95  | 65-95  |
| Glass Powders                     | 4-59                              | 4-34   | 4-39   | 4-54   | 4-49   | 4-44   | 4-34   |
| Fluoride of Alkaline Earth Metal  | 0.5-25                            | 0.5-20 | 0.5-10 | 0.5-20 | 0.5-15 | 0.5-15 | 0.5-15 |
| Carbonate of Alkaline Earth Metal | 0.5-50                            | 0.5-30 | 0.5-25 | 0.5-25 | 0.5-45 | 0.5-40 | 0.5-25 |

Otherwise, when at least one molybdate is selected from at least one molybdate group of the groups (A) to

5 exceeding excessively the upper limit of the defined range are unpreferred, since the resistance value of the electrical resistor completed by sintering may become too high. On the contrary, when the amount of the said molybdate is too large and the amount of glass is too small, the binder ability of materials at the time of sintering may drop to such a degree that it is impossible to stably retain the sintered body on a circuit substrate. It is to be noted, however, that when the resistor is for 10 instance laminated on and embedded in a circuit substrate, the molybdate and the fluoride of an alkaline earth metal may be used in an amount of not only higher than their upper limits but also 100%.

An amount of the fluoride of an alkaline earth metal 15 either exceeding excessively the upper limit or short excessively of the lower limit may also be unpreferred, since the temperature dependence coefficient of the finished electrical resistor exceeds  $\pm 500 \text{ ppm}/^\circ\text{C}$ . (the absolute value of  $\pm 500$  is larger than 500), when the 20 carbonate of an alkaline earth metal is present, the value may be made not to exceed  $\pm 300 \text{ ppm}/^\circ\text{C}$ .

It is further noted that when it is not intended to use both the carbonate and fluoride of an alkaline earth

metal, it is preferable to apply the following compositional ratio.

| Group         | Preferred Composition in weight % |       |       |       |       |       |       |
|---------------|-----------------------------------|-------|-------|-------|-------|-------|-------|
|               | A                                 | B     | C     | D     | E     | F     | G     |
| Molybdate     | 30-96                             | 55-95 | 50-96 | 35-96 | 40-96 | 45-96 | 50-96 |
| Glass Powders | 4-70                              | 4-45  | 4-50  | 4-65  | 4-60  | 4-55  | 4-50  |

(G) as already referred to, preferred compositions are composed of 34.8 to 95.0% by weight of the molybdate, 2.1 to 49.5% by weight of glass powders, 0.3 to 29.9% by weight of the fluoride of an alkaline earth metal and 0.3 to 33.3% by weight of the carbonate of an alkaline earth metal.

It is noted that when the carbonate of an alkaline earth metal is not used, it is preferable to apply the following compositional ratio.

Otherwise, it is to be understood, however, that when 45 at least one molybdate is selected from each of at least two groups of the aforesaid groups (A) to (G), preferred compositions are composed of 50-96% by weight of the molybdate and 4 to 50% by weight of the glass powders.

It is to be noted, however, that the fluorides of an 50 alkaline earth metal and the carbonate of an alkaline earth metal may be used in an amount of departing from

| Group                            | Preferred Composition in weight % |          |          |        |          |          |          |
|----------------------------------|-----------------------------------|----------|----------|--------|----------|----------|----------|
|                                  | A                                 | B        | C        | D      | E        | F        | G        |
| Molybdate                        | 30-95                             | 60-95    | 55-95    | 40-95  | 40-95    | 50-95    | 55-95    |
| Glass Powders                    | 4.5-69.5                          | 4.5-39.5 | 4.5-44.5 | 4.5-59 | 4.5-54.5 | 4.5-49.5 | 4.5-44.5 |
| Fluoride of Alkaline Earth Metal | 0.5-40                            | 0.5-20   | 0.3-30   | 0.5-30 | 0.5-20   | 0.5-25   | 0.3-30   |

Otherwise, it is to be understood, however, that when 60 at least one molybdate is selected from each of at least two groups of the aforesaid groups (A) to (G), preferred compositions are composed of 35.0 to 95.6% by weight of the molybdate, 2.8 to 49.9% by weight of the glass powders and 0.5 to 30.0% by weight of the fluoride of an alkaline earth metal.

An amount of the molybdate short excessively of the lower limit of the defined range and an amount of glass

the defined range, if improvements in the temperature dependence coefficient of resistance is achieved.

Preferably, the aforesaid vehicle should be burned off 65 anywhere prior to sintering. Preferable to this end are organic vehicles, i.e., in which resins are dissolved or dispersed in organic solvents, if required, with the addition of various additives such as plasticizers and disper-

sants. Examples of the organic solvents include butyl carbitol acetate, butyl carbitol and turpentine oil, whilst examples of the resins include cellulose derivatives such as ethyl cellulose and nitrocellulose and other resins.

Although the proportion of the organic vehicles with the resistor material powders varies depending upon, e.g., the organic solvents and resins used, the ratio of the organic solvents to the resins to be applied should suitably be in a range of 20 to 50% by weight of the former with respect to 80 to 50% by weight of the latter. These components are pasted with the resistor material by three-roll milling.

The thus obtained resistor material paste is applied on a substrate, and is further subjected to the treatments to be described later to make a resistor. The substrate may be prepared not only by sintering a ceramic green sheet along with a conductive material and a resistor material, but also by previously sintering a ceramic green sheet and applying thereon a resistor material and a conductor material, followed by sintering. Such procedures may also be applied to the formation of laminates.

As the aforesaid ceramic green sheet, use may be made of that obtained by slip-casting a slurry, etc., said slurry being prepared by mixing the organic vehicle with an oxide mixture of ceramic constituents comprising, for instance, 35 to 45% by weight of aluminium oxide ( $Al_2O_3$ ), 25 to 35% by weight of silicon oxide ( $SiO_2$ ), 10 to 15% by weight of boron oxide ( $B_2O_3$ ), 7 to 13% by weight of calcium oxide ( $CaO$ ) and 7 to 10% by weight of magnesium oxide ( $MgO$ ). In this case, when the molybdate of the aforesaid groups is not used with glass, an increased amount of a glassy component may be contained in the aforesaid ceramic green sheet so as to achieve an effect similar to that achieved by the use of glass. The aforesaid organic vehicles may be comprised of acrylic resins such as acryl ester, resins such as polyvinyl butyral, plasticizers such as glycerin and diethyl phthalate, dispersants such as carbonates, and solvents such as organic solvents.

It is preferred that the aforesaid resistive material paste is applied on the ceramic green sheet by means of, e.g., screen printing and, after drying, is heat-treated at 400° to 500° C. to decompose and burn the resinous component.

In this case, a paste of a conductive material of a base metal such as Ni or Cu or a noble metal such as Ag or Ag-Pd is also simultaneously applied on the ceramic green sheet in the same manner.

The paste compositions of the conductive material of a base metal such as Ni or Cu or a noble metal such as 50 Ag or Ag-Pd are exemplified by those obtained by adding 2 to 15% by weight of glass frits to 98 to 85% by weight of the powders of the respective metals.

The resistor material and/or the conductive material are/is incorporated into the ceramic green sheet in this manner. In the case of a fixed chip resistor, by this sintering it is possible to form the conductive material and/or the thick-film resistor material simultaneously into/on the substrates. On the other hand, in the case of the laminate, another similar ceramic green sheet is further put thereon, and after repeating this process, the multilayered board is sintered.

When the conductor material of a base metal such as Ni or Cu is used as the conductor material in this case, sintering should preferably be carried out in a nonoxidizing atmosphere so as to prevent any increase in the resistance value due to its oxidation. The sintering temperature is exemplified by, e.g., 800° to 1100° C., and the

sintering time is exemplified by, e.g., 0.5 to 2 hours. A nitrogen gas or other inert gases which may or may not contain a hydrogen gas may be used as the nonoxidizing atmosphere. When the conductor material of a noble metal such as Ag or Ag-Pd is used, on the other hand, sintering may be carried out in an oxidizing atmosphere of air, for instance.

The circuitry substrate having the conductor and/or resistor incorporated thereinto is completed in the manner as mentioned above. According to the present invention, however, any cracking, distortion, swelling, etc., which may be caused by sintering, are not found in the sintered substrate and the resistor, to say nothing of in the sintered substrate and the conductor, and the resistor shows a resistance value change within only  $\pm 0.1\%$  with respect to changes in a relative humidity of 10 to 90% at 25° C. Further, even after the resistor has been allowed to stand for at least 1000 hours in a high-temperature and-humidity atmosphere, the change in its resistance value is limited to within  $\pm 2\%$ , and the temperature-dependent coefficient of its resistance value in the case of using the fluorides can be reduced not to exceed  $\pm 500$  ppm/°C., while that in the case of using the fluorides and carbonates not to exceed  $\pm 300$  ppm/°C. Such effects appear to be due to the fact that the resistor is well matched with the conductor and the sintered substrate and on the basis of the unique humidity resistance of the resistor comprising the sintered body comprised of the molybdate of the aforesaid groups and glass; however, details thereon are not yet clarified. By X-ray diffraction analysis, the resistor has been found to contain the molybdate. Also, the presence of the bulk and acicular particles has been observed under a transmission type electron microscope (TEM).

In the present invention, the molybdates selected as mentioned above may be used; however, the whole or a part of the precursors of such molybdates may be used in place thereof by a heat treatment. In either case, it is preferable that they are mixed with glass and heat-treated, and the resulting product is pulverized into a resistor material. Alternatively, the molybdates and/or their precursors may be mixed with the aforesaid vehicles, etc. without any heat treatment to prepare a paste, which is applied on, e.g., a ceramic green sheet, heat-treated for the removal of the organics, and is thereafter sintered directly into a resistor.

Referring to the glass used, it is to be understood that the mixed material of the oxides forming it may result in a sinterable state with the molybdate selected. The whole or a part of such oxides is put to a pasty state together with the molybdate selected and/or its precursor. The paste is then applied on the substrate, and the aforesaid glassy components are formed into glass in the process of either one of the steps of burning off the organics and the later sintering step. The glass is sintered with the molybdate selected and/or its precursor to thereby prepare a resistor. For instance, since  $CaO$  (calcium oxide) and  $B_2O_3$  (boron oxide) that are the components of glass materials may be obtained from  $CaCO_3$  (calcium carbonate) and  $H_3BO_3$  (boric acid) by heating,  $HCO_3$  and  $H_3BO_3$  may be used in place of the whole or a part of  $CaO$  and  $B_2O_3$ , respectively. By the resistor material referred to in the present disclosure is meant a material which may be comprised of the molybdate selected, the glass and the fluoride of an alkaline earth metal as a result of the treating processes involved.

## EXAMPLES

The present invention will now be explained with reference to the following non-restrictive examples.

## EXAMPLE 1

The respective components were weighed and mixed together according in the compositional ratio calculated as oxides and specified in Table 1.

TABLE 1

|         | Compositional Ratio in % by Weight |                               |      |      |      |                  |
|---------|------------------------------------|-------------------------------|------|------|------|------------------|
|         | SiO <sub>2</sub>                   | B <sub>2</sub> O <sub>3</sub> | ZnO  | CaO  | SrO  | ZrO <sub>2</sub> |
| Glass A | 20.0                               | 29.0                          | 13.0 | 10.0 | 11.0 | 17.0             |
| Glass B | 18.0                               | 28.5                          | 20.2 | 10.5 | —    | 23.0             |

The respective mixtures of Glass A and Glass B were separately molten in alumina crucibles at 1400° C., and

the obtained melts were poured in water for rapid cooling. The thus cooled products were taken out of the water, and were milled together with ethanol, and were pulverized by alumina balls into glass powders having a particle size of 10  $\mu\text{m}$  or lower.

The respective molybdates belonging to the aforesaid groups (A) to (G) were synthesized from molybdenum oxide and the oxides of the respective elements. However, the molybdate of an alkaline earth metal was prepared by mixing molybdenum oxide with the carbonate of an alkaline earth metal in a molar ratio of 1:1 and heat-treating the mixture at 700° C. for 1 hour.

The powders obtained from each of Glass A and Glass B, the aforesaid molybdates and the fluorides of alkaline earth metals were weighed and mixed together in the proportions specified in the respective columns of Tables 2-9.

TABLE 2

| Nos.                                              | Molybdates<br>(wt. %) | (Ex. 1)(Group A)<br>Composition |                       |                      |                  |                  |                   | Carbonates<br>(wt. %) |                   |                   |    |
|---------------------------------------------------|-----------------------|---------------------------------|-----------------------|----------------------|------------------|------------------|-------------------|-----------------------|-------------------|-------------------|----|
|                                                   |                       | Glass<br>A<br>(wt. %)           | Glass<br>B<br>(wt. %) | Fluorides<br>(wt. %) |                  |                  | SrCO <sub>3</sub> | BaCO <sub>3</sub>     | MgCO <sub>3</sub> | CaCO <sub>3</sub> |    |
|                                                   |                       |                                 |                       | SrF <sub>2</sub>     | BaF <sub>2</sub> | MgF <sub>2</sub> |                   |                       |                   |                   |    |
| <u>MgMoO<sub>4</sub></u>                          |                       |                                 |                       |                      |                  |                  |                   |                       |                   |                   |    |
| 1                                                 | 25                    | 58.4                            | —                     |                      |                  |                  | 8.3               | 8.3                   |                   |                   |    |
| 2                                                 | 41.7                  | 41.7                            | —                     |                      |                  |                  | 8.3               | 8.3                   |                   |                   |    |
| 3                                                 | 62.5                  | 20.9                            | —                     |                      |                  |                  | 8.3               | 8.3                   |                   |                   |    |
| 4                                                 | 80                    | 3.4                             | —                     |                      |                  |                  | 8.3               | 8.3                   |                   |                   |    |
| 5                                                 | 41.7                  | —                               | 41.7                  |                      |                  |                  | 8.3               | 8.3                   |                   |                   |    |
| 6                                                 | 62.5                  | —                               | 20.9                  |                      |                  |                  | 8.3               | 8.3                   |                   |                   |    |
| 7                                                 | 40                    | —                               | 59                    |                      |                  |                  | 0.5               |                       |                   | 0.5               |    |
| 8                                                 | 40                    | —                               | 5                     |                      |                  |                  | 5                 |                       |                   | 50                |    |
| 9                                                 | 60                    | —                               | 5                     |                      |                  |                  | 30                |                       |                   | 5                 |    |
| 10                                                | 60                    | —                               | 20                    |                      |                  |                  | 10                |                       |                   | 10                |    |
| 11                                                | 80                    | —                               | 10                    |                      |                  |                  | 5                 |                       |                   | 5                 |    |
| 12                                                | 80                    | —                               | 7                     |                      |                  |                  | 3                 |                       |                   | 10                |    |
| 13                                                | 95                    | —                               | 4                     |                      |                  |                  | 0.5               |                       |                   | 0.5               |    |
| 14                                                | 40                    | —                               | 59                    | 0.5                  |                  |                  |                   | 0.5                   |                   |                   |    |
| 15                                                | 40                    | —                               | 5                     | 5                    |                  |                  |                   | 50                    |                   |                   |    |
| 16                                                | 60                    | —                               | 5                     | 30                   |                  |                  |                   | 5                     |                   |                   |    |
| 17                                                | 60                    | —                               | 20                    | 10                   |                  |                  |                   | 10                    |                   |                   |    |
| 18                                                | 80                    | —                               | 10                    | 5                    |                  |                  |                   | 5                     |                   |                   |    |
| 19                                                | 80                    | —                               | 7                     | 3                    |                  |                  |                   | 10                    |                   |                   |    |
| 20                                                | 95                    | —                               | 4                     | 0.5                  |                  |                  |                   | 0.5                   |                   |                   |    |
| 21                                                | 60                    | —                               | 20                    |                      |                  |                  | 10                |                       |                   |                   | 10 |
| 22                                                | 80                    | —                               | 7                     |                      |                  |                  | 3                 |                       |                   |                   | 10 |
| 23                                                | 60                    | —                               | 20                    |                      |                  |                  | 10                | 10                    |                   |                   |    |
| 24                                                | 80                    | —                               | 7                     |                      |                  |                  | 3                 | 10                    |                   |                   |    |
| 25                                                | 60                    | —                               | 20                    |                      |                  |                  | 10                |                       | 10                |                   |    |
| 26                                                | 80                    | —                               | 7                     |                      |                  |                  | 3                 |                       | 10                |                   |    |
| 27                                                | 60                    | —                               | 10                    |                      |                  | 20               |                   |                       |                   | 10                |    |
| 28                                                | 80                    | —                               | 10                    |                      |                  | 5                |                   |                       |                   | 5                 |    |
| 29                                                | 60                    | —                               | 10                    | 20                   |                  |                  |                   |                       |                   | 10                |    |
| 30                                                | 80                    | —                               | 10                    | 5                    |                  |                  |                   |                       |                   | 5                 |    |
| 31                                                | 60                    | —                               | 10                    |                      | 20               |                  |                   |                       |                   | 10                |    |
| 32                                                | 80                    | —                               | 10                    |                      | 5                |                  |                   |                       |                   | 5                 |    |
| 33                                                | 40                    | —                               | 5                     | 2                    | 2                | 1                |                   |                       | 25                |                   | 25 |
| 34                                                | 60                    | —                               | 20                    | 5                    | 5                |                  | 3                 | 3                     |                   |                   | 4  |
| <u>Mg<sub>2</sub>Mo<sub>3</sub>O<sub>11</sub></u> |                       |                                 |                       |                      |                  |                  |                   |                       |                   |                   |    |
| 35                                                | 25                    | —                               | 58.4                  |                      |                  |                  | 8.3               | 8.3                   |                   |                   |    |
| 36                                                | 41.7                  | —                               | 41.7                  |                      |                  |                  | 8.3               | 8.3                   |                   |                   |    |
| 37                                                | 62.5                  | —                               | 20.9                  |                      |                  |                  | 8.3               | 8.3                   |                   |                   |    |
| 38                                                | 80                    | —                               | 3.4                   |                      |                  |                  | 8.3               | 8.3                   |                   |                   |    |
| 39                                                | 41.7                  | 41.7                            | —                     |                      |                  |                  | 8.3               | 8.3                   |                   |                   |    |
| 40                                                | 62.5                  | 20.9                            | —                     |                      |                  |                  | 8.3               | 8.3                   |                   |                   |    |
| 41                                                | 40                    | —                               | 59                    | 0.5                  |                  |                  |                   |                       |                   | 0.5               |    |
| 42                                                | 30                    | —                               | 5                     | 5                    |                  |                  |                   |                       |                   | 50                |    |
| 43                                                | 60                    | —                               | 5                     | 30                   |                  |                  |                   |                       |                   | 5                 |    |
| 44                                                | 60                    | —                               | 20                    | 10                   |                  |                  |                   |                       |                   | 10                |    |
| 45                                                | 80                    | —                               | 10                    | 5                    |                  |                  |                   |                       |                   | 5                 |    |
| 46                                                | 80                    | —                               | 7                     | 3                    |                  |                  |                   |                       |                   | 10                |    |
| 47                                                | 95                    | —                               | 4                     | 0.5                  |                  |                  |                   |                       |                   | 0.5               |    |
| 48                                                | 60                    | —                               | 20                    | 10                   |                  |                  |                   |                       |                   | 10                |    |
| 49                                                | 80                    | —                               | 7                     | 3                    |                  |                  |                   |                       |                   | 10                |    |
| 50                                                | 60                    | —                               | 20                    | 10                   |                  |                  |                   | 10                    |                   |                   |    |
| 51                                                | 80                    | —                               | 7                     | 3                    |                  |                  |                   | 10                    |                   |                   |    |
| 52                                                | 60                    | —                               | 20                    | 10                   |                  |                  |                   |                       | 10                |                   |    |

TABLE 2-continued

| Nos. | (Ex. 1)(Group A)<br>Composition      |                                                   |            |         |                  |                  |                      |                  |                   |                       |                   |                   |
|------|--------------------------------------|---------------------------------------------------|------------|---------|------------------|------------------|----------------------|------------------|-------------------|-----------------------|-------------------|-------------------|
|      | Molybdates                           |                                                   | Glass<br>A |         | Glass<br>B       |                  | Fluorides<br>(wt. %) |                  |                   | Carbonates<br>(wt. %) |                   |                   |
|      | (wt. %)                              | (wt. %)                                           | (wt. %)    | (wt. %) | SrF <sub>2</sub> | BaF <sub>2</sub> | MgF <sub>2</sub>     | CaF <sub>2</sub> | SrCO <sub>3</sub> | BaCO <sub>3</sub>     | MgCO <sub>3</sub> | CaCO <sub>3</sub> |
| 53   | 80                                   |                                                   |            |         | 7                | 3                |                      |                  |                   | 10                    |                   |                   |
| 54   | 60                                   | —                                                 | —          | 10      |                  |                  | 20                   |                  |                   |                       | 10                |                   |
| 55   | 80                                   | —                                                 | —          | 10      |                  |                  | 5                    |                  |                   |                       | 5                 |                   |
| 56   | 60                                   | —                                                 | —          | 10      |                  |                  |                      | 20               |                   |                       | 10                |                   |
| 57   | 80                                   | —                                                 | —          | 10      |                  |                  |                      | 5                |                   |                       | 5                 |                   |
| 58   | 60                                   | —                                                 | —          | 10      |                  | 20               |                      |                  |                   |                       | 10                |                   |
| 59   | 80                                   | —                                                 | —          | 10      |                  | 5                |                      |                  |                   |                       | 5                 |                   |
| 60   | 40                                   | —                                                 | —          | 5       | 2                |                  | 1                    | 2                |                   | 25                    | 25                |                   |
| 61   | 60                                   | —                                                 | —          | 20      | 5                |                  | 5                    | 3                | 3                 |                       | 4                 |                   |
|      | <u>MgMoO<sub>4</sub></u>             | <u>Mg<sub>2</sub>Mo<sub>3</sub>O<sub>11</sub></u> |            |         |                  |                  |                      |                  |                   |                       |                   |                   |
| 62   | 40                                   | 40                                                | 3.4        |         |                  |                  |                      |                  | 8.3               | 8.3                   |                   |                   |
| 63   | 30                                   | 30                                                | —          | 20      | 2.5              | 2.5              | 2.5                  | 2.5              | 2.5               | 2.5                   | 2.5               |                   |
|      | <u>CaMoO<sub>4</sub></u>             |                                                   |            |         |                  |                  |                      |                  |                   |                       |                   |                   |
| 64   | 25                                   | —                                                 | 58.4       | —       |                  |                  |                      |                  | 8.3               | 8.3                   |                   |                   |
| 65   | 41.7                                 | —                                                 | 41.7       | —       |                  |                  |                      |                  | 8.3               | 8.3                   |                   |                   |
| 66   | 62.5                                 | —                                                 | 20.9       | —       |                  |                  |                      |                  | 8.3               | 8.3                   |                   |                   |
| 67   | 80                                   | —                                                 | 3.4        | —       |                  |                  |                      |                  | 8.3               | 8.3                   |                   |                   |
| 68   | 41.7                                 | —                                                 | 41.7       | —       |                  |                  |                      |                  | 8.3               | 8.3                   |                   |                   |
| 69   | 62.5                                 | —                                                 | 20.9       | —       |                  |                  |                      |                  | 8.3               | 8.3                   |                   |                   |
| 70   | 40                                   | —                                                 | 59         | 0.5     |                  |                  |                      |                  |                   |                       | 0.5               |                   |
| 71   | 40                                   | —                                                 | 5          | 5       |                  |                  |                      |                  |                   |                       | 50                |                   |
| 72   | 60                                   | —                                                 | 5          | 30      |                  |                  |                      |                  |                   |                       | 5                 |                   |
| 73   | 60                                   | —                                                 | 20         | 10      |                  |                  |                      |                  |                   |                       | 10                |                   |
| 74   | 80                                   | —                                                 | 10         | 5       |                  |                  |                      |                  |                   |                       | 5                 |                   |
| 75   | 80                                   | —                                                 | 7          | 3       |                  |                  |                      |                  |                   |                       | 10                |                   |
| 76   | 95                                   | —                                                 | 4          | 0.5     |                  |                  |                      |                  |                   |                       | 0.5               |                   |
| 77   | 40                                   | —                                                 | 59         | —       |                  |                  |                      | 0.5              | 0.5               |                       |                   |                   |
| 78   | 40                                   | —                                                 | 5          | —       |                  |                  |                      | 5                | 50                |                       |                   |                   |
| 79   | 60                                   | —                                                 | 5          | —       |                  |                  |                      | 30               | 5                 |                       |                   |                   |
| 80   | 60                                   | —                                                 | 20         | —       |                  |                  |                      | 10               | 10                |                       |                   |                   |
| 81   | 80                                   | —                                                 | 10         | —       |                  |                  |                      | 5                | 5                 |                       |                   |                   |
| 82   | 80                                   | —                                                 | 7          | —       |                  |                  |                      | 3                | 10                |                       |                   |                   |
| 83   | 95                                   | —                                                 | 4          | —       |                  |                  |                      | 0.5              | 0.5               |                       |                   |                   |
| 84   | 60                                   | —                                                 | 20         | 10      |                  |                  |                      |                  |                   | 10                    |                   |                   |
| 85   | 80                                   | —                                                 | 7          | 3       |                  |                  |                      |                  |                   | 10                    |                   |                   |
| 86   | 60                                   | —                                                 | 20         | 10      |                  |                  |                      |                  | 10                |                       |                   |                   |
| 87   | 80                                   | —                                                 | 7          | 3       |                  |                  |                      |                  | 10                |                       |                   |                   |
| 88   | 60                                   | —                                                 | 20         | 10      |                  |                  |                      |                  |                   | 10                    |                   |                   |
| 89   | 80                                   | —                                                 | 7          | 3       |                  |                  |                      |                  |                   | 10                    |                   |                   |
| 90   | 60                                   | —                                                 | 10         | —       |                  |                  | 20                   |                  |                   |                       | 10                |                   |
| 91   | 80                                   | —                                                 | 10         | —       |                  |                  | 5                    |                  |                   |                       | 5                 |                   |
| 92   | 60                                   | —                                                 | 10         | —       |                  |                  |                      | 20               |                   |                       | 10                |                   |
| 93   | 80                                   | —                                                 | 10         | —       |                  |                  |                      | 5                |                   |                       | 5                 |                   |
| 94   | 60                                   | —                                                 | 10         | —       |                  |                  | 20                   |                  |                   |                       | 10                |                   |
| 95   | 80                                   | —                                                 | 10         | —       |                  |                  | 5                    |                  |                   |                       | 5                 |                   |
| 96   | 40                                   | —                                                 | 5          | —       |                  |                  | 2                    | 1                | 2                 | 25                    | 25                |                   |
| 97   | 60                                   | —                                                 | 20         | —       |                  |                  | 5                    | 5                | 3                 | 3                     | 4                 |                   |
|      | <u>Ca<sub>2</sub>MoO<sub>6</sub></u> |                                                   |            |         |                  |                  |                      |                  |                   |                       |                   |                   |
| 98   | 25                                   | —                                                 | 58.4       | —       |                  |                  |                      |                  | 8.3               | 8.3                   |                   |                   |
| 99   | 41.7                                 | —                                                 | 41.7       | —       |                  |                  |                      |                  | 8.3               | 8.3                   |                   |                   |
| 100  | 62.5                                 | —                                                 | 20.9       | —       |                  |                  |                      |                  | 8.3               | 8.3                   |                   |                   |
| 101  | 80                                   | —                                                 | 3.4        | —       |                  |                  |                      |                  | 8.3               | 8.3                   |                   |                   |
| 102  | 41.7                                 | 41.7                                              | —          | —       |                  |                  |                      |                  | 8.3               | 8.3                   |                   |                   |
| 103  | 62.5                                 | 20.9                                              | —          | —       |                  |                  |                      |                  | 8.3               | 8.3                   |                   |                   |
| 104  | 40                                   | —                                                 | 59         | —       |                  |                  | 0.5                  |                  |                   |                       | 0.5               |                   |
| 105  | 30                                   | —                                                 | 5          | —       |                  |                  | 5                    |                  |                   |                       | 50                |                   |
| 106  | 60                                   | —                                                 | 5          | —       |                  |                  | 30                   |                  |                   |                       | 5                 |                   |
| 107  | 60                                   | —                                                 | 20         | —       |                  |                  | 10                   |                  |                   |                       | 10                |                   |
| 108  | 80                                   | —                                                 | 10         | —       |                  |                  | 5                    |                  |                   |                       | 5                 |                   |
| 109  | 80                                   | —                                                 | 7          | —       |                  |                  | 3                    |                  |                   |                       | 10                |                   |
| 110  | 95                                   | 4                                                 | —          | —       |                  |                  | 0.5                  |                  |                   |                       | 0.5               |                   |
| 111  | 60                                   | 20                                                | —          | —       |                  |                  | 10                   |                  |                   |                       | 10                |                   |
| 112  | 80                                   | 7                                                 | —          | —       |                  |                  | 3                    |                  |                   |                       | 10                |                   |
| 113  | 60                                   | 20                                                | —          | —       |                  |                  | 10                   |                  |                   | 10                    |                   |                   |
| 114  | 80                                   | —                                                 | 7          | —       |                  |                  | 3                    |                  |                   | 10                    |                   |                   |
| 115  | 60                                   | 20                                                | —          | —       |                  |                  | 10                   |                  |                   | 10                    |                   |                   |
| 116  | 80                                   | 7                                                 | —          | —       |                  |                  | 3                    |                  |                   | 10                    |                   |                   |
| 117  | 60                                   | —                                                 | 10         | —       |                  |                  | 20                   |                  |                   |                       | 10                |                   |
| 118  | 80                                   | —                                                 | 10         | —       |                  |                  | 5                    |                  |                   |                       | 5                 |                   |
| 119  | 60                                   | —                                                 | 10         | —       |                  |                  |                      | 20               |                   |                       | 10                |                   |
| 120  | 80                                   | —                                                 | 10         | —       |                  |                  |                      | 5                |                   |                       | 5                 |                   |
| 121  | 60                                   | —                                                 | 10         | 20      |                  |                  |                      |                  |                   |                       | 10                |                   |
| 122  | 80                                   | —                                                 | 10         | 5       |                  |                  |                      |                  |                   |                       | 5                 |                   |
| 123  | 40                                   | —                                                 | 5          | 2       |                  |                  | 2                    | 1                |                   | 25                    | 25                |                   |
| 124  | 60                                   | —                                                 | 20         | 5       |                  |                  | 5                    | 3                | 3                 |                       | 4                 |                   |

TABLE 2-continued

| Nos. | (Ex. 1)(Group A)<br>Composition      |                                  |                       |                       |                      |                  |                  |                       |                   |                   |
|------|--------------------------------------|----------------------------------|-----------------------|-----------------------|----------------------|------------------|------------------|-----------------------|-------------------|-------------------|
|      | Molybdates<br>(wt. %)                |                                  | Glass<br>A<br>(wt. %) | Glass<br>B<br>(wt. %) | Fluorides<br>(wt. %) |                  |                  | Carbonates<br>(wt. %) |                   |                   |
|      | CaMoO <sub>4</sub>                   | Ca <sub>3</sub> MoO <sub>6</sub> |                       |                       | SrF <sub>2</sub>     | BaF <sub>2</sub> | MgF <sub>2</sub> | CaF <sub>2</sub>      | SrCO <sub>3</sub> | BaCO <sub>3</sub> |
| 125  | 40                                   | 40                               | 3.4                   | —                     |                      |                  |                  |                       | 8.3               | 8.3               |
| 126  | 30                                   | 30                               | —                     | 20                    | 2.5                  | 2.5              | 2.5              | 2.5                   | 2.5               | 2.5               |
|      | <u>SrMoO<sub>4</sub></u>             |                                  |                       |                       |                      |                  |                  |                       |                   |                   |
| 127  | 25                                   | —                                | 58.4                  | —                     |                      |                  |                  |                       | 8.3               | 8.3               |
| 128  | 41.7                                 | —                                | 41.7                  | —                     |                      |                  |                  |                       | 8.3               | 8.3               |
| 129  | 62.5                                 | —                                | 20.9                  | —                     |                      |                  |                  |                       | 8.3               | 8.3               |
| 130  | 80                                   | —                                | 3.4                   | —                     |                      |                  |                  |                       | 8.3               | 8.3               |
| 131  | 41.7                                 | —                                | 41.7                  | —                     |                      |                  |                  |                       | 8.3               | 8.3               |
| 132  | 62.5                                 | —                                | 20.9                  | —                     |                      |                  |                  |                       | 8.3               | 8.3               |
| 133  | 40                                   | —                                | 59                    | —                     |                      |                  |                  | 0.5                   | 0.5               |                   |
| 134  | 40                                   | —                                | 5                     | —                     |                      |                  | 5                | 50                    |                   |                   |
| 135  | 60                                   | —                                | 5                     | —                     |                      |                  | 30               | 5                     |                   |                   |
| 136  | 60                                   | —                                | 20                    | —                     |                      |                  | 10               | 10                    |                   |                   |
| 137  | 80                                   | —                                | 10                    | —                     |                      |                  | 5                | 5                     |                   |                   |
| 138  | 80                                   | —                                | 7                     | —                     |                      |                  | 3                | 10                    |                   |                   |
| 139  | 95                                   | —                                | 4                     | —                     |                      |                  | 0.5              | 0.5                   |                   |                   |
| 140  | 40                                   | —                                | 59                    | —                     | 0.5                  |                  |                  |                       |                   | 0.5               |
| 141  | 40                                   | —                                | 5                     | —                     | 5                    |                  |                  |                       |                   | 50                |
| 142  | 60                                   | —                                | 5                     | —                     | 30                   |                  |                  |                       |                   | 5                 |
| 143  | 60                                   | —                                | 20                    | —                     | 10                   |                  |                  |                       |                   | 10                |
| 144  | 80                                   | —                                | 10                    | —                     | 5                    |                  |                  |                       |                   | 5                 |
| 145  | 80                                   | —                                | 7                     | —                     | 3                    |                  |                  |                       |                   | 10                |
| 146  | 95                                   | —                                | 4                     | —                     | 0.5                  |                  |                  |                       |                   | 0.5               |
| 147  | 60                                   | —                                | 20                    | —                     |                      |                  | 10               |                       |                   | 10                |
| 148  | 80                                   | —                                | 7                     | —                     |                      |                  | 3                |                       |                   | 10                |
| 149  | 60                                   | —                                | 20                    | —                     |                      |                  | 10               |                       |                   | 10                |
| 150  | 80                                   | —                                | 7                     | —                     |                      |                  | 3                |                       |                   | 10                |
| 151  | 60                                   | —                                | 20                    | —                     |                      |                  | 10               |                       |                   | 10                |
| 152  | 80                                   | —                                | 7                     | —                     |                      |                  | 3                |                       |                   | 10                |
| 153  | 60                                   | —                                | 10                    | —                     | 20                   |                  |                  |                       | 10                |                   |
| 154  | 80                                   | —                                | 10                    | —                     | 5                    |                  |                  |                       | 5                 |                   |
| 155  | 60                                   | —                                | 10                    | —                     | 20                   |                  |                  |                       | 10                |                   |
| 156  | 80                                   | —                                | 10                    | 5                     |                      |                  |                  |                       | 5                 |                   |
| 157  | 60                                   | —                                | 10                    | —                     | 20                   |                  |                  |                       | 10                |                   |
| 158  | 80                                   | —                                | 10                    | —                     | 5                    |                  |                  |                       | 5                 |                   |
| 159  | 40                                   | —                                | 5                     | —                     | 2                    |                  | 1                |                       | 25                |                   |
| 160  | 60                                   | —                                | 20                    | 5                     | 5                    |                  |                  | 3                     | 3                 | 25                |
|      | <u>Sr<sub>3</sub>MoO<sub>6</sub></u> |                                  |                       |                       |                      |                  |                  |                       |                   |                   |
| 161  | 25                                   | —                                | 58.4                  | —                     |                      |                  |                  | 8.3                   | 8.3               |                   |
| 162  | 41.7                                 | —                                | 41.7                  | —                     |                      |                  |                  | 8.3                   | 8.3               |                   |
| 163  | 62.5                                 | —                                | 20.9                  | —                     |                      |                  |                  | 8.3                   | 8.3               |                   |
| 164  | 80                                   | —                                | 3.4                   | —                     |                      |                  |                  | 8.3                   | 8.3               |                   |
| 165  | 41.7                                 | 41.7                             | —                     | —                     |                      |                  |                  | 8.3                   | 8.3               |                   |
| 166  | 62.5                                 | 20.9                             | —                     | —                     |                      |                  |                  | 8.3                   | 8.3               |                   |
| 167  | 40                                   | —                                | 59                    | 0.5                   |                      |                  |                  |                       |                   | 0.5               |
| 168  | 40                                   | —                                | 5                     | 5                     |                      |                  |                  |                       |                   | 50                |
| 169  | 60                                   | —                                | 5                     | 30                    |                      |                  |                  |                       |                   | 5                 |
| 170  | 60                                   | —                                | 20                    | 10                    |                      |                  |                  |                       |                   | 10                |
| 171  | 80                                   | —                                | 10                    | 5                     |                      |                  |                  |                       |                   | 5                 |
| 172  | 80                                   | —                                | 7                     | 3                     |                      |                  |                  |                       |                   | 10                |
| 173  | 95                                   | —                                | 4                     | 0.5                   |                      |                  |                  |                       |                   | 0.5               |
| 174  | 60                                   | —                                | 20                    | 10                    |                      |                  |                  |                       |                   | 10                |
| 175  | 80                                   | —                                | 7                     | 3                     |                      |                  |                  |                       |                   | 10                |
| 176  | 60                                   | —                                | 20                    | 10                    |                      |                  |                  |                       |                   | 10                |
| 177  | 80                                   | —                                | 7                     | 3                     |                      |                  |                  |                       |                   | 10                |
| 178  | 60                                   | —                                | 20                    | 10                    |                      |                  | 10               |                       |                   |                   |
| 179  | 80                                   | —                                | 7                     | 3                     |                      |                  | 10               |                       |                   |                   |
| 180  | 60                                   | —                                | 10                    | —                     | 20                   |                  |                  |                       | 10                |                   |
| 181  | 80                                   | —                                | 10                    | —                     | 5                    |                  |                  |                       | 5                 |                   |
| 182  | 60                                   | —                                | 10                    | —                     |                      | 20               |                  |                       | 10                |                   |
| 183  | 80                                   | —                                | 10                    | —                     | 5                    |                  |                  |                       | 5                 |                   |
| 184  | 60                                   | —                                | 10                    | —                     | 20                   |                  |                  |                       | 10                |                   |
| 185  | 80                                   | —                                | 10                    | —                     | 5                    |                  |                  |                       | 5                 |                   |
| 186  | 40                                   | —                                | 5                     | —                     | 2                    |                  | 1                | 2                     | 25                |                   |
| 187  | 60                                   | —                                | 20                    | —                     | 5                    |                  | 5                | 3                     | 3                 | 4                 |
|      | <u>SrMoO<sub>4</sub></u>             |                                  |                       |                       |                      |                  |                  |                       |                   |                   |
| 188  | 40                                   | 40                               | 3.4                   | —                     |                      |                  |                  | 8.3                   | 8.3               |                   |
| 189  | 30                                   | 30                               | —                     | 20                    | 2.5                  | 2.5              | 2.5              | 2.5                   | 2.5               | 2.5               |
|      | <u>BaMoO<sub>4</sub></u>             |                                  |                       |                       |                      |                  |                  |                       |                   |                   |
| 190  | 25                                   | —                                | 58.4                  | —                     |                      |                  |                  | 8.3                   | 8.3               |                   |
| 191  | 41.7                                 | —                                | 41.7                  | —                     |                      |                  |                  | 8.3                   | 8.3               |                   |
| 192  | 62.5                                 | —                                | 20.9                  | —                     |                      |                  |                  | 8.3                   | 8.3               |                   |
| 193  | 80                                   | —                                | 3.4                   | —                     |                      |                  |                  | 8.3                   | 8.3               |                   |
| 194  | 41.7                                 | —                                | 41.7                  | 41.7                  |                      |                  |                  | 8.3                   | 8.3               |                   |

TABLE 2-continued

| Nos.                                 | Molybdates<br>(wt. %)                                                                      | (Ex. I)(Group A)<br>Composition      |                       |                                      |                  |                  |                  |                       |                   |                   |                   |
|--------------------------------------|--------------------------------------------------------------------------------------------|--------------------------------------|-----------------------|--------------------------------------|------------------|------------------|------------------|-----------------------|-------------------|-------------------|-------------------|
|                                      |                                                                                            | Glass<br>A<br>(wt. %)                | Glass<br>B<br>(wt. %) | Fluorides<br>(wt. %)                 |                  |                  |                  | Carbonates<br>(wt. %) |                   |                   |                   |
|                                      |                                                                                            |                                      |                       | SrF <sub>2</sub>                     | BaF <sub>2</sub> | MgF <sub>2</sub> | CaF <sub>2</sub> | SrCO <sub>3</sub>     | BaCO <sub>3</sub> | MgCO <sub>3</sub> | CaCO <sub>3</sub> |
| 195                                  | 62.5                                                                                       | —                                    | 20.9                  |                                      |                  |                  | 8.3              | 8.3                   |                   |                   | 0.5               |
| 196                                  | 40                                                                                         | —                                    | 59                    |                                      | 0.5              |                  |                  |                       |                   |                   | 50                |
| 197                                  | 40                                                                                         | —                                    | 5                     |                                      | 5                |                  |                  |                       |                   |                   | 5                 |
| 198                                  | 60                                                                                         | —                                    | 5                     |                                      | 30               |                  |                  |                       |                   |                   | 10                |
| 199                                  | 60                                                                                         | —                                    | 20                    |                                      | 10               |                  |                  |                       |                   |                   | 10                |
| 200                                  | 80                                                                                         | —                                    | 7                     |                                      | 3                |                  |                  |                       |                   |                   | 10                |
| 201                                  | 95                                                                                         | —                                    | 4                     |                                      | 0.5              |                  |                  |                       |                   |                   | 0.5               |
| 202                                  | 60                                                                                         | —                                    | 20                    |                                      | 10               |                  |                  |                       |                   |                   | 10                |
| 203                                  | 60                                                                                         | —                                    | 20                    |                                      | 10               |                  |                  | 10                    |                   |                   | 10                |
| 204                                  | 60                                                                                         | —                                    | 20                    |                                      | 10               |                  |                  | 10                    |                   |                   | 10                |
| 205                                  | 80                                                                                         | —                                    | 7                     |                                      |                  | 3                |                  |                       |                   |                   | 10                |
| 206                                  | 80                                                                                         | —                                    | 10                    |                                      |                  |                  | 3                |                       |                   |                   | 10                |
| 207                                  | 80                                                                                         | —                                    | 7                     | 3                                    |                  |                  |                  |                       |                   |                   | 10                |
| 208                                  | 40                                                                                         | —                                    | 5                     |                                      | 5                |                  |                  |                       |                   |                   | 0.5               |
| 209                                  | 40                                                                                         | —                                    | 5                     |                                      |                  |                  | 5                |                       |                   |                   | 10                |
| 210                                  | 40                                                                                         | —                                    | 5                     |                                      | 2.5              |                  | 2.5              |                       |                   |                   | 10                |
| <u>Ba<sub>2</sub>MoO<sub>5</sub></u> |                                                                                            |                                      |                       |                                      |                  |                  |                  |                       |                   |                   |                   |
| 211                                  | 25                                                                                         | —                                    | 58.4                  |                                      |                  |                  | 8.3              | 8.3                   |                   |                   |                   |
| 212                                  | 41.7                                                                                       | —                                    | 41.7                  |                                      |                  |                  | 8.3              | 8.3                   |                   |                   |                   |
| 213                                  | 62.5                                                                                       | —                                    | 20.9                  |                                      |                  |                  | 8.3              | 8.3                   |                   |                   |                   |
| 214                                  | 80                                                                                         | —                                    | 3.4                   |                                      |                  |                  | 8.3              | 8.3                   |                   |                   |                   |
| 215                                  | 40                                                                                         | —                                    | 59                    | 0.5                                  |                  |                  |                  |                       |                   |                   | 0.5               |
| 216                                  | 40                                                                                         | —                                    | 5                     | 5                                    |                  |                  |                  |                       |                   |                   | 50                |
| 217                                  | 60                                                                                         | —                                    | 20                    | 10                                   |                  |                  |                  |                       |                   |                   | 10                |
| 218                                  | 60                                                                                         | —                                    | 5                     | 30                                   |                  |                  |                  |                       |                   |                   | 5                 |
| 219                                  | 80                                                                                         | —                                    | 7                     | 3                                    |                  |                  |                  |                       |                   |                   | 10                |
| 220                                  | 95                                                                                         | —                                    | 4                     | 0.5                                  |                  |                  |                  |                       |                   |                   | 0.5               |
| 221                                  | 60                                                                                         | —                                    | 20                    | 10                                   |                  |                  |                  | 3                     | 3                 |                   | 4                 |
| 222                                  | 60                                                                                         | —                                    | 20                    | 10                                   |                  |                  |                  |                       |                   |                   | 10                |
| 223                                  | 60                                                                                         | —                                    | 20                    | 10                                   |                  |                  |                  |                       |                   |                   | 10                |
| 224                                  | 80                                                                                         | —                                    | 7                     |                                      | 3                |                  |                  |                       |                   |                   | 10                |
| 225                                  | 80                                                                                         | —                                    | 7                     |                                      |                  | 3                |                  |                       |                   |                   | 10                |
| 226                                  | 80                                                                                         | —                                    | 7                     | 3                                    |                  |                  |                  |                       |                   |                   | 10                |
| 227                                  | 60                                                                                         | —                                    | 5                     | 20                                   |                  |                  | 10               |                       |                   |                   | 5                 |
| 228                                  | 60                                                                                         | —                                    | 5                     | 20                                   |                  |                  | 10               | 2.5                   |                   |                   | 2.5               |
| 229                                  | 60                                                                                         | —                                    | 5                     | 10                                   | 10               | 10               |                  |                       | 3                 |                   | 2                 |
| <u>Ba<sub>3</sub>MoO<sub>6</sub></u> |                                                                                            |                                      |                       |                                      |                  |                  |                  |                       |                   |                   |                   |
| 230                                  | 41.7                                                                                       | 41.7                                 |                       |                                      |                  |                  | 8.3              | 8.3                   |                   |                   |                   |
| 231                                  | 62.5                                                                                       | 20.9                                 |                       |                                      |                  |                  | 8.3              | 8.3                   |                   |                   |                   |
| 232                                  | 41.7                                                                                       | —                                    | 41.7                  |                                      |                  |                  | 8.3              | 8.3                   |                   |                   |                   |
| 233                                  | 62.5                                                                                       | —                                    | 20.9                  |                                      |                  |                  | 8.3              | 8.3                   |                   |                   |                   |
| 234                                  | 40                                                                                         | —                                    | 59                    |                                      | 0.5              |                  |                  |                       |                   |                   | 0.5               |
| 235                                  | 40                                                                                         | —                                    | 5                     |                                      | 5                |                  |                  |                       |                   |                   | 50                |
| 236                                  | 60                                                                                         | —                                    | 20                    |                                      |                  | 10               |                  |                       |                   |                   | 10                |
| 237                                  | 60                                                                                         | —                                    | 5                     |                                      | 30               |                  |                  |                       |                   |                   | 5                 |
| 238                                  | 80                                                                                         | —                                    | 7                     |                                      | 3                |                  |                  |                       |                   |                   | 10                |
| 239                                  | 95                                                                                         | —                                    | 4                     |                                      | 0.5              |                  |                  | 0.5                   |                   |                   |                   |
| 240                                  | 60                                                                                         | —                                    | 20                    |                                      | 10               |                  |                  |                       |                   |                   | 10                |
| 241                                  | 60                                                                                         | —                                    | 20                    |                                      | 10               |                  |                  |                       |                   |                   | 10                |
| 242                                  | 60                                                                                         | —                                    | 20                    |                                      | 10               |                  |                  |                       |                   |                   | 10                |
| 243                                  | 80                                                                                         | —                                    | 7                     |                                      |                  | 3                |                  | 3                     |                   |                   | 10                |
| 244                                  | 80                                                                                         | —                                    | 7                     | 3                                    |                  |                  |                  |                       |                   |                   | 10                |
| 245                                  | 80                                                                                         | —                                    | 7                     |                                      | 3                |                  |                  |                       |                   |                   | 10                |
| <u>BaMoO<sub>4</sub></u>             |                                                                                            | <u>Ba<sub>3</sub>MoO<sub>6</sub></u> |                       |                                      |                  |                  |                  |                       |                   |                   |                   |
| 246                                  | 40                                                                                         | 40                                   |                       |                                      |                  |                  | 5                |                       |                   |                   | 5                 |
| <u>BaMoO<sub>4</sub></u>             |                                                                                            | <u>Ba<sub>2</sub>MoO<sub>5</sub></u> |                       | <u>Ba<sub>3</sub>MoO<sub>6</sub></u> |                  |                  |                  |                       |                   |                   |                   |
| 247                                  | 30                                                                                         | 20                                   | 20                    | 20                                   | 7                |                  | 1.5              | 1.5                   | 5                 |                   |                   |
| 248                                  | 20.8                                                                                       | 20.8                                 | 20.8                  | 20.8                                 | 7                | 1                | 0.5              | 0.5                   | 1                 | 3                 | 2                 |
| 249                                  | (Mg <sub>0.3</sub> Ca <sub>0.7</sub> )MoO <sub>4</sub>                                     | 41.7                                 | 41.7                  | —                                    |                  | 8.3              |                  |                       |                   |                   | 8.3               |
| 250                                  | (Mg <sub>0.7</sub> Ca <sub>0.3</sub> )MoO <sub>4</sub>                                     | 41.7                                 | 41.7                  | —                                    |                  | 8.3              |                  |                       |                   |                   | 8.3               |
| 251                                  | (Ca <sub>0.3</sub> Sr <sub>0.7</sub> )MoO <sub>4</sub>                                     | 41.7                                 | 41.7                  | —                                    |                  | 8.3              |                  |                       |                   |                   | 8.3               |
| 252                                  | (Ca <sub>0.7</sub> Sr <sub>0.3</sub> )MoO <sub>4</sub>                                     | 41.7                                 | 41.7                  | —                                    |                  | 8.3              |                  |                       |                   |                   | 8.3               |
| 253                                  | (Mg <sub>0.3</sub> Ba <sub>0.7</sub> )MoO <sub>4</sub>                                     | 41.7                                 | 41.7                  | —                                    |                  | 8.3              |                  |                       |                   |                   | 8.3               |
| 254                                  | (Mg <sub>0.7</sub> Ba <sub>0.3</sub> )MoO <sub>4</sub>                                     | 41.7                                 | 41.7                  | —                                    |                  | 8.3              |                  |                       |                   |                   | 8.3               |
| 255                                  | (Mg <sub>0.2</sub> Ca <sub>0.2</sub> Ba <sub>0.6</sub> )MoO <sub>4</sub>                   | 41.7                                 | 41.7                  | —                                    |                  | 8.3              |                  |                       |                   |                   | 8.3               |
| 256                                  | (Mg <sub>0.3</sub> Ca <sub>0.4</sub> Ba <sub>0.3</sub> )MoO <sub>4</sub>                   | 41.7                                 | 41.7                  | —                                    |                  | 8.3              |                  |                       |                   |                   | 8.3               |
| 257                                  | (Ca <sub>0.2</sub> Sr <sub>0.6</sub> Ba <sub>0.2</sub> )MoO <sub>4</sub>                   | 41.7                                 | 41.7                  | —                                    |                  | 8.3              |                  |                       |                   |                   | 8.3               |
| 258                                  | (Ca <sub>0.4</sub> Sr <sub>0.3</sub> Ba <sub>0.3</sub> )MoO <sub>4</sub>                   | 41.7                                 | 41.7                  | —                                    |                  | 8.3              |                  |                       |                   |                   | 8.3               |
| 259                                  | (Mg <sub>0.2</sub> Ca <sub>0.2</sub> Sr <sub>0.2</sub> Ba <sub>0.4</sub> )MoO <sub>4</sub> | 41.7                                 | 41.7                  | —                                    |                  | 8.3              |                  |                       |                   |                   | 8.3               |
| 260                                  | (Mg <sub>0.2</sub> Ca <sub>0.3</sub> Sr <sub>0.3</sub> Ba <sub>0.2</sub> )MoO <sub>4</sub> | 41.7                                 | 41.7                  | —                                    |                  | 8.3              |                  |                       |                   |                   | 8.3               |
| 261                                  | (Ca <sub>2.0</sub> Sr <sub>1.0</sub> )MoO <sub>6</sub>                                     | 41.7                                 | 41.7                  | —                                    |                  | 8.3              |                  |                       |                   |                   | 8.3               |
| 262                                  | (Ca <sub>1.0</sub> Sr <sub>2.0</sub> )MoO <sub>6</sub>                                     | 41.7                                 | 41.7                  | —                                    |                  | 8.3              |                  |                       |                   |                   | 8.3               |
| 263                                  | (Sr <sub>2.0</sub> Ba <sub>1.0</sub> )MoO <sub>6</sub>                                     | 41.7                                 | 41.7                  | —                                    |                  | 8.3              |                  |                       |                   |                   | 8.3               |
| 264                                  | (Sr <sub>1.0</sub> Ba <sub>2.0</sub> )MoO <sub>6</sub>                                     | 41.7                                 | 41.7                  | —                                    |                  | 8.3              |                  |                       |                   |                   | 8.3               |
| 265                                  | MgMoO <sub>4</sub>                                                                         | 29.2                                 | —                     | 20.8                                 |                  |                  |                  | 8.3                   | 8.3               |                   |                   |

TABLE 2-continued

| Nos. | Molybdates<br>(wt. %)                           | (Ex. 1)(Group A)<br>Composition |                  |                       |                  |                      |  | Carbonates<br>(wt. %) |                   |                   |
|------|-------------------------------------------------|---------------------------------|------------------|-----------------------|------------------|----------------------|--|-----------------------|-------------------|-------------------|
|      |                                                 | Glass<br>A<br>(wt. %)           |                  | Glass<br>B<br>(wt. %) |                  | Fluorides<br>(wt. %) |  | SrCO <sub>3</sub>     | BaCO <sub>3</sub> | MgCO <sub>3</sub> |
|      |                                                 | SrF <sub>2</sub>                | BaF <sub>2</sub> | MgF <sub>2</sub>      | CaF <sub>2</sub> |                      |  |                       |                   |                   |
| 266  | Ca <sub>3</sub> MoO <sub>6</sub>                | 33.4                            |                  |                       |                  |                      |  |                       |                   |                   |
| 266  | CaMoO <sub>4</sub>                              | 29.2                            | —                | 20.8                  |                  |                      |  | 8.3                   | 8.3               |                   |
|      | Sr <sub>3</sub> MoO <sub>6</sub>                | 33.4                            |                  |                       |                  |                      |  |                       |                   |                   |
| 267  | SrMoO <sub>4</sub>                              | 29.2                            | —                | 20.8                  |                  |                      |  | 8.3                   | 8.3               |                   |
|      | Ba <sub>2</sub> MoO <sub>5</sub>                | 33.4                            |                  |                       |                  |                      |  |                       |                   |                   |
| 268  | BaMoO <sub>4</sub>                              | 29.2                            | —                | 20.8                  |                  |                      |  | 8.3                   | 8.3               |                   |
|      | Mg <sub>2</sub> Mo <sub>3</sub> O <sub>11</sub> | 33.4                            |                  |                       |                  |                      |  |                       |                   |                   |
| 269  | MgMoO <sub>4</sub>                              | 20.8                            | —                | 20.8                  |                  |                      |  | 8.3                   | 8.3               |                   |
|      | Sr <sub>3</sub> MoO <sub>6</sub>                | 20.8                            |                  |                       |                  |                      |  |                       |                   |                   |
|      | Ba <sub>3</sub> MoO <sub>6</sub>                | 20.8                            |                  |                       |                  |                      |  |                       |                   |                   |
| 270  | Mg <sub>2</sub> Mo <sub>3</sub> O <sub>11</sub> | 12.5                            | —                | 20.8                  |                  |                      |  | 8.3                   | 8.3               |                   |
|      | CaMoO <sub>4</sub>                              | 16.7                            |                  |                       |                  |                      |  |                       |                   |                   |
|      | SrMoO <sub>4</sub>                              | 16.7                            |                  |                       |                  |                      |  |                       |                   |                   |
|      | BaMoO <sub>4</sub>                              | 16.7                            |                  |                       |                  |                      |  |                       |                   |                   |
| 271  | MgMoO <sub>4</sub>                              | 30                              | —                | 20                    |                  |                      |  | 10                    | 10                |                   |
|      | Ca <sub>3</sub> MoO <sub>6</sub>                | 30                              |                  |                       |                  |                      |  |                       |                   |                   |
| 272  | CaMoO <sub>4</sub>                              | 30                              | —                | 20                    |                  |                      |  | 10                    | 10                |                   |
|      | Sr <sub>3</sub> MoO <sub>6</sub>                | 30                              |                  |                       |                  |                      |  |                       |                   |                   |
| 273  | SrMoO <sub>4</sub>                              | 30                              | —                | 20                    |                  |                      |  | 10                    | 10                |                   |
|      | Ba <sub>2</sub> MoO <sub>5</sub>                | 30                              |                  |                       |                  |                      |  |                       |                   |                   |
| 274  | BaMoO <sub>4</sub>                              | 30                              | —                | 20                    |                  |                      |  | 10                    | 10                |                   |
|      | Mg <sub>2</sub> Mo <sub>3</sub> O <sub>11</sub> | 30                              |                  |                       |                  |                      |  |                       |                   |                   |
| 275  | MgMoO <sub>4</sub>                              | 20                              | —                | 20                    |                  |                      |  | 10                    | 10                |                   |
|      | Sr <sub>3</sub> MoO <sub>6</sub>                | 20                              |                  |                       |                  |                      |  |                       |                   |                   |
|      | Ba <sub>3</sub> MoO <sub>6</sub>                | 20                              |                  |                       |                  |                      |  |                       |                   |                   |
| 276  | Mg <sub>2</sub> Mo <sub>3</sub> O <sub>11</sub> | 15                              | —                | 20                    |                  |                      |  | 10                    | 10                |                   |
|      | CaMoO <sub>4</sub>                              | 15                              |                  |                       |                  |                      |  |                       |                   |                   |
|      | SrMoO <sub>4</sub>                              | 15                              |                  |                       |                  |                      |  |                       |                   |                   |
|      | BaMoO <sub>4</sub>                              | 15                              |                  |                       |                  |                      |  |                       |                   |                   |

TABLE 3

(Ex. 1 - Group B)

| Nos                                  | Molybdate<br>(wt. %) | Glass<br>A<br>(wt. %) | Glass<br>B<br>(wt. %) | Fluorides<br>(wt. %) |                  |                  | Carbonate<br>(wt. %) |                   |                   |                   |
|--------------------------------------|----------------------|-----------------------|-----------------------|----------------------|------------------|------------------|----------------------|-------------------|-------------------|-------------------|
|                                      |                      |                       |                       | SrF <sub>2</sub>     | BaF <sub>2</sub> | MgF <sub>2</sub> | SrCO <sub>3</sub>    | BaCO <sub>3</sub> | MgCO <sub>3</sub> | CaCO <sub>3</sub> |
| <u>ZnMoO<sub>4</sub></u>             |                      |                       |                       |                      |                  |                  |                      |                   |                   |                   |
| 1                                    | 45.9                 | 37.5                  | —                     |                      |                  | 8.3              | 8.3                  |                   |                   |                   |
| 2                                    | 54.2                 | 29.2                  | —                     |                      |                  | 8.3              | 8.3                  |                   |                   |                   |
| 3                                    | 66.7                 | 16.7                  | —                     |                      |                  | 8.3              | 8.3                  |                   |                   |                   |
| 4                                    | 80                   | 3.4                   | —                     |                      |                  | 8.3              | 8.3                  |                   |                   |                   |
| 5                                    | 54.2                 | —                     | 29.2                  |                      |                  | 8.3              | 8.3                  |                   |                   |                   |
| 6                                    | 66.7                 | —                     | 16.7                  |                      |                  | 8.3              | 8.3                  |                   |                   |                   |
| 7                                    | 65                   | —                     | 34                    |                      | 0.5              |                  |                      |                   | 0.5               |                   |
| 8                                    | 65                   | —                     | 4                     |                      | 1                |                  |                      |                   | 30                |                   |
| 9                                    | 75                   | —                     | 4                     |                      | 20               |                  |                      |                   | 1                 |                   |
| 10                                   | 75                   | —                     | 10                    |                      | 3                |                  |                      |                   | 12                |                   |
| 11                                   | 85                   | —                     | 5                     |                      | 5                |                  |                      |                   | 5                 |                   |
| 12                                   | 95                   | —                     | 4                     |                      | 0.5              |                  |                      |                   | 0.5               |                   |
| 13                                   | 65                   | —                     | 4                     |                      | 1                |                  |                      |                   | 30                |                   |
| 14                                   | 75                   | —                     | 10                    |                      | 3                |                  |                      |                   | 12                |                   |
| 15                                   | 65                   | —                     | 4                     |                      | 1                |                  | 30                   |                   |                   |                   |
| 16                                   | 75                   | —                     | 10                    |                      | 3                |                  | 12                   |                   |                   |                   |
| 17                                   | 65                   | —                     | 4                     |                      | 1                |                  | 30                   |                   |                   |                   |
| 18                                   | 75                   | —                     | 10                    |                      | 3                |                  | 12                   |                   |                   |                   |
| 19                                   | 75                   | —                     | 4                     |                      |                  | 20               |                      |                   | 1                 |                   |
| 20                                   | 85                   | —                     | 5                     |                      |                  | 5                |                      |                   | 5                 |                   |
| 21                                   | 75                   | —                     | 4                     | 20                   |                  |                  |                      |                   | 1                 |                   |
| 22                                   | 85                   | —                     | 5                     | 5                    |                  |                  |                      |                   | 5                 |                   |
| 23                                   | 75                   | —                     | 4                     |                      | 20               |                  |                      |                   | 1                 |                   |
| 24                                   | 85                   | —                     | 5                     |                      | 5                |                  |                      |                   | 5                 |                   |
| 25                                   | 75                   | —                     | 10                    |                      |                  | 3                |                      | 6                 | 6                 |                   |
| 26                                   | 75                   | —                     | 10                    | 1.5                  |                  |                  | 1.5                  | 6                 | 6                 | 6                 |
| 27                                   | 75                   | —                     | 10                    | 1                    | 1                |                  | 1                    | 4                 | 4                 | 4                 |
| <u>ZnMo<sub>2</sub>O<sub>7</sub></u> |                      |                       |                       |                      |                  |                  |                      |                   |                   |                   |
| 28                                   | 45.9                 | 37.5                  | —                     |                      |                  | 8.3              | 8.3                  |                   |                   |                   |
| 29                                   | 54.2                 | 29.2                  | —                     |                      |                  | 8.3              | 8.3                  |                   |                   |                   |
| 30                                   | 66.7                 | 16.7                  | —                     |                      |                  | 8.3              | 8.3                  |                   |                   |                   |
| 31                                   | 80                   | 3.4                   | —                     |                      |                  | 8.3              | 8.3                  |                   |                   |                   |
| 32                                   | 54.2                 | —                     | 29.2                  |                      |                  | 8.3              | 8.3                  |                   |                   |                   |
| 33                                   | 66.7                 | —                     | 16.7                  |                      |                  | 8.3              | 8.3                  |                   |                   |                   |
| 34                                   | 65                   | —                     | 34                    |                      |                  | 0.5              | 0.5                  |                   |                   |                   |

TABLE 3-continued

(Ex. 1 - Group B)

| NOS                                              | Molybdate<br>(wt. %)                           | Glass<br>A<br>(wt. %) | Glass<br>B<br>(wt. %) | Fluorides<br>(wt. %) |                  |                  |                  | Carbonate<br>(wt. %) |                   |                   |                   |
|--------------------------------------------------|------------------------------------------------|-----------------------|-----------------------|----------------------|------------------|------------------|------------------|----------------------|-------------------|-------------------|-------------------|
|                                                  |                                                |                       |                       | SrF <sub>2</sub>     | BaF <sub>2</sub> | MgF <sub>2</sub> | CaF <sub>2</sub> | SrCO <sub>3</sub>    | BaCO <sub>3</sub> | MgCO <sub>3</sub> | CaCO <sub>3</sub> |
| 35                                               | 65                                             | —                     | 4                     |                      |                  |                  | 1                | 30                   |                   |                   |                   |
| 36                                               | 75                                             | —                     | 4                     |                      |                  |                  | 20               | 1                    |                   |                   |                   |
| 37                                               | 75                                             | —                     | 10                    |                      |                  |                  | 3                | 12                   |                   |                   |                   |
| 38                                               | 85                                             | —                     | 5                     |                      |                  |                  | 5                | 5                    |                   |                   |                   |
| 39                                               | 95                                             | —                     | 4                     |                      |                  |                  | 0.5              | 0.5                  |                   |                   |                   |
| 40                                               | 65                                             | —                     | 4                     |                      |                  |                  | 1                |                      | 30                |                   |                   |
| 41                                               | 75                                             | —                     | 10                    |                      |                  |                  | 3                |                      |                   | 12                |                   |
| 42                                               | 65                                             | —                     | 4                     |                      |                  |                  | 1                |                      |                   | 30                |                   |
| 43                                               | 75                                             | —                     | 10                    |                      |                  |                  | 3                |                      |                   | 12                |                   |
| 44                                               | 65                                             | —                     | 4                     |                      |                  |                  | 1                |                      | 30                |                   |                   |
| 45                                               | 75                                             | —                     | 10                    |                      |                  |                  | 3                |                      | 12                |                   |                   |
| 46                                               | 75                                             | —                     | 4                     |                      |                  | 20               |                  | 1                    |                   |                   |                   |
| 47                                               | 85                                             | —                     | 5                     |                      |                  | 5                |                  | 5                    |                   |                   |                   |
| 48                                               | 75                                             | —                     | 4                     | 20                   |                  |                  |                  | 1                    |                   |                   |                   |
| 49                                               | 85                                             | —                     | 5                     | 5                    |                  |                  |                  | 5                    |                   |                   |                   |
| 50                                               | 75                                             | —                     | 4                     |                      | 20               |                  |                  | 1                    |                   |                   |                   |
| 51                                               | 85                                             | —                     | 5                     |                      | 5                |                  |                  | 5                    |                   |                   |                   |
| 52                                               | 65                                             | —                     | 4                     |                      |                  |                  | 1                |                      | 15                | 15                |                   |
| 53                                               | 65                                             | —                     | 4                     | 0.5                  |                  |                  | 0.5              |                      | 20                |                   | 10                |
| 54                                               | 65                                             | —                     | 4                     |                      | 0.5              |                  | 0.5              |                      | 15                |                   | 15                |
| <u>Zn<sub>3</sub>Mo<sub>2</sub>O<sub>9</sub></u> |                                                |                       |                       |                      |                  |                  |                  |                      |                   |                   |                   |
| 55                                               | 54.2                                           | 29.2                  | —                     |                      |                  |                  |                  | 8.3                  | 8.3               |                   |                   |
| 56                                               | 66.7                                           | 16.7                  | —                     |                      |                  |                  |                  | 8.3                  | 8.3               |                   |                   |
| 57                                               | 54.2                                           | —                     | 29.2                  |                      |                  |                  |                  | 8.3                  | 8.3               |                   |                   |
| 58                                               | 66.7                                           | —                     | 16.7                  |                      |                  |                  |                  | 8.3                  | 8.3               |                   |                   |
| 59                                               | 65                                             | —                     | 34                    | 0.5                  |                  |                  |                  |                      | 0.5               |                   |                   |
| 60                                               | 65                                             | —                     | 4                     | 1                    |                  |                  |                  |                      | 30                |                   |                   |
| 61                                               | 75                                             | —                     | 4                     | 20                   |                  |                  |                  |                      | 1                 |                   |                   |
| 62                                               | 75                                             | —                     | 10                    | 3                    |                  |                  |                  |                      | 12                |                   |                   |
| 63                                               | 85                                             | —                     | 5                     | 5                    |                  |                  |                  |                      | 5                 |                   |                   |
| 64                                               | 95                                             | —                     | 4                     | 0.5                  |                  |                  |                  |                      | 0.5               |                   |                   |
| 65                                               | 65                                             | —                     | 4                     | 1                    |                  |                  |                  |                      | 30                |                   |                   |
| 66                                               | 75                                             | —                     | 10                    | 3                    |                  |                  |                  |                      | 12                |                   |                   |
| 67                                               | 65                                             | —                     | 4                     | 1                    |                  |                  |                  |                      | 30                |                   |                   |
| 68                                               | 75                                             | —                     | 10                    | 3                    |                  |                  |                  |                      | 12                |                   |                   |
| 69                                               | 65                                             | —                     | 4                     | 1                    |                  |                  |                  | 30                   |                   |                   |                   |
| 70                                               | 75                                             | —                     | 10                    | 3                    |                  |                  |                  | 12                   |                   |                   |                   |
| 71                                               | 75                                             | —                     | 4                     |                      | 20               |                  |                  |                      | 1                 |                   |                   |
| 72                                               | 85                                             | —                     | 5                     |                      | 5                |                  |                  |                      | 5                 |                   |                   |
| 73                                               | 75                                             | —                     | 4                     |                      |                  | 20               |                  |                      | 1                 |                   |                   |
| 74                                               | 85                                             | —                     | 5                     |                      |                  | 5                |                  |                      | 5                 |                   |                   |
| 75                                               | 75                                             | —                     | 4                     |                      | 20               |                  |                  |                      | 1                 |                   |                   |
| 76                                               | 85                                             | —                     | 5                     |                      | 5                |                  |                  |                      | 5                 |                   |                   |
| 77                                               | 85                                             | —                     | 5                     | 5                    |                  |                  |                  | 2.5                  |                   | 2.5               |                   |
| 78                                               | 85                                             | —                     | 5                     |                      | 2.5              |                  |                  | 2.5                  |                   | 2.5               |                   |
| 79                                               | 85                                             | —                     | 5                     | 2.5                  | 2.5              |                  |                  | 1                    | 3                 | 2.5               | 1                 |
| 80                                               | ZnMoO <sub>4</sub>                             | 35                    | —                     | 10                   |                  |                  | 3                |                      |                   |                   | 12                |
|                                                  | ZnMo <sub>2</sub> O <sub>7</sub>               | 40                    |                       |                      |                  |                  |                  |                      |                   |                   |                   |
| 81                                               | ZnMoO <sub>4</sub>                             | 25                    | 16.7                  | —                    |                  |                  |                  | 8.3                  | 8.3               |                   |                   |
|                                                  | ZnMo <sub>2</sub> O <sub>7</sub>               | 25                    |                       |                      |                  |                  |                  |                      |                   |                   |                   |
|                                                  | Zn <sub>3</sub> Mo <sub>2</sub> O <sub>9</sub> | 16.7                  |                       |                      |                  |                  |                  |                      |                   |                   |                   |
| 82                                               | ZnMoO <sub>4</sub>                             | 20                    | —                     | 10                   | 1.5              |                  |                  | 1.5                  |                   | 6                 | 6                 |
|                                                  | ZnMo <sub>2</sub> O <sub>7</sub>               | 25                    |                       |                      |                  |                  |                  |                      |                   |                   |                   |
|                                                  | Zn <sub>3</sub> Mo <sub>2</sub> O <sub>9</sub> | 30                    |                       |                      |                  |                  |                  |                      |                   |                   |                   |
| 83                                               | ZnMoO <sub>4</sub>                             | 20                    | —                     | 10                   | 1                | 1                | 0.5              | 0.5                  | 3                 | 3                 | 3                 |
|                                                  | ZnMo <sub>2</sub> O <sub>7</sub>               | 25                    |                       |                      |                  |                  |                  |                      |                   |                   |                   |
|                                                  | Zn <sub>3</sub> Mo <sub>2</sub> O <sub>9</sub> | 30                    |                       |                      |                  |                  |                  |                      |                   |                   |                   |

TABLE 4

(Ex. 1 - Group C)

| NOS | Molybdate<br>Al <sub>2</sub> Mo <sub>3</sub> O <sub>12</sub><br>(wt. %) | Glass A<br>(wt. %) | Glass B<br>(wt. %) | Composition      |                  |                  |                  | Fluorides<br>(wt. %) |                   |                   |                   | Carbonate<br>(%) |  |  |  |
|-----|-------------------------------------------------------------------------|--------------------|--------------------|------------------|------------------|------------------|------------------|----------------------|-------------------|-------------------|-------------------|------------------|--|--|--|
|     |                                                                         |                    |                    | SrF <sub>2</sub> | BaF <sub>2</sub> | MgF <sub>2</sub> | CaF <sub>2</sub> | SrCO <sub>3</sub>    | BaCO <sub>3</sub> | MgCO <sub>3</sub> | CaCO <sub>3</sub> |                  |  |  |  |
| 1   | 41.7                                                                    | 41.7               | —                  |                  |                  |                  |                  | 8.3                  | 8.3               |                   |                   |                  |  |  |  |
| 2   | 54.2                                                                    | 29.2               | —                  |                  |                  |                  |                  | 8.3                  | 8.3               |                   |                   |                  |  |  |  |
| 3   | 66.7                                                                    | 16.7               | —                  |                  |                  |                  |                  | 8.3                  | 8.3               |                   |                   |                  |  |  |  |
| 4   | 80                                                                      | 3.4                | —                  |                  |                  |                  |                  | 8.3                  | 8.3               |                   |                   |                  |  |  |  |
| 5   | 41.7                                                                    | —                  | 41.7               |                  |                  |                  |                  | 8.3                  | 8.3               |                   |                   |                  |  |  |  |
| 6   | 54.2                                                                    | —                  | 29.3               |                  |                  |                  |                  | 8.3                  | 8.3               |                   |                   |                  |  |  |  |
| 7   | 66.7                                                                    | —                  | 16.7               |                  |                  |                  |                  | 8.3                  | 8.3               |                   |                   |                  |  |  |  |
| 8   | 80                                                                      | —                  | 3.4                |                  |                  |                  |                  | 8.3                  | 8.3               |                   |                   |                  |  |  |  |
| 9   | 66.8                                                                    | 8.3                | 8.3                |                  |                  |                  |                  | 8.3                  | 8.3               |                   |                   |                  |  |  |  |

TABLE 4-continued

| NOS | Molybdate<br>$\text{Al}_2\text{Mo}_3\text{O}_{12}$<br>(wt. %) | (Ex. 1 - Group C)<br>Composition |                    |                      |                |                |                          |                 |                 |
|-----|---------------------------------------------------------------|----------------------------------|--------------------|----------------------|----------------|----------------|--------------------------|-----------------|-----------------|
|     |                                                               | Glass A<br>(wt. %)               | Glass B<br>(wt. %) | Fluorides<br>(wt. %) |                |                | Carbonate<br>(<br>%<br>) |                 |                 |
|     |                                                               |                                  |                    | $\text{SrF}_2$       | $\text{BaF}_2$ | $\text{MgF}_2$ | $\text{CaF}_2$           | $\text{SrCO}_3$ | $\text{BaCO}_3$ |
| 10  | 60                                                            | —                                | 39                 | 0.5                  |                |                | 0.5                      |                 |                 |
| 11  | 60                                                            | —                                | 5                  |                      | 10             |                |                          | 25              |                 |
| 12  | 75                                                            | —                                | 10                 |                      | 5              |                |                          | 10              |                 |
| 13  | 85                                                            | —                                | 7                  |                      | 3              |                |                          | 5               |                 |
| 14  | 95                                                            | —                                | 4                  | 0.5                  |                |                | 0.5                      |                 |                 |
| 15  | 60                                                            | —                                | 39                 |                      |                | 0.5            |                          | 0.5             |                 |
| 16  | 60                                                            | —                                | 5                  |                      |                | 10             |                          | 25              |                 |
| 17  | 75                                                            | —                                | 10                 |                      |                | 5              |                          | 10              |                 |
| 18  | 85                                                            | —                                | 7                  |                      |                | 3              |                          | 5               |                 |
| 19  | 95                                                            | —                                | 4                  |                      |                | 0.5            |                          | 0.5             |                 |
| 20  | 75                                                            | —                                | 10                 |                      | 5              |                |                          | 10              |                 |
| 21  | 85                                                            | —                                | 7                  |                      | 3              |                |                          | 5               |                 |
| 22  | 75                                                            | —                                | 10                 |                      | 5              |                |                          |                 | 10              |
| 23  | 85                                                            | —                                | 7                  |                      | 3              |                |                          |                 | 5               |
| 24  | 75                                                            | —                                | 10                 |                      | 5              |                |                          | 10              |                 |
| 25  | 85                                                            | —                                | 7                  |                      | 3              |                |                          | 5               |                 |
| 26  | 75                                                            | —                                | 10                 |                      |                | 5              |                          | 10              |                 |
| 27  | 85                                                            | —                                | 7                  |                      |                | 3              |                          | 5               |                 |
| 28  | 75                                                            | —                                | 10                 |                      |                |                | 5                        | 10              |                 |
| 29  | 85                                                            | —                                | 7                  |                      |                |                | 3                        | 5               |                 |
| 30  | 75                                                            | —                                | 10                 | 5                    |                |                |                          | 10              |                 |
| 31  | 85                                                            | —                                | 7                  | 3                    |                |                |                          | 5               |                 |
| 32  | 75                                                            | —                                | 10                 |                      | 5              |                |                          | 5               |                 |
| 33  | 75                                                            | —                                | 10                 | 2.5                  |                |                | 2.5                      | 5               |                 |
| 34  | 75                                                            | —                                | 10                 | 2                    | 2              | 1              |                          | 3               |                 |
| 35  | 85                                                            | —                                | 7                  | 1                    | 1              |                | 1                        | 2               | 2               |
|     |                                                               |                                  |                    |                      |                |                |                          |                 | 1               |

TABLE 5

| NOS | Molybdate<br>$\text{ZrMo}_2\text{O}_8$<br>(wt. %) | (Ex. 1 - Group D)<br>Composition |                    |                      |                |                |                       |                 |                 |
|-----|---------------------------------------------------|----------------------------------|--------------------|----------------------|----------------|----------------|-----------------------|-----------------|-----------------|
|     |                                                   | Glass A<br>(wt. %)               | Glass B<br>(wt. %) | Fluorides<br>(wt. %) |                |                | Carbonates<br>(wt. %) |                 |                 |
|     |                                                   |                                  |                    | $\text{SrF}_2$       | $\text{BaF}_2$ | $\text{MgF}_2$ | $\text{CaF}_2$        | $\text{SrCO}_3$ | $\text{BaCO}_3$ |
| 1   | 29.2                                              | 54.2                             | —                  |                      |                |                | 8.3                   | 8.3             |                 |
| 2   | 45.9                                              | 37.5                             | —                  |                      |                |                | 8.3                   | 8.3             |                 |
| 3   | 62.5                                              | 20.9                             | —                  |                      |                |                | 8.3                   | 8.3             |                 |
| 4   | 80                                                | 3.4                              | —                  |                      |                |                | 8.3                   | 8.3             |                 |
| 5   | 45.9                                              | —                                | 37.5               |                      |                |                | 8.3                   | 8.3             |                 |
| 6   | 62.5                                              | —                                | 20.9               |                      |                |                | 8.3                   | 8.3             |                 |
| 7   | 45                                                | —                                | 54                 | 0.5                  |                |                |                       | 0.5             |                 |
| 8   | 45                                                | —                                | 4                  | 1                    |                |                |                       | 50              |                 |
| 9   | 60                                                | —                                | 20                 | 5                    |                |                |                       | 15              |                 |
| 10  | 60                                                | —                                | 10                 | 20                   |                |                |                       | 10              |                 |
| 11  | 80                                                | —                                | 10                 | 5                    |                |                |                       | 5               |                 |
| 12  | 80                                                | —                                | 7                  | 10                   |                |                |                       | 3               |                 |
| 13  | 95                                                | —                                | 4                  | 0.5                  |                |                |                       | 0.5             |                 |
| 14  | 45                                                | —                                | 54                 |                      | 0.5            |                |                       |                 | 0.5             |
| 15  | 45                                                | —                                | 4                  |                      | 1              |                |                       |                 | 50              |
| 16  | 60                                                | —                                | 20                 |                      | 5              |                |                       |                 | 15              |
| 17  | 60                                                | —                                | 10                 |                      | 20             |                |                       |                 | 10              |
| 18  | .80                                               | —                                | 10                 |                      |                | 5              |                       |                 | 5               |
| 19  | 80                                                | —                                | 7                  |                      |                | 10             |                       |                 | 3               |
| 20  | 95                                                | —                                | 4                  |                      | 0.5            |                |                       |                 | 0.5             |
| 21  | 60                                                | —                                | 20                 | 5                    |                |                |                       | 15              |                 |
| 22  | 80                                                | —                                | 10                 | 5                    |                |                |                       | 5               |                 |
| 23  | 60                                                | —                                | 20                 | 5                    |                |                |                       |                 | 15              |
| 24  | 80                                                | —                                | 10                 | 5                    |                |                |                       |                 | 5               |
| 25  | 60                                                | —                                | 20                 | 5                    |                |                | 15                    |                 |                 |
| 26  | 80                                                | —                                | 10                 | 5                    |                |                | 5                     |                 |                 |
| 27  | 60                                                | —                                | 10                 |                      |                | 20             |                       |                 | 10              |
| 28  | 80                                                | —                                | 7                  |                      |                | 10             |                       |                 | 3               |
| 29  | 60                                                | —                                | 10                 |                      |                | 20             |                       |                 | 10              |
| 30  | 80                                                | —                                | 7                  |                      |                | 10             |                       |                 | 3               |
| 31  | 60                                                | —                                | 10                 |                      | 20             |                |                       |                 | 10              |
| 32  | 80                                                | —                                | 7                  | 10                   |                |                |                       |                 | 3               |
| 33  | 45                                                | —                                | 4                  | 1                    |                |                | 30                    |                 | 20              |
| 34  | 45                                                | —                                | 4                  |                      | 0.5            |                | 0.5                   | 20              |                 |
|     | <u><math>\text{HfMo}_2\text{O}_8</math></u>       |                                  |                    |                      |                |                |                       |                 |                 |
| 35  | 29.2                                              | —                                | 54.2               |                      |                |                | 8.3                   | 8.3             |                 |
| 36  | 45.9                                              | —                                | 37.5               |                      |                |                | 8.3                   | 8.3             |                 |
| 37  | 62.5                                              | —                                | 20.9               |                      |                |                | 8.3                   | 8.3             |                 |

TABLE 5-continued

(Ex. 1 - Group D)

Composition

| NOs | Molybdate<br>(wt. %)                                                       | Glass A<br>(wt. %) | Glass B<br>(wt. %) | Fluorides<br>(wt. %) |                  |                  |                  | Carbonates<br>(wt. %) |                   |                   |                   |
|-----|----------------------------------------------------------------------------|--------------------|--------------------|----------------------|------------------|------------------|------------------|-----------------------|-------------------|-------------------|-------------------|
|     |                                                                            |                    |                    | SrF <sub>2</sub>     | BaF <sub>2</sub> | MgF <sub>2</sub> | CaF <sub>2</sub> | SrCO <sub>3</sub>     | BaCO <sub>3</sub> | MgCO <sub>3</sub> | CaCO <sub>3</sub> |
| 38  | 80                                                                         | —                  | 3.4                |                      |                  |                  | 8.3              | 8.3                   |                   |                   |                   |
| 39  | 45.9                                                                       | 37.5               | —                  |                      |                  |                  | 8.3              | 8.3                   |                   |                   |                   |
| 40  | 62.5                                                                       | 20.9               | —                  |                      |                  |                  | 8.3              | 8.3                   |                   |                   |                   |
| 41  | 45                                                                         | —                  | 54                 |                      |                  |                  | 0.5              | 0.5                   |                   |                   |                   |
| 42  | 45                                                                         | —                  | 4                  |                      |                  |                  | 1                | 50                    |                   |                   |                   |
| 43  | 60                                                                         | —                  | 20                 |                      |                  |                  | 5                | 15                    |                   |                   |                   |
| 44  | 60                                                                         | —                  | 10                 |                      |                  |                  | 20               | 10                    |                   |                   |                   |
| 45  | 80                                                                         | —                  | 10                 |                      |                  |                  | 5                | 5                     |                   |                   |                   |
| 46  | 80                                                                         | —                  | 7                  |                      |                  |                  | 10               | 3                     |                   |                   |                   |
| 47  | 95                                                                         | —                  | 4                  |                      |                  |                  | 0.5              | 0.5                   |                   |                   |                   |
| 48  | 60                                                                         | —                  | 20                 |                      |                  |                  | 5                |                       | 15                |                   |                   |
| 49  | 80                                                                         | —                  | 10                 |                      |                  |                  | 5                |                       | 5                 |                   |                   |
| 50  | 60                                                                         | —                  | 20                 |                      |                  |                  | 5                |                       |                   | 15                |                   |
| 51  | 80                                                                         | —                  | 10                 |                      |                  |                  | 5                |                       |                   | 5                 |                   |
| 52  | 60                                                                         | —                  | 20                 |                      |                  |                  | 5                |                       | 15                |                   |                   |
| 53  | 80                                                                         | —                  | 10                 |                      |                  |                  | 5                |                       | 5                 |                   |                   |
| 54  | 60                                                                         | —                  | 10                 |                      |                  |                  | 20               | 10                    |                   |                   |                   |
| 55  | 80                                                                         | —                  | 7                  |                      |                  |                  | 10               | 3                     |                   |                   |                   |
| 56  | 60                                                                         | —                  | 10                 |                      |                  |                  | 20               |                       | 10                |                   |                   |
| 57  | 80                                                                         | —                  | 7                  |                      |                  |                  | 10               |                       | 3                 |                   |                   |
| 58  | 60                                                                         | —                  | 10                 |                      |                  |                  | 20               |                       | 10                |                   |                   |
| 59  | 80                                                                         | —                  | 7                  |                      |                  |                  | 10               |                       | 3                 |                   |                   |
| 60  | 45                                                                         | —                  | 4                  |                      |                  |                  | 1                |                       | 30                |                   | 20                |
| 61  | 45                                                                         | —                  | 4                  | 0.5                  | 0.5              |                  | 1                |                       | 20                | 10                | 20                |
| 62  | (Zr <sub>0.5</sub> Mo <sub>0.5</sub> )Mo <sub>2</sub> O <sub>8</sub><br>80 | —                  | 10                 | 1                    | 2                | 1                | 1                | 1                     | 1                 | 1                 | 2                 |
| 63  | ZrMo <sub>2</sub> O <sub>8</sub> 40<br>HfMo <sub>2</sub> O <sub>8</sub> 40 | —                  | 10                 | 5                    |                  |                  |                  |                       | 5                 |                   |                   |
| 64  | ZrMo <sub>2</sub> O <sub>8</sub> 40<br>HfMo <sub>2</sub> O <sub>8</sub> 40 | —                  | 10                 | 1                    | 2                | 1                | 1                | 1                     | 1                 | 1                 | 2                 |

TABLE 6

(Ex. 1 - Group E)

Composition

| NOs | Molybdates<br>(wt. %)            | Glass A<br>(wt. %) | Glass B<br>(wt. %) | Fluorides<br>(wt. %) |                  |                  |                  | Carbonate<br>(%)  |                   |                   |                   |
|-----|----------------------------------|--------------------|--------------------|----------------------|------------------|------------------|------------------|-------------------|-------------------|-------------------|-------------------|
|     |                                  |                    |                    | SrF <sub>2</sub>     | BaF <sub>2</sub> | MgF <sub>2</sub> | CaF <sub>2</sub> | SrCO <sub>3</sub> | BaCO <sub>3</sub> | MgCO <sub>3</sub> | CaCO <sub>3</sub> |
|     | Y <sub>6</sub> MoO <sub>12</sub> |                    |                    |                      |                  |                  |                  |                   |                   |                   |                   |
| 1   | 33.4                             | 50                 | —                  |                      |                  |                  | 8.3              | 8.3               |                   |                   |                   |
| 2   | 45.9                             | 37.5               | —                  |                      |                  |                  | 8.3              | 8.3               |                   |                   |                   |
| 3   | 62.5                             | 20.9               | —                  |                      |                  |                  | 8.3              | 8.3               |                   |                   |                   |
| 4   | 80                               | 3.4                | —                  |                      |                  |                  | 8.3              | 8.3               |                   |                   |                   |
| 5   | 45.9                             | —                  | 37.5               |                      |                  |                  | 8.3              | 8.3               |                   |                   |                   |
| 6   | 62.5                             | —                  | 20.9               |                      |                  |                  | 8.3              | 8.3               |                   |                   |                   |
| 7   | 50                               | —                  | 49                 | 0.5                  |                  |                  |                  |                   | 0.5               |                   |                   |
| 8   | 50                               | —                  | 20                 | 10                   |                  |                  |                  |                   | 20                |                   |                   |
| 9   | 50                               | —                  | 4                  | 1                    |                  |                  |                  |                   | 45                |                   |                   |
| 10  | 65                               | —                  | 10                 | 15                   |                  |                  |                  |                   | 10                |                   |                   |
| 11  | 65                               | —                  | 20                 | 10                   |                  |                  |                  |                   | 5                 |                   |                   |
| 12  | 80                               | —                  | 10                 | 5                    |                  |                  |                  |                   | 5                 |                   |                   |
| 13  | 80                               | —                  | 5                  | 7.5                  |                  |                  |                  |                   | 7.5               |                   |                   |
| 14  | 95                               | —                  | 4                  | 0.5                  |                  |                  |                  |                   | 0.5               |                   |                   |
| 15  | 50                               | —                  | 49                 |                      |                  |                  | 0.5              |                   | 0.5               |                   |                   |
| 16  | 50                               | —                  | 20                 |                      |                  |                  | 10               |                   | 20                |                   |                   |
| 17  | 50                               | —                  | 4                  |                      |                  |                  | 1                |                   | 45                |                   |                   |
| 18  | 65                               | —                  | 10                 |                      |                  |                  | 15               |                   | 10                |                   |                   |
| 19  | 65                               | —                  | 20                 |                      |                  |                  | 10               |                   | 5                 |                   |                   |
| 20  | 80                               | —                  | 10                 |                      |                  |                  | 5                |                   | 5                 |                   |                   |
| 21  | 80                               | —                  | 5                  |                      |                  |                  | 7.5              |                   | 7.5               |                   |                   |
| 22  | 95                               | —                  | 4                  |                      |                  |                  | 0.5              |                   | 0.5               |                   |                   |
| 23  | 50                               | —                  | 20                 | 10                   |                  |                  |                  |                   | 20                |                   |                   |
| 24  | 80                               | —                  | 10                 | 5                    |                  |                  |                  |                   | 5                 |                   |                   |
| 25  | 50                               | —                  | 20                 | 10                   |                  |                  |                  | 20                |                   |                   |                   |
| 26  | 80                               | —                  | 10                 | 5                    |                  |                  |                  | 10                |                   |                   |                   |
| 27  | 50                               | —                  | 20                 | 10                   |                  |                  |                  | 20                |                   |                   |                   |
| 28  | 80                               | —                  | 10                 | 5                    |                  |                  |                  | 5                 |                   |                   |                   |
| 29  | 65                               | —                  | 20                 |                      |                  |                  | 10               |                   |                   | 5                 |                   |
| 30  | 80                               | —                  | 10                 |                      |                  |                  | 5                |                   |                   | 5                 |                   |
| 31  | 65                               | —                  | 20                 |                      |                  |                  | 10               |                   |                   | 5                 |                   |
| 32  | 80                               | —                  | 10                 |                      |                  |                  | 5                |                   |                   | 5                 |                   |
| 33  | 65                               | —                  | 20                 |                      |                  |                  | 10               |                   |                   | 5                 |                   |
| 34  | 80                               | —                  | 10                 |                      |                  |                  | 5                |                   |                   | 5                 |                   |
| 35  | 50                               | —                  | 20                 | 10                   |                  |                  |                  |                   | 10                | 10                |                   |

TABLE 6-continued

| NOS                                   | Molybdates<br>(wt. %) | (Ex. 1 - Group E)<br>Composition |                    |                      |                  |                  |                  |                   |                   |                   |
|---------------------------------------|-----------------------|----------------------------------|--------------------|----------------------|------------------|------------------|------------------|-------------------|-------------------|-------------------|
|                                       |                       | Glass A<br>(wt. %)               | Glass B<br>(wt. %) | Fluorides<br>(wt. %) |                  |                  |                  | Carbonate<br>(%)  |                   |                   |
|                                       |                       |                                  |                    | SrF <sub>2</sub>     | BaF <sub>2</sub> | MgF <sub>2</sub> | CaF <sub>2</sub> | SrCO <sub>3</sub> | BaCO <sub>3</sub> | MgCO <sub>3</sub> |
| 36                                    | 50                    | —                                | 20                 | 5                    | 5                |                  |                  | 10                | 10                |                   |
| 37                                    | 50                    | —                                | 20                 | 3                    | 4                | 3                |                  | 5                 | 5                 | 10                |
| 38                                    | 50                    | —                                | 20                 | 3                    | 3                | 2                | 2                | 5                 | 5                 | 5                 |
| <u>La<sub>6</sub>MoO<sub>12</sub></u> |                       |                                  |                    |                      |                  |                  |                  |                   |                   |                   |
| 39                                    | 33.4                  | —                                | 50                 |                      |                  |                  |                  | 8.3               | 8.3               |                   |
| 40                                    | 45.9                  | —                                | 37.5               |                      |                  |                  |                  | 8.3               | 8.3               |                   |
| 41                                    | 62.5                  | —                                | 20.9               |                      |                  |                  |                  | 8.3               | 8.3               |                   |
| 42                                    | 80                    | —                                | 3.4                |                      |                  |                  |                  | 8.3               | 8.3               |                   |
| 43                                    | 45.9                  | 37.5                             | —                  |                      |                  |                  |                  | 8.3               | 8.3               |                   |
| 44                                    | 62.5                  | 20.9                             | —                  |                      |                  |                  |                  | 8.3               | 8.3               |                   |
| 45                                    | 50                    | —                                | 49                 | 0.5                  |                  |                  |                  |                   |                   | 0.5               |
| 46                                    | 50                    | —                                | 20                 | 10                   |                  |                  |                  |                   |                   | 20                |
| 47                                    | 50                    | —                                | 4                  | 1                    |                  |                  |                  |                   |                   | 45                |
| 48                                    | 65                    | —                                | 10                 | 15                   |                  |                  |                  |                   |                   | 10                |
| 49                                    | 65                    | —                                | 20                 | 10                   |                  |                  |                  |                   |                   | 5                 |
| 50                                    | 80                    | —                                | 10                 | 5                    |                  |                  |                  |                   |                   | 5                 |
| 51                                    | 80                    | —                                | 5                  | 7.5                  |                  |                  |                  |                   |                   | 7.5               |
| 52                                    | 95                    | —                                | 4                  | 0.5                  |                  |                  |                  |                   |                   | 0.5               |
| 53                                    | 80                    | —                                | 5                  | 7.5                  |                  |                  |                  |                   |                   | 7.5               |
| 54                                    | 50                    | —                                | 20                 |                      | 5                | 5                |                  |                   |                   | 20                |
| 55                                    | 50                    | —                                | 20                 | 5                    | 5                |                  |                  |                   |                   | 20                |
| 56                                    | 50                    | —                                | 20                 | 4                    | 3                | 3                |                  |                   |                   | 20                |
| <u>Ce<sub>6</sub>MoO<sub>12</sub></u> |                       |                                  |                    |                      |                  |                  |                  |                   |                   |                   |
| 57                                    | 45.9                  | 37.5                             | —                  |                      |                  |                  |                  | 8.3               | 8.3               |                   |
| 58                                    | 62.5                  | —                                | 20.9               |                      |                  |                  |                  | 8.3               | 8.3               |                   |
| 59                                    | 80                    | —                                | 5                  | 7.5                  |                  |                  |                  |                   |                   | 7.5               |
| <u>Pr<sub>6</sub>MoO<sub>12</sub></u> |                       |                                  |                    |                      |                  |                  |                  |                   |                   |                   |
| 60                                    | 45.9                  | 37.5                             | —                  |                      |                  |                  |                  | 8.3               | 8.3               |                   |
| 61                                    | 62.5                  | —                                | 20.9               |                      |                  |                  |                  | 8.3               | 8.3               |                   |
| 62                                    | 80                    | —                                | 5                  | 7.5                  |                  |                  |                  |                   |                   | 7.5               |
| <u>Nd<sub>6</sub>MoO<sub>12</sub></u> |                       |                                  |                    |                      |                  |                  |                  |                   |                   |                   |
| 63                                    | 45.9                  | 37.5                             | —                  |                      |                  |                  |                  | 8.3               | 8.3               |                   |
| 64                                    | 62.5                  | —                                | 20.9               |                      |                  |                  |                  | 8.3               | 8.3               |                   |
| 65                                    | 80                    | —                                | 5                  | 7.5                  |                  |                  |                  |                   |                   | 7.5               |
| <u>Sm<sub>6</sub>MoO<sub>12</sub></u> |                       |                                  |                    |                      |                  |                  |                  |                   |                   |                   |
| 66                                    | 45.9                  | 37.5                             | —                  |                      |                  |                  |                  | 8.3               | 8.3               |                   |
| 67                                    | 62.5                  | —                                | 20.9               |                      |                  |                  |                  | 8.3               | 8.3               |                   |
| 68                                    | 80                    | —                                | 5                  | 7.5                  |                  |                  |                  |                   |                   | 7.5               |
| <u>Eu<sub>6</sub>MoO<sub>12</sub></u> |                       |                                  |                    |                      |                  |                  |                  |                   |                   |                   |
| 69                                    | 45.9                  | 37.5                             | —                  |                      |                  |                  |                  | 8.3               | 8.3               |                   |
| 70                                    | 62.5                  | —                                | 20.9               |                      |                  |                  |                  | 8.3               | 8.3               |                   |
| 71                                    | 80                    | —                                | 5                  | 7.5                  |                  |                  |                  |                   |                   | 7.5               |
| <u>Gd<sub>6</sub>MoO<sub>12</sub></u> |                       |                                  |                    |                      |                  |                  |                  |                   |                   |                   |
| 72                                    | 45.9                  | 37.5                             | —                  |                      |                  |                  |                  | 8.3               | 8.3               |                   |
| 73                                    | 62.5                  | —                                | 20.9               |                      |                  |                  |                  | 8.3               | 8.3               |                   |
| 74                                    | 80                    | —                                | 5                  | 7.5                  |                  |                  |                  |                   |                   | 7.5               |
| <u>Tb<sub>6</sub>MoO<sub>12</sub></u> |                       |                                  |                    |                      |                  |                  |                  |                   |                   |                   |
| 75                                    | 45.9                  | 37.5                             | —                  |                      |                  |                  |                  | 8.3               | 8.3               |                   |
| 76                                    | 62.5                  | —                                | 20.9               |                      |                  |                  |                  | 8.3               | 8.3               |                   |
| 77                                    | 80                    | —                                | 5                  | 7.5                  |                  |                  |                  |                   |                   | 7.5               |
| <u>Dy<sub>6</sub>MoO<sub>12</sub></u> |                       |                                  |                    |                      |                  |                  |                  |                   |                   |                   |
| 78                                    | 45.9                  | 37.5                             | —                  |                      |                  |                  |                  | 8.3               | 8.3               |                   |
| 79                                    | 62.5                  | —                                | 20.9               |                      |                  |                  |                  | 8.3               | 8.3               |                   |
| 80                                    | 80                    | —                                | 5                  | 7.5                  |                  |                  |                  |                   |                   | 7.5               |
| <u>Ho<sub>6</sub>MoO<sub>12</sub></u> |                       |                                  |                    |                      |                  |                  |                  |                   |                   |                   |
| 81                                    | 45.9                  | 37.5                             | —                  |                      |                  |                  |                  | 8.3               | 8.3               |                   |
| 82                                    | 62.5                  | —                                | 20.9               |                      |                  |                  |                  | 8.3               | 8.3               |                   |
| 83                                    | 80                    | —                                | 5                  | 7.5                  |                  |                  |                  |                   |                   | 7.5               |
| <u>Er<sub>6</sub>MoO<sub>12</sub></u> |                       |                                  |                    |                      |                  |                  |                  |                   |                   |                   |
| 84                                    | 45.9                  | 37.5                             | —                  |                      |                  |                  |                  | 8.3               | 8.3               |                   |
| 85                                    | 62.5                  | —                                | 20.9               |                      |                  |                  |                  | 8.3               | 8.3               |                   |
| 86                                    | 80                    | —                                | 5                  | 7.5                  |                  |                  |                  |                   |                   | 7.5               |
| <u>Tm<sub>6</sub>MoO<sub>12</sub></u> |                       |                                  |                    |                      |                  |                  |                  |                   |                   |                   |
| 87                                    | 45.9                  | 37.5                             | —                  |                      |                  |                  |                  | 8.3               | 8.3               |                   |
| 88                                    | 62.5                  | —                                | 20.9               |                      |                  |                  |                  | 8.3               | 8.3               |                   |
| 89                                    | 80                    | —                                | 5                  | 7.5                  |                  |                  |                  |                   |                   | 7.5               |
| <u>Yb<sub>6</sub>MoO<sub>12</sub></u> |                       |                                  |                    |                      |                  |                  |                  |                   |                   |                   |
| 90                                    | 45.9                  | 37.5                             | —                  |                      |                  |                  |                  | 8.3               | 8.3               |                   |
| 91                                    | 62.5                  | —                                | 20.9               |                      |                  |                  |                  | 8.3               | 8.3               |                   |
| 92                                    | 80                    | —                                | 5                  | 7.5                  |                  |                  |                  |                   |                   | 7.5               |
| <u>Lu<sub>6</sub>MoO<sub>12</sub></u> |                       |                                  |                    |                      |                  |                  |                  |                   |                   |                   |
| 93                                    | 45.9                  | 37.5                             | —                  |                      |                  |                  |                  | 8.3               | 8.3               |                   |
| 94                                    | 62.5                  | —                                | 20.9               |                      |                  |                  |                  | 8.3               | 8.3               |                   |

TABLE 6-continued

| NOs | Molybdates<br>(wt. %)                                                           | Composition        |                    |                      |                  |                  |                   | Carbonate<br>(%)  |                   |                   |
|-----|---------------------------------------------------------------------------------|--------------------|--------------------|----------------------|------------------|------------------|-------------------|-------------------|-------------------|-------------------|
|     |                                                                                 | Glass A<br>(wt. %) | Glass B<br>(wt. %) | Fluorides<br>(wt. %) |                  |                  | SrCO <sub>3</sub> | BaCO <sub>3</sub> | MgCO <sub>3</sub> | CaCO <sub>3</sub> |
|     |                                                                                 |                    |                    | SrF <sub>2</sub>     | BaF <sub>2</sub> | MgF <sub>2</sub> |                   |                   |                   |                   |
| 95  | 80                                                                              | —                  | —                  | 5                    | 7.5              | —                | —                 | —                 | —                 | 7.5               |
| 96  | (Y <sub>3.0</sub> Ce <sub>3.0</sub> )MoO <sub>12</sub> 65                       | —                  | —                  | 20                   | 10               | —                | —                 | 5                 | —                 | —                 |
| 97  | (Pr <sub>3.0</sub> Eu <sub>3.0</sub> )MoO <sub>12</sub> 65                      | —                  | —                  | 20                   | 10               | —                | —                 | 5                 | —                 | —                 |
| 98  | (Gd <sub>3.0</sub> Dy <sub>3.0</sub> )MoO <sub>12</sub> 65                      | —                  | —                  | 20                   | 10               | —                | —                 | 5                 | —                 | —                 |
| 99  | (La <sub>2.0</sub> Nd <sub>2.0</sub> Tb <sub>2.0</sub> )MoO <sub>12</sub><br>65 | —                  | —                  | 20                   | 10               | —                | —                 | 5                 | —                 | —                 |
| 100 | (Ho <sub>2.0</sub> Tm <sub>2.0</sub> Yb <sub>2.0</sub> )MoO <sub>12</sub><br>65 | —                  | —                  | 20                   | 10               | —                | —                 | 5                 | —                 | —                 |
| 101 | Y <sub>6</sub> MoO <sub>12</sub> 40                                             | —                  | —                  | 5                    | —                | —                | 7.5               | 7.5               | —                 | —                 |
|     | La <sub>6</sub> MoO <sub>12</sub> 40                                            | —                  | —                  | —                    | —                | —                | —                 | —                 | —                 | —                 |
| 102 | Nd <sub>6</sub> MoO <sub>12</sub> 40                                            | —                  | —                  | 5                    | —                | —                | 7.5               | 7.5               | —                 | —                 |
|     | Sm <sub>6</sub> MoO <sub>12</sub> 40                                            | —                  | —                  | —                    | —                | —                | —                 | —                 | —                 | —                 |
| 103 | Gd <sub>6</sub> MoO <sub>12</sub> 40                                            | —                  | —                  | 5                    | —                | —                | 7.5               | 7.5               | —                 | —                 |
|     | Dy <sub>6</sub> MoO <sub>12</sub> 40                                            | —                  | —                  | —                    | —                | —                | —                 | —                 | —                 | —                 |
| 104 | Ho <sub>6</sub> MoO <sub>12</sub> 20                                            | —                  | —                  | 5                    | —                | —                | 7.5               | 7.5               | —                 | —                 |
|     | Er <sub>6</sub> MoO <sub>12</sub> 30                                            | —                  | —                  | —                    | —                | —                | —                 | —                 | —                 | —                 |
|     | Tm <sub>6</sub> MoO <sub>12</sub> 30                                            | —                  | —                  | —                    | —                | —                | —                 | —                 | —                 | —                 |
| 105 | Yb <sub>6</sub> MoO <sub>12</sub> 20                                            | —                  | —                  | 5                    | —                | —                | 7.5               | 7.5               | —                 | —                 |
|     | Lu <sub>6</sub> MoO <sub>12</sub> 30                                            | —                  | —                  | —                    | —                | —                | —                 | —                 | —                 | —                 |
|     | Eu <sub>6</sub> MoO <sub>12</sub> 30                                            | —                  | —                  | —                    | —                | —                | —                 | —                 | —                 | —                 |

TABLE 7

| NOs | Molybdates<br>Nb <sub>2</sub> Mo <sub>3</sub> O <sub>14</sub><br>(wt. %) | Composition        |                    |                      |                  |                  |                   | Carbonates<br>(wt. %) |                   |                   |
|-----|--------------------------------------------------------------------------|--------------------|--------------------|----------------------|------------------|------------------|-------------------|-----------------------|-------------------|-------------------|
|     |                                                                          | Glass A<br>(wt. %) | Glass B<br>(wt. %) | Fluorides<br>(wt. %) |                  |                  | SrCO <sub>3</sub> | BaCO <sub>3</sub>     | MgCO <sub>3</sub> | CaCO <sub>3</sub> |
|     |                                                                          |                    |                    | SrF <sub>2</sub>     | BaF <sub>2</sub> | MgF <sub>2</sub> |                   |                       |                   |                   |
| 1   | 37.5                                                                     | —                  | 45.9               | —                    | —                | —                | 8.3               | 8.3                   | —                 | —                 |
| 2   | 54.2                                                                     | —                  | 29.2               | —                    | —                | —                | 8.3               | 8.3                   | —                 | —                 |
| 3   | 66.7                                                                     | —                  | 16.7               | —                    | —                | —                | 8.3               | 8.3                   | —                 | —                 |
| 4   | 80                                                                       | —                  | 3.4                | —                    | —                | —                | 8.3               | 8.3                   | —                 | —                 |
| 5   | 54.2                                                                     | —                  | —                  | 29.2                 | —                | —                | 8.3               | 8.3                   | —                 | —                 |
| 6   | 66.7                                                                     | —                  | —                  | 16.7                 | —                | —                | 8.3               | 8.3                   | —                 | —                 |
| 7   | 55                                                                       | —                  | —                  | 44                   | 0.5              | —                | —                 | —                     | 0.5               | —                 |
| 8   | 55                                                                       | —                  | —                  | 4                    | 1                | —                | —                 | —                     | 40                | —                 |
| 9   | 70                                                                       | —                  | —                  | 10                   | 15               | —                | —                 | —                     | 5                 | —                 |
| 10  | 70                                                                       | —                  | —                  | 10                   | 5                | —                | —                 | —                     | 15                | —                 |
| 11  | 80                                                                       | —                  | —                  | 7                    | 3                | —                | —                 | —                     | 10                | —                 |
| 12  | 95                                                                       | —                  | —                  | 4                    | 0.5              | —                | —                 | —                     | 0.5               | —                 |
| 13  | 70                                                                       | —                  | —                  | 10                   | 15               | —                | —                 | —                     | 5                 | —                 |
| 14  | 80                                                                       | —                  | —                  | 7                    | 3                | —                | —                 | —                     | 10                | —                 |
| 15  | 70                                                                       | —                  | —                  | 10                   | 15               | —                | 5                 | —                     | —                 | —                 |
| 16  | 80                                                                       | —                  | —                  | 7                    | 3                | —                | 10                | —                     | —                 | —                 |
| 17  | 70                                                                       | —                  | —                  | 10                   | 15               | —                | —                 | 5                     | —                 | —                 |
| 18  | 80                                                                       | —                  | —                  | 7                    | 3                | —                | 10                | —                     | —                 | —                 |
| 19  | 55                                                                       | —                  | —                  | 4                    | —                | 1                | —                 | —                     | 40                | —                 |
| 20  | 70                                                                       | —                  | —                  | 10                   | —                | 5                | —                 | —                     | 15                | —                 |
| 21  | 55                                                                       | —                  | —                  | 4                    | —                | —                | 1                 | —                     | 40                | —                 |
| 22  | 70                                                                       | —                  | —                  | 10                   | —                | —                | 5                 | —                     | 15                | —                 |
| 23  | 55                                                                       | —                  | —                  | 4                    | 1                | —                | —                 | —                     | 40                | —                 |
| 24  | 70                                                                       | —                  | —                  | 10                   | 5                | —                | —                 | —                     | 15                | —                 |
| 25  | 70                                                                       | —                  | —                  | 10                   | —                | 5                | —                 | 10                    | —                 | 5                 |
| 26  | 70                                                                       | —                  | —                  | 10                   | 2.5              | —                | 2.5               | 5                     | —                 | 5                 |
|     | <u>Ta<sub>2</sub>Mo<sub>3</sub>O<sub>14</sub></u>                        | —                  | —                  | —                    | —                | —                | —                 | —                     | —                 | —                 |
| 27  | 37.5                                                                     | —                  | —                  | 45.9                 | —                | —                | 8.3               | 8.3                   | —                 | —                 |
| 28  | 54.2                                                                     | —                  | —                  | 29.2                 | —                | —                | 8.3               | 8.3                   | —                 | —                 |
| 29  | 66.7                                                                     | —                  | —                  | 16.7                 | —                | —                | 8.3               | 8.3                   | —                 | —                 |
| 30  | 80                                                                       | —                  | —                  | 3.4                  | —                | —                | 8.3               | 8.3                   | —                 | —                 |
| 31  | 54.2                                                                     | 29.2               | —                  | —                    | —                | —                | 8.3               | 8.3                   | —                 | —                 |
| 32  | 66.7                                                                     | 16.7               | —                  | —                    | —                | —                | 8.3               | 8.3                   | —                 | —                 |
| 33  | 55                                                                       | —                  | —                  | 44                   | —                | —                | 0.5               | 0.5                   | —                 | —                 |
| 34  | 55                                                                       | —                  | —                  | 4                    | —                | —                | 1                 | 40                    | —                 | —                 |
| 35  | 70                                                                       | —                  | —                  | 10                   | —                | —                | 15                | 5                     | —                 | —                 |
| 36  | 70                                                                       | —                  | —                  | 10                   | —                | —                | 5                 | 15                    | —                 | —                 |
| 37  | 80                                                                       | —                  | —                  | 7                    | —                | —                | 3                 | 10                    | —                 | —                 |
| 38  | 95                                                                       | —                  | —                  | 4                    | —                | —                | 0.5               | 0.5                   | —                 | —                 |
| 39  | 70                                                                       | —                  | —                  | 10                   | —                | —                | 15                | —                     | 5                 | —                 |
| 40  | 80                                                                       | —                  | —                  | 7                    | —                | —                | 3                 | —                     | 10                | —                 |
| 41  | 70                                                                       | —                  | —                  | 10                   | —                | —                | 15                | —                     | 5                 | —                 |
| 42  | 80                                                                       | —                  | —                  | 7                    | —                | —                | 3                 | —                     | 10                | —                 |
| 43  | 70                                                                       | —                  | —                  | 10                   | —                | —                | 15                | 5                     | —                 | —                 |

TABLE 7-continued

| NOS | Molybdates<br>$\text{Nb}_2\text{Mo}_3\text{O}_{14}$<br>(wt. %) | Composition        |                    |                      |     |                       |                  |                  |                  |                   |                   |                   |
|-----|----------------------------------------------------------------|--------------------|--------------------|----------------------|-----|-----------------------|------------------|------------------|------------------|-------------------|-------------------|-------------------|
|     |                                                                | (Ex. 1 - Group F)  |                    |                      |     | Carbonates<br>(wt. %) |                  |                  |                  |                   |                   |                   |
|     |                                                                | Glass A<br>(wt. %) | Glass B<br>(wt. %) | Fluorides<br>(wt. %) |     | SrF <sub>2</sub>      | BaF <sub>2</sub> | MgF <sub>2</sub> | CaF <sub>2</sub> | SrCO <sub>3</sub> | BaCO <sub>3</sub> | MgCO <sub>3</sub> |
| 44  | 80                                                             | —                  | 7                  |                      |     |                       |                  | 3                |                  | 10                |                   |                   |
| 45  | 55                                                             | —                  | 4                  |                      |     |                       | 1                |                  |                  | 40                |                   |                   |
| 46  | 70                                                             | —                  | 10                 |                      |     |                       | 5                |                  |                  | 15                |                   |                   |
| 47  | 55                                                             | —                  | 4                  | 1                    |     |                       |                  |                  |                  | 40                |                   |                   |
| 48  | 70                                                             | —                  | 10                 | 5                    |     |                       |                  |                  |                  | 15                |                   |                   |
| 49  | 55                                                             | —                  | 4                  |                      | 1   |                       |                  |                  |                  | 40                |                   |                   |
| 50  | 70                                                             | —                  | 10                 |                      | 5   |                       |                  |                  |                  | 15                |                   |                   |
| 51  | 70                                                             | —                  | 10                 |                      | 2.5 |                       |                  | 2.5              | 10               |                   |                   | 5                 |
| 52  | 70                                                             | —                  | 10                 | 2                    | 2   | 1                     |                  |                  |                  | 5                 | 5                 |                   |
| 53  | $(\text{Nb}_{1.0}\text{Ta}_{1.0})\text{Mo}_3\text{O}_{14}$     | 7                  | 1                  | 1                    | 0.5 | 0.5                   | 0.5              | 3                | 3                | 2                 | 2                 |                   |
|     | 80                                                             |                    |                    |                      |     |                       |                  |                  |                  |                   |                   |                   |
| 54  | $\text{Nb}_2\text{Mo}_3\text{O}_{14}$ 40                       | —                  | 7                  | 1                    | 1   | 0.5                   | 0.5              | 3                | 3                | 2                 | 2                 |                   |
|     | $\text{Ta}_2\text{Mo}_3\text{O}_{14}$ 40                       |                    |                    |                      |     |                       |                  |                  |                  |                   |                   |                   |

TABLE 8

| Nos | Molybdate<br>$\text{MnMoO}_4$<br>(wt. %) | Composition           |                       |                      |     |                       |                  |                  |                  | Carbonates<br>(wt. %) |                   |                   |
|-----|------------------------------------------|-----------------------|-----------------------|----------------------|-----|-----------------------|------------------|------------------|------------------|-----------------------|-------------------|-------------------|
|     |                                          | (Ex. 1-Group G)       |                       |                      |     | Carbonates<br>(wt. %) |                  |                  |                  |                       |                   |                   |
|     |                                          | Glass<br>A<br>(wt. %) | Glass<br>B<br>(wt. %) | Fluorides<br>(wt. %) |     | SrF <sub>2</sub>      | BaF <sub>2</sub> | MgF <sub>2</sub> | CaF <sub>2</sub> | SrCO <sub>3</sub>     | BaCO <sub>3</sub> | MgCO <sub>3</sub> |
| 1   | 41.7                                     | 41.7                  | —                     |                      |     |                       |                  | 8.3              | 8.3              |                       |                   |                   |
| 2   | 54.2                                     | 29.2                  | —                     |                      |     |                       |                  | 8.3              | 8.3              |                       |                   |                   |
| 3   | 66.7                                     | 16.7                  | —                     |                      |     |                       |                  | 8.3              | 8.3              |                       |                   |                   |
| 4   | 80                                       | 3.4                   | —                     |                      |     |                       |                  | 8.3              | 8.3              |                       |                   |                   |
| 5   | 41.7                                     | —                     | 41.7                  |                      |     |                       |                  | 8.3              | 8.3              |                       |                   |                   |
| 6   | 54.2                                     | —                     | 29.2                  |                      |     |                       |                  | 8.3              | 8.3              |                       |                   |                   |
| 7   | 66.7                                     | —                     | 16.7                  |                      |     |                       |                  | 8.3              | 8.3              |                       |                   |                   |
| 8   | 80                                       | —                     | 3.4                   |                      |     |                       |                  | 8.3              | 8.3              |                       |                   |                   |
| 9   | 66.8                                     | 8.3                   | 8.3                   |                      |     |                       |                  | 8.3              | 8.3              |                       |                   |                   |
| 10  | 65                                       | —                     | 34                    |                      | 0.5 |                       |                  | 0.5              |                  |                       |                   |                   |
| 11  | 65                                       | —                     | 5                     |                      | 5   |                       |                  |                  | 25               |                       |                   |                   |
| 12  | 75                                       | —                     | 10                    |                      | 5   |                       |                  |                  | 10               |                       |                   |                   |
| 13  | 75                                       | —                     | 5                     |                      | 15  |                       |                  |                  | 5                |                       |                   |                   |
| 14  | 85                                       | —                     | 7                     |                      | 3   |                       |                  |                  | 5                |                       |                   |                   |
| 15  | 95                                       | —                     | 4                     |                      | 0.5 |                       |                  | 0.5              |                  |                       |                   |                   |
| 16  | 65                                       | —                     | 34                    |                      |     | 0.5                   |                  |                  |                  | 0.5                   |                   |                   |
| 17  | 65                                       | —                     | 5                     |                      |     | 5                     |                  |                  |                  | 25                    |                   |                   |
| 18  | 75                                       | —                     | 10                    |                      |     | 5                     |                  |                  |                  | 10                    |                   |                   |
| 19  | 75                                       | —                     | 5                     |                      |     | 15                    |                  |                  |                  | 5                     |                   |                   |
| 20  | 85                                       | —                     | 7                     |                      |     | 3                     |                  |                  |                  | 5                     |                   |                   |
| 21  | 95                                       | —                     | 4                     |                      |     | 0.5                   |                  |                  | 0.5              |                       |                   |                   |
| 22  | 75                                       | —                     | 10                    |                      | 5   |                       |                  |                  |                  | 10                    |                   |                   |
| 23  | 85                                       | —                     | 7                     |                      | 3   |                       |                  |                  |                  | 5                     |                   |                   |
| 24  | 75                                       | —                     | 10                    |                      | 5   |                       |                  |                  |                  |                       | 10                |                   |
| 25  | 85                                       | —                     | 7                     |                      | 3   |                       |                  |                  |                  |                       | 5                 |                   |
| 26  | 75                                       | —                     | 10                    |                      | 5   |                       |                  |                  | 10               |                       |                   |                   |
| 27  | 85                                       | —                     | 7                     |                      | 3   |                       |                  |                  | 5                |                       |                   |                   |
| 28  | 75                                       | —                     | 5                     |                      |     | 15                    |                  |                  |                  | 5                     |                   |                   |
| 29  | 85                                       | —                     | 7                     |                      |     | 3                     |                  |                  |                  | 5                     |                   |                   |
| 30  | 75                                       | —                     | 5                     | 15                   |     |                       |                  |                  |                  |                       |                   |                   |
| 31  | 85                                       | —                     | 7                     | 3                    |     |                       |                  |                  |                  |                       |                   |                   |
| 32  | 75                                       | —                     | 5                     |                      | 15  |                       |                  |                  |                  |                       |                   |                   |
| 33  | 85                                       | —                     | 7                     |                      | 3   |                       |                  |                  |                  |                       |                   |                   |
| 34  | 65                                       | —                     | 5                     |                      | 5   |                       |                  |                  | 15               |                       |                   |                   |
| 35  | 65                                       | —                     | 5                     | 2.5                  |     | 2.5                   |                  | 15               |                  | 10                    |                   |                   |
| 36  | 65                                       | —                     | 7                     | 1                    | 1   | 1                     |                  | 10               |                  | 5                     |                   |                   |
|     |                                          |                       |                       |                      |     |                       |                  |                  |                  |                       |                   |                   |

TABLE 9

| Nos | A                                     | B                        | C                                   | D                                             | E                                 | F | G                                     | Glass |   | Fluo-                  | Car-                    |
|-----|---------------------------------------|--------------------------|-------------------------------------|-----------------------------------------------|-----------------------------------|---|---------------------------------------|-------|---|------------------------|-------------------------|
|     |                                       |                          |                                     |                                               |                                   |   |                                       | A     | B |                        |                         |
| 1   | $\text{MgMoO}_4$<br>24.7              | $\text{ZnMoO}_4$<br>24.8 |                                     |                                               |                                   |   |                                       |       |   | $\text{MgF}_2$<br>49.5 | $\text{MgCo}_3$<br>0.5  |
| 2   | $\text{CaMoO}_4$<br>25.0              |                          | $\text{Y}_6\text{MoO}_{12}$<br>25.0 |                                               |                                   |   |                                       |       |   | $\text{MgF}_2$<br>33.3 | $\text{MgCo}_3$<br>8.3  |
| 3   | $\text{SrMoO}_4$<br>25.0              |                          |                                     | $\text{Al}_2\text{Mo}_3\text{O}_{12}$<br>25.0 |                                   |   |                                       |       |   | $\text{MgF}_2$<br>21.4 | $\text{MgCo}_3$<br>14.3 |
| 4   | $\text{BaMoO}_4$<br>25.0              |                          |                                     |                                               | $\text{ZrMo}_2\text{O}_8$<br>25.0 |   |                                       |       |   | $\text{MgF}_2$<br>12.5 | $\text{MgCo}_3$<br>18.7 |
| 5   | $\text{Mg}_2\text{Mo}_3\text{O}_{11}$ |                          |                                     |                                               |                                   |   | $\text{Nb}_2\text{Mo}_3\text{O}_{14}$ |       |   | $\text{MgF}_2$<br>12.5 | $\text{MgCo}_3$<br>18.8 |

TABLE 9-continued

(Ex. 1-plural Groups)

| Nos | A                                                       | B                                                       | C                                                       | D                                                       | E                                                       | F                                                       | G                          | Glass       |                          | Fluo-rides                       | Car-bonates              |
|-----|---------------------------------------------------------|---------------------------------------------------------|---------------------------------------------------------|---------------------------------------------------------|---------------------------------------------------------|---------------------------------------------------------|----------------------------|-------------|--------------------------|----------------------------------|--------------------------|
|     |                                                         |                                                         |                                                         |                                                         |                                                         |                                                         |                            | A           | B                        |                                  |                          |
| 6   | 24.2<br>Ca <sub>3</sub> MoO <sub>6</sub><br>47.5        |                                                         |                                                         |                                                         |                                                         | 24.2                                                    | MnMoO <sub>4</sub><br>47.5 | 5.4         | 23.1<br>CaF <sub>2</sub> | 23.1<br>MgCo <sub>3</sub><br>0.5 |                          |
| 7   | ZnMo <sub>2</sub> O <sub>7</sub><br>22.6                | La <sub>2</sub> Mo <sub>2</sub> O <sub>9</sub><br>22.6  |                                                         |                                                         |                                                         |                                                         |                            | 4.0         | 0.5<br>CaF <sub>2</sub>  | 0.5<br>CaCo <sub>3</sub>         |                          |
| 8   | Zn <sub>3</sub> Mo <sub>2</sub> O <sub>9</sub><br>23.1  |                                                         | Al <sub>2</sub> Mo <sub>3</sub> O <sub>12</sub><br>23.1 |                                                         |                                                         |                                                         |                            | 45.3        | 9.0<br>CaF <sub>2</sub>  | 0.5<br>CaCo <sub>3</sub>         |                          |
| 9   | ZnMoO <sub>4</sub><br>23.3                              |                                                         |                                                         | HfMo <sub>2</sub> O <sub>8</sub><br>23.3                |                                                         |                                                         |                            | 30.8        | 15.4<br>CaF <sub>2</sub> | 7.6<br>CaCo <sub>3</sub>         |                          |
| 10  | ZnMo <sub>2</sub> O <sub>7</sub><br>23.1                |                                                         |                                                         | Ta <sub>2</sub> Mo <sub>3</sub> O <sub>14</sub><br>23.1 |                                                         |                                                         |                            | 20.0        | 20.0<br>CaF <sub>2</sub> | 13.4<br>CaCo <sub>3</sub>        |                          |
| 11  | Zn <sub>3</sub> Mo <sub>2</sub> O <sub>9</sub><br>32.0  |                                                         |                                                         |                                                         |                                                         | MnMoO <sub>4</sub><br>32.0                              |                            | 11.6        | 24.9<br>SrF <sub>2</sub> | 17.3<br>CaCo <sub>3</sub>        |                          |
| 12  | CeMo <sub>2</sub> O <sub>8</sub><br>30.0                | Al <sub>2</sub> Mo <sub>3</sub> O <sub>12</sub><br>30.0 |                                                         |                                                         |                                                         |                                                         |                            | 7.1         | 0.4<br>SrF <sub>2</sub>  | 28.5<br>CaCo <sub>3</sub>        |                          |
| 13  | Pr <sub>2</sub> MoO <sub>6</sub><br>20.7                |                                                         | ZrMo <sub>2</sub> O <sub>8</sub><br>20.7                |                                                         |                                                         |                                                         |                            |             | 2.5<br>SrF <sub>2</sub>  | 31.2<br>SrCo <sub>3</sub>        |                          |
| 14  | Nd <sub>2</sub> Mo <sub>3</sub> O <sub>12</sub><br>21.4 |                                                         |                                                         | Nb <sub>2</sub> Mo <sub>3</sub> O <sub>14</sub><br>21.4 |                                                         |                                                         |                            | 41.5        | 16.6<br>SrF <sub>2</sub> | 0.5<br>SrCo <sub>3</sub>         |                          |
| 15  | Sm <sub>6</sub> Mo <sub>12</sub><br>21.5                |                                                         |                                                         |                                                         |                                                         | MnMoO <sub>4</sub><br>21.5                              |                            | 28.6        | 21.4<br>SrF <sub>2</sub> | 7.2<br>SrCo <sub>3</sub>         |                          |
| 16  |                                                         | Al <sub>2</sub> Mo <sub>3</sub> O <sub>12</sub><br>30.7 | HfMo <sub>2</sub> O <sub>8</sub><br>30.7                |                                                         |                                                         |                                                         |                            | 18.4        | 26.4<br>BaF <sub>2</sub> | 12.3<br>SrCo <sub>3</sub>        |                          |
| 17  |                                                         | Al <sub>2</sub> Mo <sub>3</sub> O <sub>12</sub><br>30.0 |                                                         | Ta <sub>2</sub> Mo <sub>3</sub> O <sub>14</sub><br>30.0 |                                                         |                                                         |                            | 15.3        | 0.4<br>BaF <sub>2</sub>  | 22.9<br>SrCo <sub>3</sub>        |                          |
| 18  |                                                         | Al <sub>2</sub> Mo <sub>3</sub> O <sub>12</sub><br>28.2 |                                                         |                                                         | MnMoO <sub>4</sub><br>28.2                              |                                                         |                            | 6.7         | 6.7<br>BaF <sub>2</sub>  | 26.6<br>SrCo <sub>3</sub>        |                          |
| 19  |                                                         |                                                         | ZrMo <sub>2</sub> O <sub>8</sub><br>19.2                | Nb <sub>2</sub> Mo <sub>3</sub> O <sub>14</sub><br>19.2 |                                                         |                                                         |                            | 38.3        | 11.8<br>BaF <sub>2</sub> | 29.4<br>BaCo <sub>3</sub>        |                          |
| 20  |                                                         |                                                         | HfMo <sub>2</sub> O <sub>8</sub><br>19.6                |                                                         | MnMoO <sub>4</sub><br>19.6                              |                                                         |                            | 26.1        | 22.9<br>BaF <sub>2</sub> | 6.6<br>BaCo <sub>3</sub>         |                          |
| 21  |                                                         |                                                         |                                                         | Ta <sub>2</sub> Mo <sub>3</sub> O <sub>14</sub><br>29.0 | MnMoO <sub>4</sub><br>29.0                              |                                                         |                            | 24.9        | 0.4<br>MgF <sub>2</sub>  | 16.7<br>BaCo <sub>3</sub>        |                          |
| 22  | Sr <sub>3</sub> MoO <sub>6</sub><br>28.6                | ZnMoO <sub>4</sub><br>14.3                              | Eu <sub>2</sub> Mo <sub>2</sub> O <sub>7</sub><br>14.3  |                                                         |                                                         |                                                         |                            |             | 14.3<br>MgF <sub>2</sub> | 7.1<br>BaCo <sub>3</sub>         |                          |
| 23  | BaMo <sub>2</sub> O <sub>7</sub><br>18.8                | ZnMo <sub>2</sub> O <sub>7</sub><br>18.8                |                                                         | Al <sub>2</sub> Mo <sub>3</sub> O <sub>12</sub><br>18.8 |                                                         |                                                         |                            |             | 6.1<br>MgF <sub>2</sub>  | 12.5<br>BaCo <sub>3</sub>        |                          |
| 24  | Ba <sub>3</sub> Mo <sub>6</sub><br>22.2                 | Zn <sub>3</sub> Mo <sub>2</sub> O <sub>9</sub><br>22.2  |                                                         |                                                         | ZrMo <sub>2</sub> O <sub>8</sub><br>8.9                 |                                                         |                            |             | 2.2<br>MgF <sub>2</sub>  | 16.7<br>BaCo <sub>3</sub>        |                          |
| 25  | MgMoO <sub>4</sub><br>13.9                              | ZnMoO <sub>4</sub><br>7.0                               |                                                         |                                                         |                                                         | Nb <sub>2</sub> Mo <sub>3</sub> O <sub>14</sub><br>13.9 |                            |             | 34.8<br>MgF <sub>2</sub> | 30.0<br>MgCo <sub>3</sub>        | 0.4                      |
| 26  | Ca <sub>3</sub> MoO <sub>4</sub><br>18.1                | ZnMo <sub>2</sub> O <sub>7</sub><br>18.1                |                                                         |                                                         |                                                         | MnMoO <sub>4</sub><br>18.1                              |                            | 36.2        | 0.5<br>CaF <sub>2</sub>  | 9.0<br>MgCo <sub>3</sub>         |                          |
| 27  | SrMoO <sub>4</sub><br>7.7                               |                                                         | Gd <sub>6</sub> MoO <sub>12</sub><br>23.1               | Al <sub>2</sub> Mo <sub>3</sub> O <sub>12</sub><br>23.1 |                                                         |                                                         |                            |             | 23.1<br>CaF <sub>2</sub> | 7.7<br>MgCo <sub>3</sub>         |                          |
| 28  | BaMo <sub>4</sub> O <sub>13</sub><br>13.3               |                                                         | Tb <sub>2</sub> Mo <sub>3</sub> O <sub>12</sub><br>26.7 |                                                         | HfMo <sub>2</sub> O <sub>8</sub><br>13.3                |                                                         |                            |             | 13.3<br>CaF <sub>2</sub> | 15.3<br>MgCo <sub>3</sub>        |                          |
| 29  | Mg <sub>2</sub> Mo <sub>3</sub> O <sub>11</sub><br>23.5 |                                                         | Dy <sub>2</sub> MoO <sub>6</sub><br>23.5                |                                                         | Ta <sub>2</sub> Mo <sub>3</sub> O <sub>14</sub><br>5.9  |                                                         |                            |             | 5.9<br>CaF <sub>2</sub>  | 13.4<br>MgCo <sub>3</sub>        |                          |
| 30  | Ca <sub>3</sub> MoO <sub>6</sub><br>8.3                 |                                                         | Ho <sub>6</sub> Mo <sub>12</sub><br>20.7                |                                                         |                                                         | MnMoO <sub>4</sub><br>20.7                              |                            | 2.1         | 17.6<br>CaF <sub>2</sub> | 23.6<br>MgCo <sub>3</sub>        |                          |
| 31  | Sr <sub>3</sub> MoO <sub>6</sub><br>9.9                 |                                                         |                                                         | Al <sub>2</sub> Mo <sub>3</sub> O <sub>12</sub><br>29.7 | ZrMo <sub>2</sub> O <sub>8</sub><br>9.9                 |                                                         |                            |             | 49.5<br>SrF <sub>2</sub> | 0.5<br>CaCo <sub>3</sub>         |                          |
| 32  | BaMo <sub>7</sub> O <sub>24</sub><br>8.3                |                                                         |                                                         | Al <sub>2</sub> Mo <sub>3</sub> O <sub>12</sub><br>25.0 |                                                         | Nb <sub>2</sub> Mo <sub>3</sub> O <sub>14</sub><br>16.7 |                            |             | 33.3<br>SrF <sub>2</sub> | 0.5<br>CaCo <sub>3</sub>         |                          |
| 33  | MgMoO <sub>4</sub><br>14.3                              |                                                         |                                                         | Al <sub>2</sub> Mo <sub>3</sub> O <sub>12</sub><br>14.3 |                                                         |                                                         | MnMoO <sub>4</sub><br>21.4 | 21.4        | 14.3<br>SrF <sub>2</sub> | 8.3<br>CaCo <sub>3</sub>         | 14.3                     |
| 34  | CaMoO <sub>4</sub><br>25.0                              |                                                         |                                                         |                                                         | HfMo <sub>2</sub> O <sub>8</sub><br>12.5                | Ta <sub>2</sub> Mo <sub>3</sub> O <sub>14</sub><br>12.5 |                            |             | 12.5<br>SrF <sub>2</sub> | 18.7<br>CaCo <sub>3</sub>        |                          |
| 35  | SrMoO <sub>4</sub><br>16.4                              |                                                         |                                                         |                                                         | ZrMo <sub>2</sub> O <sub>8</sub><br>16.4                |                                                         | MnMoO <sub>4</sub><br>16.4 | 5.5         | 23.5<br>SrF <sub>2</sub> | 21.8<br>CaCo <sub>3</sub>        |                          |
| 36  | BaMoO <sub>4</sub><br>26.6                              |                                                         |                                                         |                                                         |                                                         | Nb <sub>2</sub> Mo <sub>3</sub> O <sub>14</sub><br>10.6 | MnMoO <sub>4</sub><br>20.6 | 2.7         | 0.3<br>BaF <sub>2</sub>  | 33.2<br>CaCo <sub>3</sub>        |                          |
| 37  | Zn <sub>3</sub> Mo <sub>2</sub> O <sub>9</sub><br>18.1  | Er <sub>2</sub> MoO <sub>6</sub><br>18.1                |                                                         | Al <sub>2</sub> Mo <sub>3</sub> O <sub>12</sub><br>9.0  |                                                         |                                                         |                            |             | 45.3<br>BaF <sub>2</sub> | 9.0<br>SrCo <sub>3</sub>         |                          |
| 38  | ZnMoO <sub>4</sub><br>7.7                               | Tm <sub>6</sub> MoO <sub>12</sub><br>23.1               |                                                         |                                                         | HfMo <sub>2</sub> O <sub>8</sub><br>15.4                |                                                         |                            |             | 30.8<br>BaF <sub>2</sub> | 15.3<br>SrCo <sub>3</sub>        |                          |
| 39  | ZnMo <sub>2</sub> O <sub>7</sub><br>6.7                 | Yb <sub>2</sub> Mo <sub>4</sub> O <sub>15</sub><br>13.3 |                                                         |                                                         | Ta <sub>2</sub> Mo <sub>3</sub> O <sub>14</sub><br>26.7 |                                                         |                            |             | 20.0<br>BaF <sub>2</sub> | 20.0<br>SrCo <sub>3</sub>        |                          |
| 40  | Zn <sub>3</sub> Mo <sub>2</sub> O <sub>9</sub><br>12.3  | Lu <sub>2</sub> Mo <sub>3</sub> O <sub>12</sub><br>12.3 |                                                         |                                                         |                                                         | MnMoO <sub>4</sub><br>11.6                              |                            | 11.6        | 11.6<br>BaF <sub>2</sub> | 13.3<br>SrCo <sub>3</sub>        |                          |
| 41  | ZnMoO <sub>4</sub><br>28.5                              |                                                         | Al <sub>2</sub> Mo <sub>3</sub> O <sub>12</sub><br>28.5 | ZrMo <sub>2</sub> O <sub>8</sub><br>7.1                 |                                                         |                                                         |                            |             | 24.9<br>MgF <sub>2</sub> | 17.3<br>SrCo <sub>3</sub>        |                          |
| 42  | ZnMo <sub>2</sub> O <sub>7</sub><br>25.0                |                                                         | Al <sub>2</sub> Mo <sub>3</sub> O <sub>12</sub><br>18.8 |                                                         | Nb <sub>2</sub> Mo <sub>3</sub> O <sub>14</sub><br>16.2 |                                                         |                            |             | 0.4<br>MgF <sub>2</sub>  | 28.4<br>SrCo <sub>3</sub>        |                          |
| 43  | Zn <sub>3</sub> Mo <sub>2</sub> O <sub>9</sub><br>16.6  |                                                         | Al <sub>2</sub> Mo <sub>3</sub> O <sub>12</sub><br>16.6 |                                                         |                                                         | MnMoO <sub>4</sub><br>8.2                               |                            | 2.5<br>41.5 | 6.3<br>16.6              | 31.2<br>MgF <sub>2</sub>         | 0.5<br>BaCo <sub>3</sub> |
| 44  | ZnMoO <sub>4</sub>                                      |                                                         |                                                         | HfMo <sub>2</sub> O <sub>8</sub>                        | Ta <sub>2</sub> Mo <sub>3</sub> O <sub>14</sub>         |                                                         |                            |             | 41.5<br>MgF <sub>2</sub> |                                  | BaCo <sub>3</sub>        |

TABLE 9-continued

| Nos | A                                               | B                                               | C                                | D                                               | E                                               | F                                               | G                                               | Glass                                           |                    | Fluo-<br>rides    | Car-<br>bonates   |                   |
|-----|-------------------------------------------------|-------------------------------------------------|----------------------------------|-------------------------------------------------|-------------------------------------------------|-------------------------------------------------|-------------------------------------------------|-------------------------------------------------|--------------------|-------------------|-------------------|-------------------|
|     |                                                 |                                                 |                                  |                                                 |                                                 |                                                 |                                                 | A                                               | B                  |                   |                   |                   |
| 45  |                                                 | 14.3                                            | ZnMo <sub>2</sub> O <sub>7</sub> |                                                 | 14.3                                            | 14.3                                            |                                                 | 28.6                                            | 21.4               | 7.1               |                   |                   |
|     |                                                 | 18.4                                            |                                  |                                                 | ZrMo <sub>2</sub> O <sub>8</sub>                | 18.4                                            | MnMoO <sub>4</sub>                              |                                                 | MgF <sub>2</sub>   | BaCo <sub>3</sub> |                   |                   |
| 46  |                                                 | Zn <sub>3</sub> Mo <sub>2</sub> O <sub>9</sub>  | 23.0                             |                                                 |                                                 | Nb <sub>2</sub> Mo <sub>3</sub> O <sub>14</sub> | 23.0                                            | 6.1                                             | 18.4               | 12.3              |                   |                   |
|     |                                                 |                                                 |                                  |                                                 |                                                 |                                                 |                                                 | 15.3                                            | 26.4               |                   |                   |                   |
| 47  |                                                 | Y <sub>2</sub> Mo <sub>3</sub> O <sub>12</sub>  | 6.7                              | Al <sub>2</sub> Mo <sub>3</sub> O <sub>12</sub> | 26.7                                            | HfMo <sub>2</sub> O <sub>8</sub>                | 26.7                                            | MnMoO <sub>4</sub>                              |                    | CaF <sub>2</sub>  | BaCo <sub>3</sub> |                   |
|     |                                                 | 29.4                                            |                                  |                                                 |                                                 |                                                 |                                                 |                                                 |                    | 6.7               | 23.0              |                   |
| 48  |                                                 | La <sub>6</sub> Mo <sub>12</sub>                | 9.4                              | Al <sub>2</sub> Mo <sub>3</sub> O <sub>12</sub> |                                                 | Ta <sub>2</sub> Mo <sub>3</sub> O <sub>14</sub> | 17.6                                            |                                                 |                    | 11.8              |                   |                   |
|     |                                                 | 23.0                                            |                                  |                                                 |                                                 |                                                 |                                                 |                                                 |                    | 2.4               | 29.4              |                   |
| 49  |                                                 | Ce <sub>2</sub> Mo <sub>3</sub> O <sub>13</sub> | 7.7                              | Al <sub>2</sub> Mo <sub>3</sub> O <sub>12</sub> |                                                 |                                                 |                                                 | MnMoO <sub>4</sub>                              |                    | CaF <sub>2</sub>  | MgCo <sub>3</sub> |                   |
|     |                                                 | 19.6                                            |                                  |                                                 |                                                 |                                                 |                                                 | 7.7                                             |                    | 23.0              | 0.3               |                   |
| 50  |                                                 | Pr <sub>2</sub> Mo <sub>3</sub> O <sub>12</sub> |                                  |                                                 | ZrMo <sub>2</sub> O <sub>8</sub>                | Nb <sub>2</sub> Mo <sub>3</sub> O <sub>14</sub> |                                                 |                                                 | 38.3               |                   |                   |                   |
|     |                                                 | 24.9                                            |                                  |                                                 | 13.1                                            | 6.5                                             |                                                 |                                                 |                    | 22.1              | 28.1              |                   |
| 51  |                                                 | Nd <sub>2</sub> MoO <sub>4</sub>                |                                  |                                                 | HfMo <sub>2</sub> O <sub>8</sub>                |                                                 | MnMoO <sub>4</sub>                              |                                                 |                    | SrF <sub>2</sub>  | MgCo <sub>3</sub> |                   |
|     |                                                 | 21.4                                            |                                  |                                                 | 24.9                                            |                                                 |                                                 | 8.3                                             |                    | 24.9              | 16.6              |                   |
| 52  |                                                 | Sm <sub>6</sub> MoO <sub>12</sub>               |                                  |                                                 |                                                 | Ta <sub>2</sub> Mo <sub>3</sub> O <sub>14</sub> | 28.6                                            | MnMoO <sub>4</sub>                              |                    | SrF <sub>2</sub>  | MgCo <sub>3</sub> |                   |
|     |                                                 |                                                 |                                  |                                                 |                                                 |                                                 | 7.1                                             |                                                 |                    | 14.3              | 7.1               |                   |
| 53  |                                                 | Al <sub>2</sub> Mo <sub>3</sub> O <sub>12</sub> | 18.7                             | ZrMo <sub>2</sub> O <sub>8</sub>                | Nb <sub>2</sub> Mo <sub>3</sub> O <sub>14</sub> | 18.7                                            |                                                 |                                                 | 6.3                | 12.6              |                   |                   |
|     |                                                 | 16.7                                            |                                  |                                                 |                                                 |                                                 |                                                 |                                                 |                    |                   | 25.0              |                   |
| 54  |                                                 | Al <sub>2</sub> Mo <sub>3</sub> O <sub>12</sub> | 16.7                             | HfMo <sub>2</sub> O <sub>8</sub>                |                                                 |                                                 | 20.0                                            | MnMoO <sub>4</sub>                              |                    | SrF <sub>2</sub>  | MgCo <sub>3</sub> |                   |
|     |                                                 | 7.0                                             |                                  |                                                 |                                                 |                                                 |                                                 |                                                 |                    | 2.2               | 16.7              |                   |
| 55  |                                                 | Al <sub>2</sub> Mo <sub>3</sub> O <sub>12</sub> |                                  |                                                 | Ta <sub>2</sub> Mo <sub>3</sub> O <sub>14</sub> | 13.9                                            | MnMoO <sub>4</sub>                              |                                                 |                    | SrF <sub>2</sub>  | CaCo <sub>3</sub> |                   |
|     |                                                 |                                                 |                                  |                                                 | 17.6                                            | 13.9                                            |                                                 | 34.8                                            |                    | 30.0              | 0.4               |                   |
| 56  |                                                 | ZrMo <sub>2</sub> O <sub>8</sub>                | 9.0                              | Nb <sub>2</sub> Mo <sub>3</sub> O <sub>14</sub> |                                                 | MnMoO <sub>4</sub>                              |                                                 |                                                 |                    | BaF <sub>2</sub>  | CaCo <sub>3</sub> |                   |
|     |                                                 |                                                 |                                  |                                                 |                                                 | 27.1                                            |                                                 |                                                 | 36.2               | 0.5               | 9.1               |                   |
| 57  | Mg <sub>2</sub> Mo <sub>3</sub> O <sub>11</sub> | ZnMoO <sub>4</sub>                              | 15.4                             | EuMoO <sub>4</sub>                              | Al <sub>2</sub> Mo <sub>3</sub> O <sub>12</sub> | 15.4                                            |                                                 |                                                 |                    | BaF <sub>2</sub>  | CaCo <sub>3</sub> |                   |
|     | 7.7                                             |                                                 |                                  |                                                 |                                                 |                                                 |                                                 |                                                 |                    | 23.1              | 7.7               |                   |
| 58  | Ca <sub>3</sub> MoO <sub>6</sub>                | ZnMo <sub>2</sub> O <sub>7</sub>                | 13.3                             | Gd <sub>2</sub> Mo <sub>6</sub> O <sub>21</sub> |                                                 | HfMo <sub>2</sub> O <sub>8</sub>                | 13.3                                            |                                                 |                    | BaF <sub>2</sub>  | CaCo <sub>3</sub> |                   |
|     |                                                 |                                                 |                                  |                                                 |                                                 |                                                 |                                                 |                                                 |                    | 13.3              | 13.4              |                   |
| 59  | Sr <sub>3</sub> MoO <sub>6</sub>                | Zn <sub>3</sub> Mo <sub>2</sub> O <sub>9</sub>  | 8.8                              | Tb <sub>6</sub> MoO <sub>12</sub>               |                                                 | Ta <sub>2</sub> Mo <sub>3</sub> O <sub>14</sub> | 17.6                                            |                                                 |                    | BaF <sub>2</sub>  | CaCo <sub>3</sub> |                   |
|     |                                                 |                                                 |                                  |                                                 |                                                 |                                                 |                                                 |                                                 |                    | 5.9               | 17.6              |                   |
| 60  | Ba <sub>2</sub> MoO <sub>5</sub>                | ZnMoO <sub>4</sub>                              | 15.5                             | Dy <sub>6</sub> MoO <sub>12</sub>               |                                                 |                                                 |                                                 | MnMoO <sub>4</sub>                              |                    | BaF <sub>2</sub>  | CaCo <sub>3</sub> |                   |
|     |                                                 |                                                 |                                  |                                                 |                                                 |                                                 |                                                 | 3.1                                             |                    | 2.1               | 22.3              |                   |
| 61  | MgMoO <sub>4</sub>                              | ZnMo <sub>2</sub> O <sub>7</sub>                | 10                               |                                                 | Al <sub>2</sub> Mo <sub>3</sub> O <sub>12</sub> | ZrMo <sub>2</sub> O <sub>8</sub>                |                                                 |                                                 |                    | MgF <sub>2</sub>  | SrCo <sub>3</sub> |                   |
|     |                                                 |                                                 |                                  |                                                 | 10                                              | 20                                              |                                                 |                                                 |                    | 49.5              | 0.5               |                   |
| 62  | CaMoO <sub>4</sub>                              | Zn <sub>3</sub> Mo <sub>2</sub> O <sub>9</sub>  | 12.5                             |                                                 | Al <sub>2</sub> Mo <sub>3</sub> O <sub>12</sub> |                                                 | Nb <sub>2</sub> Mo <sub>3</sub> O <sub>14</sub> |                                                 |                    | MgF <sub>2</sub>  | SrCo <sub>3</sub> |                   |
|     |                                                 |                                                 |                                  |                                                 | 12.5                                            |                                                 | 12.5                                            |                                                 |                    | 33.3              | 8.3               |                   |
| 63  | SrMoO <sub>4</sub>                              | ZnMoO <sub>4</sub>                              | 14.3                             |                                                 | Al <sub>2</sub> Mo <sub>3</sub> O <sub>12</sub> | 10.7                                            |                                                 | MnMoO <sub>4</sub>                              |                    | MgF <sub>2</sub>  | SrCo <sub>3</sub> |                   |
|     |                                                 |                                                 |                                  |                                                 |                                                 |                                                 |                                                 | 10.7                                            |                    | 21.4              | 14.3              |                   |
| 64  | BaMoO <sub>4</sub>                              | ZnMo <sub>2</sub> O <sub>7</sub>                | 9.4-                             |                                                 |                                                 | HfMo <sub>2</sub> O <sub>8</sub>                | Ta <sub>2</sub> Mo <sub>3</sub> O <sub>14</sub> |                                                 |                    | MgF <sub>2</sub>  | SrCo <sub>3</sub> |                   |
|     |                                                 |                                                 | 15.6                             |                                                 |                                                 | 15.6                                            | 9.4                                             |                                                 |                    | 12.5              | 18.8              |                   |
| 65  | Mg <sub>2</sub> Mo <sub>3</sub> O <sub>11</sub> | Zn <sub>3</sub> Mo <sub>2</sub> O <sub>9</sub>  | 10.9                             |                                                 |                                                 | ZrMo <sub>2</sub> O <sub>8</sub>                | 13.7                                            | MnMoO <sub>4</sub>                              |                    | MgF <sub>2</sub>  | SrCo <sub>3</sub> |                   |
|     |                                                 |                                                 |                                  |                                                 |                                                 |                                                 |                                                 | 13.7                                            |                    | 5.5               | 23.5              |                   |
| 66  | Ca <sub>3</sub> MoO <sub>6</sub>                | ZnMoO <sub>4</sub>                              | 15.9                             |                                                 |                                                 |                                                 | Nb <sub>2</sub> Mo <sub>3</sub> O <sub>14</sub> | MnMoO <sub>4</sub>                              |                    | CaF <sub>2</sub>  | SrCo <sub>3</sub> |                   |
|     |                                                 |                                                 |                                  |                                                 |                                                 |                                                 | 15.9                                            | 15.9                                            |                    | 2.4               | 0.3               |                   |
| 67  | Sr <sub>3</sub> MoO <sub>6</sub>                | Ho <sub>2</sub> Mo <sub>3</sub> O <sub>12</sub> | 9.0                              |                                                 | Al <sub>2</sub> Mo <sub>3</sub> O <sub>12</sub> | HfMo <sub>2</sub> O <sub>8</sub>                | 9.0                                             |                                                 |                    | CaF <sub>2</sub>  | BaCo <sub>3</sub> |                   |
|     |                                                 |                                                 |                                  |                                                 | 13.6                                            | 13.6                                            |                                                 |                                                 |                    | 45.2              | 9.0               |                   |
| 68  | BaMo <sub>3</sub> O <sub>10</sub>               | Er <sub>6</sub> MoO <sub>12</sub>               | 7.7                              |                                                 | Al <sub>2</sub> Mo <sub>3</sub> O <sub>12</sub> | 7.7                                             | Ta <sub>2</sub> Mo <sub>3</sub> O <sub>14</sub> | 15.4                                            |                    | CaF <sub>2</sub>  | BaCo <sub>3</sub> |                   |
|     |                                                 |                                                 |                                  |                                                 |                                                 |                                                 |                                                 |                                                 |                    | 30.8              | 7.6               |                   |
| 69  | MgMoO <sub>4</sub>                              | Tm <sub>2</sub> Mo <sub>6</sub> O <sub>12</sub> | 13.3                             |                                                 | Al <sub>2</sub> Mo <sub>3</sub> O <sub>12</sub> | 10.0                                            |                                                 | MnMoO <sub>4</sub>                              |                    | CaF <sub>2</sub>  | BaCo <sub>3</sub> |                   |
|     |                                                 |                                                 |                                  |                                                 | 10.0                                            | 10.0                                            |                                                 | 13.3                                            |                    | 20.0              | 13.4              |                   |
| 70  | CaMoO <sub>4</sub>                              | Yb <sub>6</sub> MoO <sub>12</sub>               | 17.3                             |                                                 |                                                 | ZrMo <sub>2</sub> O <sub>8</sub>                | Nb <sub>2</sub> Mo <sub>3</sub> O <sub>14</sub> |                                                 |                    | CaF <sub>2</sub>  | BaCo <sub>3</sub> |                   |
|     |                                                 |                                                 |                                  |                                                 |                                                 | 5.8                                             | 5.8                                             |                                                 |                    | 11.6              | 24.9              |                   |
| 71  | SrMoO <sub>4</sub>                              | Lu <sub>6</sub> MoO <sub>12</sub>               | 17.8                             |                                                 |                                                 | HfMo <sub>2</sub> O <sub>8</sub>                |                                                 | MnMoO <sub>4</sub>                              |                    | SrF <sub>2</sub>  | BaCo <sub>3</sub> |                   |
|     |                                                 |                                                 |                                  |                                                 |                                                 | 17.8                                            |                                                 | 14.2                                            |                    | 7.1               | 0.4               |                   |
| 72  | BaMoO <sub>4</sub>                              | Yb <sub>6</sub> MoO <sub>12</sub>               | 18.7                             |                                                 |                                                 | Ta <sub>2</sub> Mo <sub>3</sub> O <sub>14</sub> | 18.7                                            | MnMoO <sub>4</sub>                              |                    | SrF <sub>2</sub>  | BaCo <sub>3</sub> |                   |
|     |                                                 |                                                 |                                  |                                                 |                                                 |                                                 | 3.8                                             |                                                 |                    | 2.5               | 6.3               |                   |
| 73  | Mg <sub>2</sub> Mo <sub>3</sub> O <sub>11</sub> |                                                 | 12.4                             |                                                 | Al <sub>2</sub> Mo <sub>3</sub> O <sub>12</sub> | ZrMo <sub>2</sub> O <sub>8</sub>                | 8.3                                             |                                                 |                    | SrF <sub>2</sub>  | MgCo <sub>3</sub> |                   |
|     |                                                 |                                                 |                                  |                                                 | 12.4                                            |                                                 |                                                 |                                                 |                    | 41.5              | 16.7              |                   |
| 74  | Ca <sub>3</sub> MoO <sub>6</sub>                |                                                 | 7.1                              |                                                 | Al <sub>2</sub> Mo <sub>3</sub> O <sub>12</sub> | HfMo <sub>2</sub> O <sub>8</sub>                | 14.3                                            | MnMoO <sub>4</sub>                              |                    | SrF <sub>2</sub>  | MgCo <sub>3</sub> |                   |
|     |                                                 |                                                 |                                  |                                                 |                                                 |                                                 |                                                 | 7.1                                             |                    | 28.6              | 7.2               |                   |
| 75  | Sr <sub>3</sub> MoO <sub>6</sub>                |                                                 | 12.3                             |                                                 | Al <sub>2</sub> Mo <sub>3</sub> O <sub>12</sub> | 12.3                                            | Ta <sub>2</sub> Mo <sub>3</sub> O <sub>14</sub> | 9.2                                             | MnMoO <sub>4</sub> |                   | SrF <sub>2</sub>  | MgCo <sub>3</sub> |
|     |                                                 |                                                 |                                  |                                                 |                                                 |                                                 |                                                 | 9.2                                             |                    | 18.4              | 26.4              |                   |
| 76  | BaMo <sub>2</sub> O <sub>7</sub>                |                                                 | 15.3                             |                                                 |                                                 | ZrMo <sub>2</sub> O <sub>8</sub>                | 15.3                                            | Nb <sub>2</sub> Mo <sub>3</sub> O <sub>14</sub> | MnMoO <sub>4</sub> |                   | BaF <sub>2</sub>  | MgCo <sub>3</sub> |
|     |                                                 |                                                 |                                  |                                                 |                                                 |                                                 | 15.3                                            | 15.3                                            | 15.3               |                   | 0.4               |                   |
| 77  | ZnMo <sub>2</sub> O <sub>7</sub>                | La <sub>2</sub> Mo <sub>3</sub> O <sub>12</sub> | 13.3                             |                                                 | Al <sub>2</sub> Mo <sub>3</sub> O <sub>12</sub> | HfMo <sub>2</sub> O <sub>8</sub>                |                                                 |                                                 |                    | BaF <sub>2</sub>  | MgCo <sub>3</sub> |                   |
|     |                                                 |                                                 |                                  |                                                 | 6.7                                             | 20.0                                            | 20.0                                            |                                                 |                    | 6.7               | 26.6              |                   |
| 78  | Zn <sub>3</sub> Mo <sub>2</sub> O <sub>9</sub>  | Pr <sub>6</sub> MoO <sub>12</sub>               | 8.8                              |                                                 | Al <sub>2</sub> Mo <sub>3</sub> O <sub>12</sub> |                                                 | Ta <sub>2</sub> Mo <sub>3</sub> O <sub>14</sub> | 12.4                                            |                    | BaF <sub>2</sub>  | MgCo <sub>3</sub> |                   |
|     |                                                 |                                                 |                                  |                                                 | 14.7                                            | 20.6                                            |                                                 |                                                 |                    | 2.4               | 29.4              |                   |
| 79  | ZnMoO <sub>4</sub>                              | Nd <sub>6</sub> MoO <sub>12</sub>               | 7.7                              |                                                 | Al <sub>2</sub> Mo <sub>3</sub> O <sub>12</sub> | 7.7                                             |                                                 | MnMoO <sub>4</sub>                              |                    | BaF <sub>2</sub>  | CaCo <sub>3</sub> |                   |
|     |                                                 |                                                 |                                  |                                                 |                                                 |                                                 |                                                 | 15.3                                            |                    | 38.3              | 0.4               |                   |
| 80  | ZnMo <sub>2</sub> O <sub>7</sub>                | Sm <sub>2</sub> Mo <sub>3</sub> O <sub>12</sub> | 9.8                              |                                                 |                                                 | ZrMo <sub>2</sub> O <sub>8</sub>                | 9.8                                             | Nb <sub>2</sub> Mo <sub>3</sub> O <sub>14</sub> |                    | BaF <sub>2</sub>  | CaCo <sub>3</sub> |                   |
|     |                                                 |                                                 |                                  |                                                 |                                                 | 9.8                                             |                                                 | 9.8                                             |                    | 26.1              | 6.6               |                   |
| 81  | Zn <sub>3</sub> Mo <sub>2</sub> O <sub>9</sub>  | Eu <sub>2</sub> MoO <sub>6</sub>                | 12.4                             |                                                 |                                                 | HfMo <sub>2</sub> O <sub>8</sub>                | 12.4                                            | MnMoO <sub>4</sub>                              |                    | MgF <sub>2</sub>  | CaCo <sub>3</sub> |                   |
|     |                                                 |                                                 |                                  |                                                 |                                                 |                                                 |                                                 |                                                 |                    | 16.6              | 16.1              |                   |
| 82  | ZnMoO <sub>4</sub>                              | Gd <sub>2</sub> Mo <sub>3</sub> O <sub>12</sub> | 14.3                             |                                                 |                                                 | Ta <sub>2</sub> Mo <sub>3</sub> O <sub>14</sub> | 14.3                                            | MnMoO <sub>4</sub>                              |                    | MgF <sub>2</sub>  | CaCo <sub>3</sub> |                   |
|     |                                                 |                                                 |                                  |                                                 |                                                 |                                                 | 14.3                                            | 14.3                                            | 14.3               |                   | 7.1               |                   |
| 83  | ZnMo <sub>2</sub> O <sub>7</sub>                |                                                 |                                  |                                                 | Al <sub>2</sub> Mo <sub>3</sub> O <sub>12</sub> | ZrMo <sub>2</sub> O <sub>8</sub>                |                                                 | Nb <sub>2</sub> Mo <sub>3</sub> O <sub>14</sub> |                    | MgF <sub>2</sub>  | CaCo <sub>3</sub> |                   |

TABLE 9-continued

| Nos | A                                               | B                                              | C                                               | D                                               | E                                | F                                               | G                  | Glass              |      | Fluo-rides       | Car-bonates       |
|-----|-------------------------------------------------|------------------------------------------------|-------------------------------------------------|-------------------------------------------------|----------------------------------|-------------------------------------------------|--------------------|--------------------|------|------------------|-------------------|
|     |                                                 |                                                |                                                 |                                                 |                                  |                                                 |                    | A                  | B    |                  |                   |
| 84  |                                                 |                                                |                                                 | 15.6                                            | 15.6                             | 12.5                                            | 12.5               | MnMoO <sub>4</sub> | 6.3  | 12.5             | 25.0              |
|     | Zn <sub>3</sub> Mo <sub>2</sub> O <sub>9</sub>  |                                                |                                                 | Al <sub>2</sub> Mo <sub>3</sub> O <sub>12</sub> | HfMo <sub>2</sub> O <sub>8</sub> |                                                 |                    |                    |      | MgF <sub>2</sub> | CaCo <sub>3</sub> |
|     |                                                 | 13.3                                           |                                                 | 13.3                                            | 13.3                             |                                                 |                    |                    | 13.3 | 2.2              | 16.7              |
| 85  | ZnMoO <sub>4</sub>                              |                                                |                                                 | Al <sub>2</sub> Mo <sub>3</sub> O <sub>12</sub> |                                  | Ta <sub>2</sub> Mo <sub>3</sub> O <sub>14</sub> | MnMoO <sub>4</sub> |                    |      | MgF <sub>2</sub> | SrCo <sub>3</sub> |
|     | 7.0                                             |                                                |                                                 | 7.0                                             |                                  | 7.0                                             | 13.9               |                    |      | 30.0             | 0.3               |
| 86. | ZnMo <sub>2</sub> O <sub>7</sub>                |                                                |                                                 |                                                 | ZrMo <sub>2</sub> O <sub>8</sub> | Nb <sub>2</sub> Mo <sub>3</sub> O <sub>14</sub> | MnMoO <sub>4</sub> |                    |      | CaF <sub>2</sub> | SrCo <sub>3</sub> |
|     | 13.6                                            |                                                |                                                 |                                                 | 13.6                             | 13.6                                            | 13.6               |                    |      | 0.4              | 9.0               |
| 87  |                                                 |                                                | Tb <sub>2</sub> MoO <sub>6</sub>                | Al <sub>2</sub> Mo <sub>3</sub> O <sub>12</sub> | HfMo <sub>2</sub> O <sub>8</sub> | Ta <sub>2</sub> Mo <sub>3</sub> O <sub>14</sub> |                    |                    |      | CaF <sub>2</sub> | SrCo <sub>3</sub> |
|     |                                                 | 11.5                                           |                                                 | 15.4                                            | 11.5                             | 15.4                                            |                    |                    |      | 7.7              | 15.4              |
| 88  | Dy <sub>2</sub> MoO <sub>6</sub>                |                                                | Al <sub>2</sub> Mo <sub>3</sub> O <sub>12</sub> | ZrMo <sub>2</sub> O <sub>8</sub>                |                                  |                                                 | MnMoO <sub>4</sub> |                    |      | CaF <sub>2</sub> | SrCo <sub>3</sub> |
|     | 13.3                                            |                                                | 13.3                                            | 13.3                                            |                                  |                                                 | 13.3               |                    |      | 13.4             | 20.1              |
| 89  | Ho <sub>2</sub> MoO <sub>6</sub>                |                                                | Al <sub>2</sub> Mo <sub>3</sub> O <sub>12</sub> |                                                 |                                  | Nb <sub>2</sub> Mo <sub>3</sub> O <sub>14</sub> | MnMoO <sub>4</sub> |                    |      | CaF <sub>2</sub> | SrCo <sub>3</sub> |
|     | 11.8                                            |                                                | 11.8                                            |                                                 |                                  | 11.8                                            | 17.6               |                    |      | 17.6             | 23.5              |
| 90  | Er <sub>6</sub> MoO <sub>12</sub>               |                                                |                                                 |                                                 | HfMo <sub>2</sub> O <sub>8</sub> | Ta <sub>2</sub> Mo <sub>3</sub> O <sub>14</sub> | MnMoO <sub>4</sub> |                    |      | CaF <sub>2</sub> | SrCo <sub>3</sub> |
|     | 12.4                                            |                                                |                                                 |                                                 | 12.4                             | 12.4                                            | 12.4               |                    |      | 22.4             | 26.0              |
| 91  |                                                 |                                                | Al <sub>2</sub> Mo <sub>3</sub> O <sub>12</sub> | ZrMo <sub>2</sub> O <sub>8</sub>                |                                  | Nb <sub>2</sub> Mo <sub>3</sub> O <sub>14</sub> | MnMoO <sub>4</sub> |                    |      | SrF <sub>2</sub> | BaCo <sub>3</sub> |
|     |                                                 | 9.9                                            |                                                 | 19.8                                            |                                  | 9.9                                             | 9.9                |                    |      | 0.5              | 0.5               |
| 92  | MgMoO <sub>4</sub>                              | Zn <sub>3</sub> Mo <sub>2</sub> O <sub>9</sub> | Tm <sub>6</sub> MoO <sub>12</sub>               | Al <sub>2</sub> Mo <sub>3</sub> O <sub>12</sub> | HfMo <sub>2</sub> O <sub>8</sub> |                                                 |                    |                    |      | SrF <sub>2</sub> | BaCo <sub>3</sub> |
|     | 8.3                                             | 16.7                                           | 8.3                                             | 8.3                                             | 8.3                              |                                                 |                    |                    |      | 8.3              | 8.4               |
| 93  | CaMoO <sub>4</sub>                              | ZnMoO <sub>4</sub>                             | Yb <sub>6</sub> MoO <sub>12</sub>               | Al <sub>2</sub> Mo <sub>3</sub> O <sub>12</sub> |                                  | Ta <sub>2</sub> Mo <sub>3</sub> O <sub>14</sub> |                    |                    |      | SrF <sub>2</sub> | BaCo <sub>3</sub> |
|     | 7.1                                             | 14.3                                           | 14.3                                            | 7.1                                             |                                  | 7.1                                             |                    |                    |      | 14.3             | 14.3              |
| 94  | SrMoO <sub>4</sub>                              | ZnMo <sub>2</sub> O <sub>7</sub>               | Lu <sub>6</sub> MoO <sub>12</sub>               | Al <sub>2</sub> Mo <sub>3</sub> O <sub>12</sub> |                                  |                                                 | MnMoO <sub>4</sub> |                    |      | SrF <sub>2</sub> | BaCo <sub>3</sub> |
|     | 12.5                                            | 12.5                                           | 12.5                                            | 6.3                                             |                                  |                                                 | 6.3                |                    |      | 18.7             | 18.7              |
| 95  | BaMoO <sub>4</sub>                              | Zn <sub>3</sub> Mo <sub>2</sub> O <sub>9</sub> | Y <sub>2</sub> Mo <sub>3</sub> O <sub>12</sub>  |                                                 | ZrMo <sub>2</sub> O <sub>8</sub> | Nb <sub>2</sub> Mo <sub>3</sub> O <sub>14</sub> |                    |                    |      | SrF <sub>2</sub> | BaCo <sub>3</sub> |
|     | 10.9                                            | 5.5                                            | 10.9                                            |                                                 | 10.9                             | 10.9                                            |                    |                    |      | 23.5             | 21.9              |
| 96  | Mg <sub>2</sub> Mo <sub>3</sub> O <sub>11</sub> | ZnMoO <sub>4</sub>                             | La <sub>2</sub> MoO <sub>6</sub>                |                                                 | HfMo <sub>2</sub> O <sub>8</sub> |                                                 | MnMoO <sub>4</sub> |                    |      | BaF <sub>2</sub> | BaCo <sub>3</sub> |
|     | 13.3                                            | 10.6                                           | 13.3                                            |                                                 | 13.3                             | 13.3                                            | 13.3               |                    |      | 0.3              | 33.3              |
| 97  | Ca <sub>3</sub> MoO <sub>6</sub>                | ZnMo <sub>2</sub> O <sub>7</sub>               | Pr <sub>2</sub> Mo <sub>3</sub> O <sub>12</sub> |                                                 |                                  | Ta <sub>2</sub> Mo <sub>3</sub> O <sub>14</sub> | MnMoO <sub>4</sub> |                    |      | BaF <sub>2</sub> | MgCo <sub>3</sub> |
|     | 9.0                                             | 9.0                                            | 9.0                                             |                                                 |                                  | 9.0                                             | 9.0                |                    |      | 9.2              | 0.5               |
| 98  | Sr <sub>3</sub> MoO <sub>6</sub>                | Zn <sub>3</sub> Mo <sub>2</sub> O <sub>9</sub> |                                                 | Al <sub>2</sub> Mo <sub>3</sub> O <sub>12</sub> | ZrMo <sub>2</sub> O <sub>8</sub> | Nb <sub>2</sub> Mo <sub>3</sub> O <sub>14</sub> |                    |                    |      | BaF <sub>2</sub> | MgCo <sub>3</sub> |
|     | 7.7                                             | 7.7                                            |                                                 | 15.4                                            | 7.7                              | 7.7                                             |                    |                    |      | 15.4             | 7.6               |
| 99  | Ba <sub>3</sub> MoO <sub>4</sub>                | ZnMoO <sub>4</sub>                             |                                                 | Al <sub>2</sub> Mo <sub>3</sub> O <sub>12</sub> | HfMo <sub>2</sub> O <sub>8</sub> |                                                 | MnMoO <sub>4</sub> |                    |      | BaF <sub>2</sub> | MgCo <sub>3</sub> |
|     | 6.7                                             | 13.3                                           |                                                 | 13.3                                            | 6.7                              |                                                 | 6.7                |                    |      | 20.0             | 13.3              |
| 100 | MgMoO <sub>4</sub>                              | ZnMo <sub>2</sub> O <sub>7</sub>               |                                                 | Al <sub>2</sub> Mo <sub>3</sub> O <sub>12</sub> |                                  | Ta <sub>2</sub> Mo <sub>3</sub> O <sub>14</sub> | MnMoO <sub>4</sub> |                    |      | BaF <sub>2</sub> | MgCo <sub>3</sub> |
|     | 5.8                                             | 11.6                                           |                                                 | 11.6                                            |                                  | 11.6                                            | 5.8                |                    |      | 24.8             | 17.2              |
| 101 | CaMoO <sub>4</sub>                              | Zn <sub>3</sub> Mo <sub>2</sub> O <sub>9</sub> |                                                 |                                                 | ZrMo <sub>2</sub> O <sub>8</sub> | Nb <sub>2</sub> Mo <sub>3</sub> O <sub>14</sub> | MnMoO <sub>4</sub> |                    |      | MgF <sub>2</sub> | MgCo <sub>3</sub> |
|     | 14.2                                            | 14.2                                           |                                                 |                                                 | 14.2                             | 14.2                                            | 7.1                |                    |      | 0.4              | 28.6              |
| 102 | SrMoO <sub>4</sub>                              |                                                | Ce <sub>6</sub> MoO <sub>12</sub>               | Al <sub>2</sub> Mo <sub>3</sub> O <sub>12</sub> | HfMo <sub>2</sub> O <sub>8</sub> | Ta <sub>2</sub> Mo <sub>3</sub> O <sub>14</sub> |                    |                    |      | MgF <sub>2</sub> | MgCo <sub>3</sub> |
|     | 12.5                                            |                                                | 12.5                                            | 12.5                                            | 12.5                             | 12.5                                            | 10.0               |                    |      | 6.2              | 31.3              |
| 103 | BaMoO <sub>4</sub>                              |                                                | Pr <sub>2</sub> MoO <sub>6</sub>                | Al <sub>2</sub> Mo <sub>3</sub> O <sub>12</sub> | ZrMo <sub>2</sub> O <sub>8</sub> |                                                 | MnMoO <sub>4</sub> |                    |      | MgF <sub>2</sub> | CaCo <sub>3</sub> |
|     | 8.3                                             |                                                | 8.3                                             | 8.3                                             | 8.3                              | 8.3                                             |                    |                    |      | 16.6             | 0.4               |
| 104 | Mg <sub>2</sub> Mo <sub>3</sub> O <sub>11</sub> |                                                | Nd <sub>2</sub> Mo <sub>3</sub> O <sub>12</sub> | Al <sub>2</sub> Mo <sub>3</sub> O <sub>12</sub> |                                  | Nb <sub>2</sub> Mo <sub>3</sub> O <sub>14</sub> | MnMoO <sub>4</sub> |                    |      | MgF <sub>2</sub> | CaCo <sub>3</sub> |
|     | 7.1                                             |                                                | 7.1                                             | 7.1                                             |                                  | 7.1                                             | 7.1                |                    |      | 21.5             | 7.7               |
| 105 | Ca <sub>3</sub> MoO <sub>6</sub>                |                                                | Sm <sub>2</sub> Mo <sub>2</sub> O <sub>7</sub>  |                                                 | HfMo <sub>2</sub> O <sub>8</sub> | Ta <sub>2</sub> Mo <sub>3</sub> O <sub>14</sub> | MnMoO <sub>4</sub> |                    |      | MgF <sub>2</sub> | CaCo <sub>3</sub> |
|     | 6.1                                             |                                                | 6.1                                             |                                                 | 6.1                              | 6.1                                             | 12.3               |                    |      | 26.4             | 12.3              |
| 106 | Sr <sub>3</sub> MoO <sub>6</sub>                |                                                |                                                 | Al <sub>2</sub> Mo <sub>3</sub> O <sub>12</sub> | ZrMo <sub>2</sub> O <sub>8</sub> | Nb <sub>2</sub> Mo <sub>3</sub> O <sub>14</sub> | MnMoO <sub>4</sub> |                    |      | CaF <sub>2</sub> | CaCo <sub>3</sub> |
|     | 7.7                                             |                                                |                                                 | 15.3                                            | 15.3                             | 15.3                                            | 7.7                |                    |      | 0.4              | 23.0              |
| 107 | ZnMoO <sub>4</sub>                              |                                                | Eu <sub>6</sub> MoO <sub>12</sub>               | Al <sub>2</sub> Mo <sub>3</sub> O <sub>12</sub> | HfMo <sub>2</sub> O <sub>8</sub> | Ta <sub>2</sub> Mo <sub>3</sub> O <sub>14</sub> |                    |                    |      | CaF <sub>2</sub> | CaCo <sub>3</sub> |
|     | 6.7                                             |                                                | 13.3                                            | 13.3                                            | 13.3                             | 13.3                                            | 13.3               |                    |      | 6.7              | 26.7              |
| 108 | ZnMo <sub>2</sub> O <sub>7</sub>                |                                                | Gd <sub>2</sub> MoO <sub>6</sub>                | Al <sub>2</sub> Mo <sub>3</sub> O <sub>12</sub> | ZrMo <sub>2</sub> O <sub>8</sub> |                                                 | MnMoO <sub>4</sub> |                    |      | CaF <sub>2</sub> | CaCo <sub>3</sub> |
|     | 9.4                                             |                                                | 11.8                                            | 11.8                                            | 11.8                             | 11.8                                            |                    |                    |      | 11.7             | 29.4              |
| 109 | Zn <sub>3</sub> Mo <sub>2</sub> O <sub>9</sub>  |                                                | Tb <sub>2</sub> Mo <sub>3</sub> O <sub>12</sub> | Al <sub>2</sub> Mo <sub>3</sub> O <sub>12</sub> |                                  | Nb <sub>2</sub> Mo <sub>3</sub> O <sub>14</sub> | MnMoO <sub>4</sub> |                    |      | CaF <sub>2</sub> | SrCo <sub>3</sub> |
|     | 7.7                                             |                                                | 7.7                                             | 7.7                                             |                                  | 7.7                                             |                    |                    |      | 22.9             | 0.3               |
| 110 | ZnMoO <sub>4</sub>                              |                                                | Dy <sub>6</sub> MoO <sub>12</sub>               |                                                 | HfMo <sub>2</sub> O <sub>8</sub> | Ta <sub>2</sub> Mo <sub>3</sub> O <sub>14</sub> | MnMoO <sub>4</sub> |                    |      | CaF <sub>2</sub> | SrCo <sub>3</sub> |
|     | 6.5                                             |                                                | 13.1                                            |                                                 | 6.5                              | 6.5                                             | 6.5                |                    |      | 28.1             | 6.6               |
| 111 | ZnMo <sub>2</sub> O <sub>7</sub>                |                                                |                                                 | Al <sub>2</sub> Mo <sub>3</sub> O <sub>12</sub> | ZrMo <sub>2</sub> O <sub>8</sub> | Nb <sub>2</sub> Mo <sub>3</sub> O <sub>14</sub> | MnMoO <sub>4</sub> |                    |      | SrF <sub>2</sub> | SrCo <sub>3</sub> |
|     | 16.6                                            |                                                |                                                 | 16.6                                            | 8.3                              | 8.3                                             | 8.3                |                    |      | 0.4              | 16.6              |
| 112 |                                                 |                                                | Ho <sub>6</sub> MoO <sub>12</sub>               | Al <sub>2</sub> Mo <sub>3</sub> O <sub>12</sub> | HfMo <sub>2</sub> O <sub>8</sub> | Ta <sub>2</sub> Mo <sub>3</sub> O <sub>14</sub> | MnMoO <sub>4</sub> |                    |      | SrF <sub>2</sub> | SrCo <sub>3</sub> |
|     |                                                 |                                                | 14.3                                            | 14.3                                            | 14.3                             | 7.1                                             | 7.1                |                    |      | 7.1              | 21.5              |
| 113 | MgMoO <sub>4</sub>                              | Zn <sub>3</sub> Mo <sub>2</sub> O <sub>9</sub> | Er <sub>2</sub> MoO <sub>6</sub>                | Al <sub>2</sub> Mo <sub>3</sub> O <sub>12</sub> | ZrMo <sub>2</sub> O <sub>8</sub> | Nb <sub>2</sub> Mo <sub>3</sub> O <sub>14</sub> |                    |                    |      | SrF <sub>2</sub> | SrCo <sub>3</sub> |
|     | 6.3                                             | 12.5                                           | 12.5                                            | 12.5                                            | 6.3                              | 6.3                                             |                    |                    |      | 12.4             | 24.9              |
| 114 | CaMoO <sub>4</sub>                              | ZnMoO <sub>4</sub>                             | Tm <sub>2</sub> MoO <sub>6</sub>                | Al <sub>2</sub> Mo <sub>3</sub> O <sub>12</sub> | HfMo <sub>2</sub> O <sub>8</sub> |                                                 | MnMoO <sub>4</sub> |                    |      | SrF <sub>2</sub> | SrCo <sub>3</sub> |
|     | 5.6                                             | 11.1                                           | 11.1                                            | 20                                              | 8.9                              |                                                 | 9.6                |                    |      | 16.7             | 27.7              |
| 115 | SrMoO <sub>4</sub>                              | ZnMo <sub>2</sub> O <sub>7</sub>               | Yb <sub>6</sub> MoO <sub>12</sub>               | Al <sub>2</sub> Mo <sub>3</sub> O <sub>12</sub> |                                  | Ta <sub>2</sub> Mo <sub>3</sub> O <sub>14</sub> | MnMoO <sub>4</sub> |                    |      | SrF <sub>2</sub> | BaCo <sub>3</sub> |
|     | 3.5                                             | 3.5                                            | 7.0                                             | 7.0                                             |                                  | 7.0                                             |                    |                    |      | 29.9             | 0.3               |
| 116 | BaMoO <sub>4</sub>                              | Zn <sub>3</sub> Mo <sub>2</sub> O <sub>9</sub> | Lu <sub>6</sub> MoO <sub>12</sub>               |                                                 | ZrMo <sub>2</sub> O <sub>8</sub> | Nb <sub>2</sub> Mo <sub>3</sub> O <sub>14</sub> | MnMoO <sub>4</sub> |                    |      | BaF <sub>2</sub> | BaCo <sub>3</sub> |
|     | 9.0                                             | 9.0                                            | 9.0                                             |                                                 | 9.0                              | 9.0                                             | 9.0                |                    |      | 0.5              | 9.2               |
| 117 | Mg <sub>2</sub> Mo <sub>3</sub> O <sub>11</sub> | ZnMoO <sub>4</sub>                             |                                                 | Al <sub>2</sub> Mo <sub>3</sub> O <sub>12</sub> | HfMo <sub>2</sub> O <sub>8</sub> | Ta <sub>2</sub> Mo <sub>3</sub> O <sub>14</sub> | MnMoO <sub>4</sub> |                    |      | BaF <sub>2</sub> | BaCo <sub>3</sub> |
|     | 15.4                                            | 7.7                                            |                                                 | 7.7                                             | 7.7                              | 7.7                                             | 7.7                |                    |      | 7.7              | 15.3              |
| 118 | Ca <sub>3</sub> MoO <sub>6</sub>                |                                                | Y <sub>2</sub> Mo <sub>3</sub> O <sub>12</sub>  | Al <sub>2</sub> Mo <sub>3</sub> O <sub>12</sub> | ZrMo <sub>2</sub> O <sub>8</sub> | Nb <sub>2</sub> Mo <sub>3</sub> O <sub>14</sub> | MnMoO <sub>4</sub> |                    |      | BaF <sub>2</sub> | BaCo <sub>3</sub> |
|     | 13.3                                            |                                                | 13.3                                            | 6.7                                             | 6.7                              | 6.7                                             | 6.7                |                    |      | 13.3             | 20.0              |
| 119 | ZnMo <sub>2</sub> O <sub>7</sub>                |                                                | La <sub>2</sub> MoO <sub>6</sub>                | Al <sub>2</sub> Mo <sub>3</sub> O <sub>12</sub> | HfMo <sub>2</sub> O <sub>8</sub> | Ta <sub>2</sub> Mo <sub>3</sub> O <sub>14</sub> | MnMoO <sub>4</sub> |                    |      | BaF <sub>2</sub> | BaCo <sub>3</sub> |
|     |                                                 |                                                | 11.8                                            | 11.8                                            | 11.8                             | 5.9                                             | 5.9                |                    |      | 17.6             | 23.5              |
| 120 | Sr <sub>3</sub> MoO <sub>6</sub>                | Zn <sub>3</sub> Mo <sub>2</sub> O <sub>9</sub> | CeMo <sub>2</sub> O <sub>8</sub>                | Al <sub>2</sub> Mo <sub>3</sub> O <sub>12</sub> | ZrMo <sub>2</sub> O <sub>8</sub> | Nb <sub>2</sub> Mo <sub>3</sub> O <sub>14</sub> | MnMoO <sub>4</sub> | 8.3                | 2.1  | BaF <sub>2</sub> | BaCo <sub>3</sub> |
|     | 5.2                                             | 5.2                                            | 5.2                                             | 9.2                                             | 10.3                             | 10.3                                            |                    |                    |      | 22.3             | 25.9              |

It is understood that Tables 2 to 8 correspond to the groups (A) to (G), and Table 9 indicates the proportions of the components selected from two or more groups.

The respective samples of the aforesaid components were heat-treated at 1000° C. for 1 hour in a gaseous atmosphere consisting of 98.5% by volume of nitrogen (N<sub>2</sub>) and 1.5% by volume of hydrogen (H<sub>2</sub>), and were thereafter pulverized together with ethanol in a pot mill and dried to obtain the heat-treated resistor material powders having a particle size of 10 µm and composed of the glass, the molybdates of the corresponding elements and the fluorides of alkaline earth metals.

The respective samples were then mixed with the carbonates of alkaline earth metals in the proportions specified in the tables. After mixing, 25 parts by weight of the organic vehicle (90 parts by weight of butyl carbitol plus 10 parts by weight of ethyl cellulose) were added to and mixed with 100 parts by weight of the resulting powdery mixtures in a ball mill to obtain the respective resistor material pastes.

On the other hand, 8 parts by weight of polyvinyl burlaral, 8 parts by weight of diethyl phthalate, 0.5 parts by weight of oleic acid, 10 parts by weight of acetone, 20 parts by weight of isopropyl alcohol and 20 parts by weight of methyl ethyl ketone were added to and mixed with 100 parts by weight of ceramic material powders consisting of 40.0% by weight of Al<sub>2</sub>O<sub>3</sub>, 35.0% by weight of SiO<sub>2</sub>, 13.0% by weight of B<sub>2</sub>O<sub>3</sub>, 7.0% by weight of CaO and 5.0% by weight of MgO by means of a ball mill to prepare a slurry, which was defoamed. Thereafter, the slurry was formed by the doctor blade process into a long ceramic green sheet of 200 µm in thickness. Cut out of this ceramic green sheet were a green sheet piece of 9 mm × 9 mm and a green sheet piece of 6 mm × 9 mm.

As shown in FIG. 1, printed on the aforesaid green sheet 1 piece 1 of 9 mm × 9 mm was a conductive material paste by means of screen printing, which was obtained by adding as the organic vehicle 20 parts by weight of butyl carbitol and 5 parts by weight of ethyl cellulose to 95 parts by weight of copper powders and 5 parts by weight of glass frit, followed by three-roll milling. The conductive paste printed ceramic green sheet piece 1 was dried at 125° C. for 10 minutes to form a conductive material film 2. Next, each of the aforesaid respective resistive material pastes was similarly screen-printed on the aforesaid green sheet piece 1 by the screen process, and was dried at 125° C. for 10 minutes to form a resistor material film 3 for a thick-film resistor.

Then, the aforesaid green sheet piece 4 of 6 mm × 9 mm was laminated upon the green sheet piece 1, as shown by a chain dash, at 100° C. and 150 Kg/cm<sup>2</sup>. Subsequently, the laminated product was heated at 400° to 500° C. in an oxidizing atmosphere of, e.g., air to decompose and burn off the organics remaining in the green sheet pieces 1, 4, the conductive film 2 and the resistive film 3.

After decomposing the organics in this manner, they were fired at 950° C. for 1 hour in a gaseous mixture consisting of 98.5% by volume of N<sub>2</sub> and 1.5% by vol-

ume of H<sub>2</sub> to obtain an integral multilayered ceramic board having a porcelain 1a formed of the sintered body of the green sheet piece 1, a porcelain layer 4a formed of the sintered body of the green sheet piece 4, a thick-film conductor 2a formed of the sintered body of the conductive film 2 and a thick-film resistor 3a formed of the sintered resistive film 3 located between the layers 1 and 4, as illustrated in FIG. 3. With regard to this multilayered ceramic board, such warping or swelling as shown in FIGS. 4 and 5 were not found, as will be described later.

The thus obtained multilayered ceramic board was polished in its layer direction to expose the resistor layer to view, which was then analyzed by X-ray diffraction (Cu K alpha rays). The results of Sample No. 1 obtained are shown in FIG. 6, from which the presence of the molybdate of the corresponding element could be ascertained. FIG. 7 is also a TEM photograph taken of said sample, which shows the acicular particles that are the reduction product of the molybdate of magnesium. In the photograph, the molybdate of magnesium is shown by a black portion on the left side, and the glass is indicated by a gray portion on the upper side. It is to be noted that the sample, of which a TEM photograph was taken, was prepared by cutting the multilayered ceramic board in the sectional direction to a band of 200 µm in width, and polishing the band to a thickness of about 20 µm, followed by thinning with an ion milling device. Although not illustrated and described, similar results could also be confirmed with respect to other samples.

Next, the resistance values (R<sub>25</sub>) and (R<sub>125</sub>) of the thick-film resistor 3a at 25° C. and at the time when heated to 125° C. were measured with a digital multimeter, and the temperature coefficient of resistance (TCR) was calculated from the following equation:

$$TCR = \frac{R_{125} - R_{25}}{R_{25}} \times 10000 \text{ (ppm/°C.)}$$

The measured resistance values R<sub>25</sub> and calculated values TCR are shown in Table 10 for the compositions of Table 2 and, similarly, in Tables 11 to 17 for the compositions of Tables 3 to 9.

After the obtained multilayered ceramic board had been permitted to stand at 60° C. and a relative humidity of 95% for 1000 hours, its resistance at 25° C. was measured to determine the rate of change with respect to the resistance at 25° C. Just as mentioned above, the results are shown in the tables.

With resistor material samples obtained by removing the carbonates and fluorides of alkaline earth metals, and by removing the former only from the aforesaid respective resistor material samples, multilayered ceramic boards were prepared and measured in the same manner as mentioned above. The results are set forth in Tables 10 to 17 with the sample numbers corresponding to the sample numbers of the 1st column in the 2nd and 3rd columns of Tables 10 to 17.

TABLE 10

| Nos | (Characteristic values corresponding to the sample in Table 2) |               |                                  |                                                |               |                                  |                                                |               |                                  |
|-----|----------------------------------------------------------------|---------------|----------------------------------|------------------------------------------------|---------------|----------------------------------|------------------------------------------------|---------------|----------------------------------|
|     | Example 1                                                      |               | Carbonate-Free                   |                                                |               | Carbonate & Fluoride-Free        |                                                |               |                                  |
|     | Resistance value at 25° C. R <sub>25</sub> (Ω)                 | TCR (ppm/°C.) | Rate of Change in Resistance (%) | Resistance value at 25° C. R <sub>25</sub> (Ω) | TCR (ppm/°C.) | Rate of Change in Resistance (%) | Resistance value at 25° C. R <sub>25</sub> (Ω) | TCR (ppm/°C.) | Rate of Change in Resistance (%) |
| 1   | 8.35 × 10 <sup>3</sup>                                         | -286          | <±2                              | 22.6 × 10 <sup>3</sup>                         | -511          | <±2                              | 18.5 × 10 <sup>3</sup>                         | -831          | <±2                              |

TABLE 10-continued

(Characteristic values corresponding to the sample in Table 2)

| Nos | Example 1                                      |               | Carbonate-Free                   |                                                |               |                                  | Carbonate & Fluoride-Free                      |               |                                  |
|-----|------------------------------------------------|---------------|----------------------------------|------------------------------------------------|---------------|----------------------------------|------------------------------------------------|---------------|----------------------------------|
|     | Resistance value at 25° C. R <sub>25</sub> (Ω) | TCR (ppm/°C.) | Rate of Change in Resistance (%) | Resistance value at 25° C. R <sub>25</sub> (Ω) | TCR (ppm/°C.) | Rate of Change in Resistance (%) | Resistance value at 25° C. R <sub>25</sub> (Ω) | TCR (ppm/°C.) | Rate of Change in Resistance (%) |
| 2   | 5.28 × 10 <sup>3</sup>                         | -252          | "                                | 14.9 × 10 <sup>3</sup>                         | -496          | "                                | 9.24 × 10 <sup>3</sup>                         | -529          | "                                |
| 3   | 2.15 × 10 <sup>3</sup>                         | -192          | "                                | 72.3 × 10 <sup>3</sup>                         | -424          | "                                | 4.11 × 10 <sup>3</sup>                         | -508          | "                                |
| 4   | 1.02 × 10 <sup>3</sup>                         | -161          | "                                | 4.55 × 10 <sup>3</sup>                         | -326          | "                                | 2.36 × 10 <sup>3</sup>                         | -456          | "                                |
| 5   | 6.49 × 10 <sup>3</sup>                         | -274          | "                                | 13.8 × 10 <sup>3</sup>                         | -405          | "                                | 9.21 × 10 <sup>3</sup>                         | -530          | "                                |
| 6   | 1.58 × 10 <sup>3</sup>                         | -173          | "                                | 6.98 × 10 <sup>3</sup>                         | -369          | "                                | 4.07 × 10 <sup>3</sup>                         | -511          | "                                |
| 7   | 3.58 × 10 <sup>3</sup>                         | -248          | "                                | 10.2 × 10 <sup>3</sup>                         | -502          | "                                | 12.6 × 10 <sup>3</sup>                         | -542          | "                                |
| 8   | 2.73 × 10 <sup>3</sup>                         | -205          | "                                | 8.24 × 10 <sup>3</sup>                         | -498          | "                                | 2.03 × 10 <sup>3</sup>                         | -501          | "                                |
| 9   | 1.03 × 10 <sup>3</sup>                         | -168          | "                                | 7.44 × 10 <sup>3</sup>                         | -472          | "                                | 1.99 × 10 <sup>3</sup>                         | -499          | "                                |
| 10  | 1.18 × 10 <sup>3</sup>                         | -177          | "                                | 8.34 × 10 <sup>3</sup>                         | -499          | "                                | 4.07 × 10 <sup>3</sup>                         | -511          | "                                |
| 11  | 899                                            | -89           | "                                | 5.21 × 10 <sup>3</sup>                         | -470          | "                                | 2.03 × 10 <sup>3</sup>                         | -501          | "                                |
| 12  | 925                                            | -97           | "                                | 4.49 × 10 <sup>3</sup>                         | -462          | "                                | 1.97 × 10 <sup>3</sup>                         | -498          | "                                |
| 13  | 676                                            | -25           | "                                | 3.32 × 10 <sup>3</sup>                         | -454          | "                                | 3.12 × 10 <sup>3</sup>                         | -505          | "                                |
| 14  | 4.03 × 10 <sup>3</sup>                         | -270          | "                                | 11.5 × 10 <sup>3</sup>                         | -504          | "                                | 12.6 × 10 <sup>3</sup>                         | -542          | "                                |
| 15  | 2.88 × 10 <sup>3</sup>                         | -211          | "                                | 8.27 × 10 <sup>3</sup>                         | -498          | "                                | 2.03 × 10 <sup>3</sup>                         | -501          | "                                |
| 16  | 2.91 × 10 <sup>3</sup>                         | -218          | "                                | 7.98 × 10 <sup>3</sup>                         | -483          | "                                | 1.99 × 10 <sup>3</sup>                         | -499          | "                                |
| 17  | 3.10 × 10 <sup>3</sup>                         | -229          | "                                | 8.20 × 10 <sup>3</sup>                         | -497          | "                                | 4.07 × 10 <sup>3</sup>                         | -511          | "                                |
| 18  | 1.03 × 10 <sup>3</sup>                         | -159          | "                                | 7.52 × 10 <sup>3</sup>                         | -474          | "                                | 2.03 × 10 <sup>3</sup>                         | -501          | "                                |
| 19  | 1.57 × 10 <sup>3</sup>                         | -198          | "                                | 8.01 × 10 <sup>3</sup>                         | -487          | "                                | 1.97 × 10 <sup>3</sup>                         | -498          | "                                |
| 20  | 755                                            | -71           | "                                | 8.13 × 10 <sup>3</sup>                         | -492          | "                                | 3.12 × 10 <sup>3</sup>                         | -505          | "                                |
| 21  | 980                                            | -135          | "                                | 8.28 × 10 <sup>3</sup>                         | -498          | "                                | 4.07 × 10 <sup>3</sup>                         | -511          | "                                |
| 22  | 805                                            | -75           | "                                | 7.73 × 10 <sup>3</sup>                         | -482          | "                                | 1.97 × 10 <sup>3</sup>                         | -498          | "                                |
| 23  | 953                                            | -109          | "                                | 7.99 × 10 <sup>3</sup>                         | -494          | "                                | 4.07 × 10 <sup>3</sup>                         | -511          | "                                |
| 24  | 785                                            | -70           | "                                | 7.66 × 10 <sup>3</sup>                         | -475          | "                                | 1.97 × 10 <sup>3</sup>                         | -498          | "                                |
| 25  | 1.09 × 10 <sup>3</sup>                         | -171          | "                                | 11.9 × 10 <sup>3</sup>                         | -510          | "                                | 4.07 × 10 <sup>3</sup>                         | -511          | "                                |
| 26  | 867                                            | -81           | "                                | 7.92 × 10 <sup>3</sup>                         | -482          | "                                | 1.97 × 10 <sup>3</sup>                         | -498          | "                                |
| 27  | 4.73 × 10 <sup>3</sup>                         | -281          | "                                | 8.10 × 10 <sup>3</sup>                         | -491          | "                                | 2.42 × 10 <sup>3</sup>                         | -503          | "                                |
| 28  | 1.13 × 10 <sup>3</sup>                         | -125          | "                                | 7.50 × 10 <sup>3</sup>                         | -472          | "                                | 2.03 × 10 <sup>3</sup>                         | -501          | "                                |
| 29  | 3.00 × 10 <sup>3</sup>                         | -229          | "                                | 8.06 × 10 <sup>3</sup>                         | -488          | "                                | 2.42 × 10 <sup>3</sup>                         | -503          | "                                |
| 30  | 854                                            | -77           | "                                | 7.14 × 10 <sup>3</sup>                         | -452          | "                                | 2.03 × 10 <sup>3</sup>                         | -501          | "                                |
| 31  | 3.95 × 10 <sup>3</sup>                         | -248          | "                                | 8.09 × 10 <sup>3</sup>                         | -489          | "                                | 2.42 × 10 <sup>3</sup>                         | -503          | "                                |
| 32  | 953                                            | -98           | "                                | 7.21 × 10 <sup>3</sup>                         | -463          | "                                | 2.03 × 10 <sup>3</sup>                         | -501          | "                                |
| 33  | 3.02 × 10 <sup>3</sup>                         | -221          | "                                | 7.75 × 10 <sup>3</sup>                         | -484          | "                                | 2.03 × 10 <sup>3</sup>                         | -507          | "                                |
| 34  | 3.77 × 10 <sup>3</sup>                         | -248          | "                                | 8.15 × 10 <sup>3</sup>                         | -492          | "                                | 4.07 × 10 <sup>3</sup>                         | -511          | "                                |
| 35  | 9.34 × 10 <sup>3</sup>                         | 233           | "                                | 14.6 × 10 <sup>3</sup>                         | 502           | "                                | 12.9 × 10 <sup>3</sup>                         | -744          | "                                |
| 36  | 5.68 × 10 <sup>3</sup>                         | 164           | "                                | 9.28 × 10 <sup>3</sup>                         | 321           | "                                | 7.11 × 10 <sup>3</sup>                         | -516          | "                                |
| 37  | 1.04 × 10 <sup>3</sup>                         | 98            | "                                | 4.67 × 10 <sup>3</sup>                         | 216           | "                                | 2.07 × 10 <sup>3</sup>                         | -440          | "                                |
| 38  | 923                                            | 87            | "                                | 3.34 × 10 <sup>3</sup>                         | 173           | "                                | 1.09 × 10 <sup>3</sup>                         | -395          | "                                |
| 39  | 3.24 × 10 <sup>3</sup>                         | 121           | "                                | 8.89 × 10 <sup>3</sup>                         | 288           | "                                | 7.14 × 10 <sup>3</sup>                         | -512          | "                                |
| 40  | 1.89 × 10 <sup>3</sup>                         | 113           | "                                | 5.11 × 10 <sup>3</sup>                         | 244           | "                                | 2.06 × 10 <sup>3</sup>                         | -438          | "                                |
| 41  | 2.05 × 10 <sup>3</sup>                         | -153          | "                                | 5.14 × 10 <sup>3</sup>                         | -478          | "                                | 5.23 × 10 <sup>3</sup>                         | -482          | "                                |
| 42  | 1.03 × 10 <sup>3</sup>                         | -108          | "                                | 2.05 × 10 <sup>3</sup>                         | -418          | "                                | 1.52 × 10 <sup>3</sup>                         | -421          | "                                |
| 43  | 847                                            | -83           | "                                | 1.23 × 10 <sup>3</sup>                         | -384          | "                                | 1.14 × 10 <sup>3</sup>                         | -397          | "                                |
| 44  | 980                                            | -89           | "                                | 1.62 × 10 <sup>3</sup>                         | -392          | "                                | 2.07 × 10 <sup>3</sup>                         | -440          | "                                |
| 45  | 658                                            | -41           | "                                | 1.54 × 10 <sup>3</sup>                         | -388          | "                                | 1.48 × 10 <sup>3</sup>                         | -420          | "                                |
| 46  | 723                                            | -37           | "                                | 1.47 × 10 <sup>3</sup>                         | -384          | "                                | 1.21 × 10 <sup>3</sup>                         | -399          | "                                |
| 47  | 521                                            | -5            | "                                | 1.14 × 10 <sup>3</sup>                         | -381          | "                                | 1.10 × 10 <sup>3</sup>                         | -395          | "                                |
| 48  | 1.23 × 10 <sup>3</sup>                         | -98           | "                                | 2.09 × 10 <sup>3</sup>                         | -436          | "                                | 2.07 × 10 <sup>3</sup>                         | -440          | "                                |
| 49  | 705                                            | -59           | "                                | 1.32 × 10 <sup>3</sup>                         | -383          | "                                | 1.21 × 10 <sup>3</sup>                         | -399          | "                                |
| 50  | 915                                            | -78           | "                                | 2.10 × 10 <sup>3</sup>                         | -434          | "                                | 2.07 × 10 <sup>3</sup>                         | -440          | "                                |
| 51  | 625                                            | -38           | "                                | 1.25 × 10 <sup>3</sup>                         | -382          | "                                | 1.21 × 10 <sup>3</sup>                         | -399          | "                                |
| 52  | 1.01 × 10 <sup>3</sup>                         | -95           | "                                | 2.13 × 10 <sup>3</sup>                         | -438          | "                                | 2.07 × 10 <sup>3</sup>                         | -440          | "                                |
| 53  | 688                                            | -50           | "                                | 1.82 × 10 <sup>3</sup>                         | -401          | "                                | 1.21 × 10 <sup>3</sup>                         | -399          | "                                |
| 54  | 3.77 × 10 <sup>3</sup>                         | -230          | "                                | 4.05 × 10 <sup>3</sup>                         | -444          | "                                | 1.54 × 10 <sup>3</sup>                         | -422          | "                                |
| 55  | 991                                            | -100          | "                                | 2.03 × 10 <sup>3</sup>                         | -417          | "                                | 1.48 × 10 <sup>3</sup>                         | -420          | "                                |
| 56  | 2.01 × 10 <sup>3</sup>                         | -131          | "                                | 3.49 × 10 <sup>3</sup>                         | -421          | "                                | 1.54 × 10 <sup>3</sup>                         | -422          | "                                |
| 57  | 795                                            | -50           | "                                | 2.09 × 10 <sup>3</sup>                         | -418          | "                                | 1.48 × 10 <sup>3</sup>                         | -420          | "                                |
| 58  | 2.95 × 10 <sup>3</sup>                         | -185          | "                                | 3.63 × 10 <sup>3</sup>                         | -423          | "                                | 1.54 × 10 <sup>3</sup>                         | -422          | "                                |
| 59  | 888                                            | -55           | "                                | 2.02 × 10 <sup>3</sup>                         | -417          | "                                | 1.48 × 10 <sup>3</sup>                         | -420          | "                                |
| 60  | 1.45 × 10 <sup>3</sup>                         | -129          | "                                | 3.51 × 10 <sup>3</sup>                         | -421          | "                                | 1.48 × 10 <sup>3</sup>                         | -420          | "                                |
| 61  | 1.01 × 10 <sup>3</sup>                         | -120          | "                                | 4.25 × 10 <sup>3</sup>                         | -445          | "                                | 2.07 × 10 <sup>3</sup>                         | -440          | "                                |
| 62  | 1.63 × 10 <sup>3</sup>                         | -136          | "                                | 4.50 × 10 <sup>3</sup>                         | 369           | "                                | 2.22 × 10 <sup>3</sup>                         | -451          | "                                |
| 63  | 2.49 × 10 <sup>3</sup>                         | -203          | "                                | 4.82 × 10 <sup>3</sup>                         | -458          | "                                | 4.08 × 10 <sup>3</sup>                         | -462          | "                                |
| 64  | 30.2 × 10 <sup>3</sup>                         | +32           | "                                | 70.5 × 10 <sup>3</sup>                         | -321          | "                                | 97.5 × 10 <sup>3</sup>                         | -829          | "                                |
| 65  | 27.9 × 10 <sup>3</sup>                         | +49           | "                                | 59.7 × 10 <sup>3</sup>                         | -286          | "                                | 25.6 × 10 <sup>3</sup>                         | -519          | "                                |
| 66  | 18.4 × 10 <sup>3</sup>                         | +116          | "                                | 36.5 × 10 <sup>3</sup>                         | -224          | "                                | 12.3 × 10 <sup>3</sup>                         | -268          | "                                |
| 67  | 2.54 × 10 <sup>3</sup>                         | +223          | "                                | 4.39 × 10 <sup>3</sup>                         | -63           | "                                | 1.86 × 10 <sup>3</sup>                         | -85           | "                                |
| 68  | 26.8 × 10 <sup>3</sup>                         | +52           | "                                | 49.3 × 10 <sup>3</sup>                         | -218          | "                                | 27.4 × 10 <sup>3</sup>                         | -436          | "                                |
| 69  | 22.4 × 10 <sup>3</sup>                         | +73           | "                                | 37.2 × 10 <sup>3</sup>                         | -163          | "                                | 12.4 × 10 <sup>3</sup>                         | -270          | "                                |
| 70  | 40.5 × 10 <sup>3</sup>                         | +52           | "                                | 62.7 × 10 <sup>3</sup>                         | -462          | "                                | 42.3 × 10 <sup>3</sup>                         | -639          | "                                |
| 71  | 32.5 × 10 <sup>3</sup>                         | +80           | "                                | 45.6 × 10 <sup>3</sup>                         | -233          | "                                | 8.26 × 10 <sup>3</sup>                         | -248          | "                                |
| 72  | 14.8 × 10 <sup>3</sup>                         | +125          | "                                | 32.8 × 10 <sup>3</sup>                         | -196          | "                                | 7.42 × 10 <sup>3</sup>                         | -236          | "                                |
| 73  | 17.3 × 10 <sup>3</sup>                         | +103          | "                                | 40.5 × 10 <sup>3</sup>                         | -214          | "                                | 12.4 × 10 <sup>3</sup>                         | -270          | "                                |
| 74  | 7.25 × 10 <sup>3</sup>                         | +178          | "                                | 47.6 × 10 <sup>3</sup>                         | -240          | "                                | 8.26 × 10 <sup>3</sup>                         | -248          | "                                |
| 75  | 9.00 × 10 <sup>3</sup>                         | +175          | "                                | 42.1 × 10 <sup>3</sup>                         | -221          | "                                | 6.98 × 10 <sup>3</sup>                         | -230          | "                                |
| 76  | 856                                            | +255          | "                                | 2.04 × 10 <sup>3</sup>                         | -99           | "                                | 2.23 × 10 <sup>3</sup>                         | -103          | "                                |

TABLE 10-continued

(Characteristic values corresponding to the sample in Table 2)

| Nos | Example 1                                      |               |                                  | Carbonate-Free                                 |               |                                  | Carbonate & Fluoride-Free                      |               |                                  |
|-----|------------------------------------------------|---------------|----------------------------------|------------------------------------------------|---------------|----------------------------------|------------------------------------------------|---------------|----------------------------------|
|     | Resistance value at 25° C. R <sub>25</sub> (Ω) | TCR (ppm/°C.) | Rate of Change in Resistance (%) | Resistance value at 25° C. R <sub>25</sub> (Ω) | TCR (ppm/°C.) | Rate of Change in Resistance (%) | Resistance value at 25° C. R <sub>25</sub> (Ω) | TCR (ppm/°C.) | Rate of Change in Resistance (%) |
| 77  | $43.1 \times 10^3$                             | +26           | "                                | $59.4 \times 10^3$                             | -398          | "                                | $42.3 \times 10^3$                             | -639          | "                                |
| 78  | $35.1 \times 10^3$                             | +62           | "                                | $41.8 \times 10^3$                             | -218          | "                                | $8.26 \times 10^3$                             | -248          | "                                |
| 79  | $19.4 \times 10^3$                             | +79           | "                                | $34.5 \times 10^3$                             | -199          | "                                | $7.42 \times 10^3$                             | -236          | "                                |
| 80  | $21.7 \times 10^3$                             | +88           | "                                | $43.2 \times 10^3$                             | -224          | "                                | $12.4 \times 10^3$                             | -270          | "                                |
| 81  | $9.85 \times 10^3$                             | +102          | "                                | $32.9 \times 10^3$                             | -198          | "                                | $8.26 \times 10^3$                             | -248          | "                                |
| 82  | $10.6 \times 10^3$                             | +105          | "                                | $30.5 \times 10^3$                             | -186          | "                                | $6.98 \times 10^3$                             | -230          | "                                |
| 83  | $1.03 \times 10^3$                             | +205          | "                                | $1.85 \times 10^3$                             | -87           | "                                | $2.23 \times 10^3$                             | -103          | "                                |
| 84  | $20.5 \times 10^3$                             | +95           | "                                | $44.6 \times 10^3$                             | -225          | "                                | $12.4 \times 10^3$                             | -270          | "                                |
| 85  | $12.3 \times 10^3$                             | +120          | "                                | $31.2 \times 10^3$                             | -196          | "                                | $6.98 \times 10^3$                             | -230          | "                                |
| 86  | $16.1 \times 10^3$                             | +111          | "                                | $38.7 \times 10^3$                             | -210          | "                                | $12.4 \times 10^3$                             | -270          | "                                |
| 87  | $6.99 \times 10^3$                             | +181          | "                                | $30.9 \times 10^3$                             | -187          | "                                | $6.98 \times 10^3$                             | -230          | "                                |
| 88  | $19.7 \times 10^3$                             | +98           | "                                | $50.2 \times 10^3$                             | -246          | "                                | $12.4 \times 10^3$                             | -270          | "                                |
| 89  | $10.8 \times 10^3$                             | +179          | "                                | $29.6 \times 10^3$                             | -185          | "                                | $6.98 \times 10^3$                             | -230          | "                                |
| 90  | $4.27 \times 10^3$                             | -55           | "                                | $51.3 \times 10^3$                             | -248          | "                                | $8.82 \times 10^3$                             | -252          | "                                |
| 91  | $10.3 \times 10^3$                             | +149          | "                                | $21.6 \times 10^3$                             | -152          | "                                | $8.26 \times 10^3$                             | -248          | "                                |
| 92  | $39.5 \times 10^3$                             | -60           | "                                | $54.9 \times 10^3$                             | -250          | "                                | $8.82 \times 10^3$                             | -252          | "                                |
| 93  | $8.08 \times 10^3$                             | +153          | "                                | $27.4 \times 10^3$                             | -172          | "                                | $8.26 \times 10^3$                             | -248          | "                                |
| 94  | $40.9 \times 10^3$                             | -39           | "                                | $48.6 \times 10^3$                             | -245          | "                                | $8.82 \times 10^3$                             | -252          | "                                |
| 95  | $8.91 \times 10^3$                             | +160          | "                                | $28.2 \times 10^3$                             | -180          | "                                | $8.26 \times 10^3$                             | -248          | "                                |
| 96  | $34.4 \times 10^3$                             | +71           | "                                | $42.5 \times 10^3$                             | -222          | "                                | $8.26 \times 10^3$                             | -248          | "                                |
| 97  | $20.9 \times 10^3$                             | +95           | "                                | $50.0 \times 10^3$                             | -246          | "                                | $12.4 \times 10^3$                             | -270          | "                                |
| 98  | $68.2 \times 10^3$                             | -234          | "                                | $97.6 \times 10^3$                             | -463          | "                                | $100.6 \times 10^3$                            | -957          | "                                |
| 99  | $27.3 \times 10^3$                             | -92           | "                                | $46.5 \times 10^3$                             | -413          | "                                | $32.4 \times 10^3$                             | -607          | "                                |
| 100 | $20.8 \times 10^3$                             | -74           | "                                | $34.8 \times 10^3$                             | -296          | "                                | $21.4 \times 10^3$                             | -483          | "                                |
| 101 | $6.24 \times 10^3$                             | -25           | "                                | $10.7 \times 10^3$                             | -152          | "                                | $5.37 \times 10^3$                             | -195          | "                                |
| 102 | $27.6 \times 10^3$                             | -96           | "                                | $35.2 \times 10^3$                             | -274          | "                                | $32.9 \times 10^3$                             | -436          | "                                |
| 103 | $18.8 \times 10^3$                             | -48           | "                                | $29.6 \times 10^3$                             | -304          | "                                | $21.1 \times 10^3$                             | -490          | "                                |
| 104 | $45.4 \times 10^3$                             | -127          | "                                | $63.2 \times 10^3$                             | -512          | "                                | $68.2 \times 10^3$                             | -802          | "                                |
| 105 | $36.6 \times 10^3$                             | -83           | "                                | $45.2 \times 10^3$                             | -262          | "                                | $12.5 \times 10^3$                             | -271          | "                                |
| 106 | $19.6 \times 10^3$                             | -18           | "                                | $30.4 \times 10^3$                             | -241          | "                                | $7.24 \times 10^3$                             | -243          | "                                |
| 107 | $22.1 \times 10^3$                             | -77           | "                                | $51.3 \times 10^3$                             | -462          | "                                | $21.4 \times 10^3$                             | -483          | "                                |
| 108 | $9.90 \times 10^3$                             | -55           | "                                | $30.3 \times 10^3$                             | -241          | "                                | $6.96 \times 10^3$                             | -338          | "                                |
| 109 | $12.3 \times 10^3$                             | -37           | "                                | $17.7 \times 10^3$                             | -200          | "                                | $6.12 \times 10^3$                             | -219          | "                                |
| 110 | $1.87 \times 10^3$                             | -60           | "                                | $32.8 \times 10^3$                             | -254          | "                                | $8.63 \times 10^3$                             | -262          | "                                |
| 111 | $20.8 \times 10^3$                             | -75           | "                                | $54.2 \times 10^3$                             | -472          | "                                | $21.1 \times 10^3$                             | -490          | "                                |
| 112 | $9.85 \times 10^3$                             | -28           | "                                | $45.3 \times 10^3$                             | -264          | "                                | $12.3 \times 10^3$                             | -270          | "                                |
| 113 | $18.6 \times 10^3$                             | -60           | "                                | $56.3 \times 10^3$                             | -481          | "                                | $21.1 \times 10^3$                             | -490          | "                                |
| 114 | $9.12 \times 10^3$                             | -29           | "                                | $17.4 \times 10^3$                             | -198          | "                                | $6.12 \times 10^3$                             | -219          | "                                |
| 115 | $21.2 \times 10^3$                             | -68           | "                                | $54.3 \times 10^3$                             | -472          | "                                | $21.4 \times 10^3$                             | -483          | "                                |
| 116 | $11.5 \times 10^3$                             | -35           | "                                | $18.6 \times 10^3$                             | -209          | "                                | $6.12 \times 10^3$                             | -219          | "                                |
| 117 | $43.6 \times 10^3$                             | -188          | "                                | $47.9 \times 10^3$                             | -306          | "                                | $14.6 \times 10^3$                             | -302          | "                                |
| 118 | $11.5 \times 10^3$                             | -58           | "                                | $28.9 \times 10^3$                             | -225          | "                                | $6.96 \times 10^3$                             | -233          | "                                |
| 119 | $38.5 \times 10^3$                             | -107          | "                                | $44.6 \times 10^3$                             | -292          | "                                | $14.6 \times 10^3$                             | -302          | "                                |
| 120 | $9.05 \times 10^3$                             | -51           | "                                | $29.3 \times 10^3$                             | -230          | "                                | $6.96 \times 10^3$                             | -233          | "                                |
| 121 | $34.5 \times 10^3$                             | -95           | "                                | $42.3 \times 10^3$                             | -290          | "                                | $14.6 \times 10^3$                             | -302          | "                                |
| 122 | $7.88 \times 10^3$                             | -50           | "                                | $29.5 \times 10^3$                             | -231          | "                                | $6.96 \times 10^3$                             | -233          | "                                |
| 123 | $38.3 \times 10^3$                             | -107          | "                                | $30.2 \times 10^3$                             | -236          | "                                | $6.96 \times 10^3$                             | -233          | "                                |
| 124 | $22.5 \times 10^3$                             | -89           | "                                | $55.4 \times 10^3$                             | -472          | "                                | $21.4 \times 10^3$                             | -483          | "                                |
| 125 | $4.73 \times 10^3$                             | -42           | "                                | $48.6 \times 10^3$                             | -321          | "                                | $3.62 \times 10^3$                             | -138          | "                                |
| 126 | $21.9 \times 10^3$                             | -55           | "                                | $48.6 \times 10^3$                             | -321          | "                                | $16.9 \times 10^3$                             | -324          | "                                |
| 127 | $2.22 \times 10^3$                             | -126          | "                                | $3.48 \times 10^3$                             | -324          | "                                | $2.36 \times 10^3$                             | -626          | "                                |
| 128 | $1.76 \times 10^3$                             | -83           | "                                | $2.32 \times 10^3$                             | -302          | "                                | $1.90 \times 10^3$                             | -490          | "                                |
| 129 | 893                                            | +64           | "                                | $1.26 \times 10^3$                             | -236          | "                                | 619                                            | -251          | "                                |
| 130 | 562                                            | +52           | "                                | 763                                            | -103          | "                                | 488                                            | +55           | "                                |
| 131 | $2.04 \times 10^3$                             | -109          | "                                | $2.88 \times 10^3$                             | -318          | "                                | $1.92 \times 10^3$                             | -505          | "                                |
| 132 | 724                                            | -63           | "                                | 846                                            | -193          | "                                | 621                                            | -250          | "                                |
| 133 | 841                                            | -216          | "                                | $1.25 \times 10^3$                             | -493          | "                                | $2.35 \times 10^3$                             | -732          | "                                |
| 134 | 803                                            | -185          | "                                | $1.09 \times 10^3$                             | -240          | "                                | 492                                            | -241          | "                                |
| 135 | 596                                            | -107          | "                                | 954                                            | -236          | "                                | 468                                            | -238          | "                                |
| 136 | 608                                            | -106          | "                                | $1.12 \times 10^3$                             | -248          | "                                | 621                                            | -250          | "                                |
| 137 | 442                                            | +56           | "                                | 974                                            | -238          | "                                | 492                                            | -241          | "                                |
| 138 | 438                                            | +58           | "                                | 968                                            | -237          | "                                | 474                                            | -239          | "                                |
| 139 | 396                                            | +95           | "                                | 942                                            | -232          | "                                | 442                                            | -235          | "                                |
| 140 | 839                                            | -238          | "                                | $1.22 \times 10^3$                             | -487          | "                                | $2.35 \times 10^3$                             | -732          | "                                |
| 141 | 798                                            | -198          | "                                | $1.10 \times 10^3$                             | -242          | "                                | 492                                            | -241          | "                                |
| 142 | 597                                            | -115          | "                                | 969                                            | -237          | "                                | 468                                            | -238          | "                                |
| 143 | 603                                            | -118          | "                                | $1.14 \times 10^3$                             | -248          | "                                | 621                                            | -250          | "                                |
| 144 | 438                                            | +5            | "                                | 975                                            | -238          | "                                | 492                                            | -241          | "                                |
| 145 | 441                                            | -15           | "                                | 965                                            | -237          | "                                | 474                                            | -239          | "                                |
| 146 | 390                                            | +21           | "                                | 948                                            | -233          | "                                | 442                                            | -235          | "                                |
| 147 | 705                                            | -159          | "                                | $1.16 \times 10^3$                             | -249          | "                                | 621                                            | -250          | "                                |
| 148 | 509                                            | -56           | "                                | 964                                            | -236          | "                                | 474                                            | -239          | "                                |
| 149 | 617                                            | -111          | "                                | $1.13 \times 10^3$                             | -248          | "                                | 621                                            | -250          | "                                |
| 150 | 459                                            | +41           | "                                | 968                                            | -237          | "                                | 474                                            | -239          | "                                |
| 151 | 668                                            | -140          | "                                | $1.18 \times 10^3$                             | -252          | "                                | 621                                            | -250          | "                                |

TABLE 10-continued

(Characteristic values corresponding to the sample in Table 2)

| Nos | Example 1                                      |               |                                  | Carbonate-Free                                 |               |                                  | Carbonate & Fluoride-Free                      |               |                                  |
|-----|------------------------------------------------|---------------|----------------------------------|------------------------------------------------|---------------|----------------------------------|------------------------------------------------|---------------|----------------------------------|
|     | Resistance value at 25° C. R <sub>25</sub> (Ω) | TCR (ppm/°C.) | Rate of Change in Resistance (%) | Resistance value at 25° C. R <sub>25</sub> (Ω) | TCR (ppm/°C.) | Rate of Change in Resistance (%) | Resistance value at 25° C. R <sub>25</sub> (Ω) | TCR (ppm/°C.) | Rate of Change in Resistance (%) |
| 152 | 481                                            | +36           | "                                | 970                                            | -237          | "                                | 474                                            | -239          | "                                |
| 153 | 636                                            | -119          | "                                | 973                                            | -237          | "                                | 470                                            | -238          | "                                |
| 154 | 481                                            | -5            | "                                | 976                                            | -238          | "                                | 492                                            | -241          | "                                |
| 155 | 578                                            | -106          | "                                | 975                                            | -239          | "                                | 470                                            | -238          | "                                |
| 156 | 425                                            | -9            | "                                | 977                                            | -238          | "                                | 492                                            | -241          | "                                |
| 157 | 615                                            | -120          | "                                | 982                                            | -240          | "                                | 470                                            | -238          | "                                |
| 158 | 469                                            | -20           | "                                | 974                                            | -239          | "                                | 492                                            | -241          | "                                |
| 159 | 846                                            | -221          | "                                | 1.01 × 10 <sup>3</sup>                         | -243          | "                                | 492                                            | -241          | "                                |
| 160 | 641                                            | -152          | "                                | 977                                            | -239          | "                                | 621                                            | -239          | "                                |
| 161 | 3.95 × 10 <sup>3</sup>                         | -212          | "                                | 8.94 × 10 <sup>3</sup>                         | -324          | "                                | 4.66 × 10 <sup>3</sup>                         | -677          | "                                |
| 162 | 3.23 × 10 <sup>3</sup>                         | -186          | "                                | 6.62 × 10 <sup>3</sup>                         | -295          | "                                | 3.51 × 10 <sup>3</sup>                         | -525          | "                                |
| 163 | 1.24 × 10 <sup>3</sup>                         | -152          | "                                | 4.63 × 10 <sup>3</sup>                         | -251          | "                                | 1.19 × 10 <sup>3</sup>                         | -400          | "                                |
| 164 | 886                                            | -82           | "                                | 1.64 × 10 <sup>3</sup>                         | -183          | "                                | 728                                            | -305          | "                                |
| 165 | 3.65 × 10 <sup>3</sup>                         | -205          | "                                | 6.49 × 10 <sup>3</sup>                         | -294          | "                                | 3.54 × 10 <sup>3</sup>                         | -520          | "                                |
| 166 | 2.02 × 10 <sup>3</sup>                         | -163          | "                                | 3.28 × 10 <sup>3</sup>                         | -198          | "                                | 1.22 × 10 <sup>3</sup>                         | -398          | "                                |
| 167 | 852                                            | -235          | "                                | 2.62 × 10 <sup>3</sup>                         | -498          | "                                | 4.12 × 10 <sup>3</sup>                         | -612          | "                                |
| 168 | 814                                            | -204          | "                                | 2.18 × 10 <sup>3</sup>                         | -352          | "                                | 983                                            | -354          | "                                |
| 169 | 605                                            | -113          | "                                | 1.94 × 10 <sup>3</sup>                         | -331          | "                                | 842                                            | -332          | "                                |
| 170 | 619                                            | -119          | "                                | 2.25 × 10 <sup>3</sup>                         | -397          | "                                | 1.19 × 10 <sup>3</sup>                         | -400          | "                                |
| 171 | 453                                            | -55           | "                                | 2.10 × 10 <sup>3</sup>                         | -357          | "                                | 983                                            | -354          | "                                |
| 172 | 449                                            | -51           | "                                | 1.65 × 10 <sup>3</sup>                         | -321          | "                                | 815                                            | -324          | "                                |
| 173 | 407                                            | -32           | "                                | 1.42 × 10 <sup>3</sup>                         | -304          | "                                | 734                                            | -307          | "                                |
| 174 | 634                                            | -124          | "                                | 2.24 × 10 <sup>3</sup>                         | -397          | "                                | 1.19 × 10 <sup>3</sup>                         | -400          | "                                |
| 175 | 463                                            | -60           | "                                | 1.70 × 10 <sup>3</sup>                         | -322          | "                                | 815                                            | -324          | "                                |
| 176 | 594                                            | -108          | "                                | 2.21 × 10 <sup>3</sup>                         | -396          | "                                | 1.19 × 10 <sup>3</sup>                         | -400          | "                                |
| 177 | 426                                            | -49           | "                                | 1.51 × 10 <sup>3</sup>                         | -320          | "                                | 815                                            | -324          | "                                |
| 178 | 581                                            | -94           | "                                | 2.28 × 10 <sup>3</sup>                         | -399          | "                                | 1.19 × 10 <sup>3</sup>                         | -400          | "                                |
| 179 | 407                                            | -35           | "                                | 1.60 × 10 <sup>3</sup>                         | -321          | "                                | 815                                            | -324          | "                                |
| 180 | 664                                            | -185          | "                                | 2.18 × 10 <sup>3</sup>                         | -369          | "                                | 997                                            | -400          | "                                |
| 181 | 499                                            | -115          | "                                | 1.99 × 10 <sup>3</sup>                         | -353          | "                                | 983                                            | -324          | "                                |
| 182 | 617                                            | -124          | "                                | 2.12 × 10 <sup>3</sup>                         | -367          | "                                | 997                                            | -368          | "                                |
| 183 | 469                                            | -100          | "                                | 2.10 × 10 <sup>3</sup>                         | -352          | "                                | 983                                            | -354          | "                                |
| 184 | 631                                            | -153          | "                                | 2.21 × 10 <sup>3</sup>                         | -370          | "                                | 997                                            | -368          | "                                |
| 185 | 481                                            | -85           | "                                | 2.09 × 10 <sup>3</sup>                         | -352          | "                                | 983                                            | -354          | "                                |
| 186 | 837                                            | -236          | "                                | 2.07 × 10 <sup>3</sup>                         | -356          | "                                | 983                                            | -354          | "                                |
| 187 | 639                                            | -169          | "                                | 2.30 × 10 <sup>3</sup>                         | -398          | "                                | 1.19 × 10 <sup>3</sup>                         | -400          | "                                |
| 188 | 592                                            | -83           | "                                | 1.03 × 10 <sup>3</sup>                         | -203          | "                                | 608                                            | -252          | "                                |
| 189 | 453                                            | -40           | "                                | 1.99 × 10 <sup>3</sup>                         | -338          | "                                | 906                                            | -341          | "                                |
| 190 | 875                                            | -109          | "                                | 1.58 × 10 <sup>3</sup>                         | -163          | "                                | 706                                            | +148          | "                                |
| 191 | 652                                            | -17           | "                                | 1.36 × 10 <sup>3</sup>                         | -124          | "                                | 518                                            | +287          | "                                |
| 192 | 426                                            | +74           | "                                | 924                                            | +320          | "                                | 270                                            | +401          | "                                |
| 193 | 349                                            | +108          | "                                | 763                                            | +263          | "                                | 196                                            | +428          | "                                |
| 194 | 775                                            | -28           | "                                | 1.40 × 10 <sup>3</sup>                         | +318          | "                                | 520                                            | +290          | "                                |
| 195 | 328                                            | +107          | "                                | 863                                            | +318          | "                                | 270                                            | +505          | "                                |
| 196 | 525                                            | +55           | "                                | 682                                            | +184          | "                                | 652                                            | +182          | "                                |
| 197 | 490                                            | +83           | "                                | 820                                            | +428          | "                                | 235                                            | +582          | "                                |
| 198 | 321                                            | +105          | "                                | 852                                            | +462          | "                                | 213                                            | +589          | "                                |
| 199 | 285                                            | +118          | "                                | 802                                            | +412          | "                                | 270                                            | +505          | "                                |
| 200 | 141                                            | +267          | "                                | 830                                            | +445          | "                                | 224                                            | +584          | "                                |
| 201 | 94                                             | +300          | "                                | 860                                            | +482          | "                                | 202                                            | +598          | "                                |
| 202 | 341                                            | +108          | "                                | 801                                            | +410          | "                                | 270                                            | +505          | "                                |
| 203 | 310                                            | +111          | "                                | 802                                            | +411          | "                                | 270                                            | +505          | "                                |
| 204 | 335                                            | +105          | "                                | 801                                            | +409          | "                                | 270                                            | +505          | "                                |
| 205 | 182                                            | +250          | "                                | 835                                            | +452          | "                                | 224                                            | +584          | "                                |
| 206 | 131                                            | +273          | "                                | 854                                            | +463          | "                                | 224                                            | +584          | "                                |
| 207 | 115                                            | +295          | "                                | 857                                            | +471          | "                                | 224                                            | +505          | "                                |
| 208 | 503                                            | +90           | "                                | 822                                            | +430          | "                                | 232                                            | +584          | "                                |
| 209 | 495                                            | +88           | "                                | 818                                            | +425          | "                                | 232                                            | +582          | "                                |
| 210 | 508                                            | +97           | "                                | 824                                            | +438          | "                                | 232                                            | +582          | "                                |
| 211 | 932                                            | -83           | "                                | 1.65 × 10 <sup>3</sup>                         | -164          | "                                | 761                                            | +108          | "                                |
| 212 | 729                                            | -65           | "                                | 1.29 × 10 <sup>3</sup>                         | -142          | "                                | 588                                            | +144          | "                                |
| 213 | 544                                            | +86           | "                                | 962                                            | +242          | "                                | 380                                            | +273          | "                                |
| 214 | 428                                            | +132          | "                                | 743                                            | +264          | "                                | 254                                            | +326          | "                                |
| 215 | 583                                            | +25           | "                                | 721                                            | +124          | "                                | 675                                            | +126          | "                                |
| 216 | 512                                            | +28           | "                                | 542                                            | +300          | "                                | 289                                            | +302          | "                                |
| 217 | 351                                            | +100          | "                                | 628                                            | +272          | "                                | 380                                            | +273          | "                                |
| 218 | 296                                            | +233          | "                                | 423                                            | +316          | "                                | 265                                            | +318          | "                                |
| 219 | 181                                            | +279          | "                                | 446                                            | +313          | "                                | 274                                            | +314          | "                                |
| 220 | 120                                            | +286          | "                                | 404                                            | +318          | "                                | 260                                            | +320          | "                                |
| 221 | 329                                            | +109          | "                                | 635                                            | +271          | "                                | 380                                            | +273          | "                                |
| 222 | 318                                            | +96           | "                                | 648                                            | +270          | "                                | 380                                            | +273          | "                                |
| 223 | 342                                            | +108          | "                                | 672                                            | +272          | "                                | 380                                            | +273          | "                                |
| 224 | 245                                            | +240          | "                                | 405                                            | +310          | "                                | 274                                            | +314          | "                                |
| 225 | 195                                            | +268          | "                                | 453                                            | +312          | "                                | 274                                            | +314          | "                                |
| 226 | 212                                            | +259          | "                                | 398                                            | +311          | "                                | 274                                            | +314          | "                                |

TABLE 10-continued

| Nos | Example 1                                      |               | Carbonate-Free                   |                                                |               |                                  | Carbonate & Fluoride-Free                      |               |                                  |
|-----|------------------------------------------------|---------------|----------------------------------|------------------------------------------------|---------------|----------------------------------|------------------------------------------------|---------------|----------------------------------|
|     | Resistance value at 25° C. R <sub>25</sub> (Ω) | TCR (ppm/°C.) | Rate of Change in Resistance (%) | Resistance value at 25° C. R <sub>25</sub> (Ω) | TCR (ppm/°C.) | Rate of Change in Resistance (%) | Resistance value at 25° C. R <sub>25</sub> (Ω) | TCR (ppm/°C.) | Rate of Change in Resistance (%) |
| 227 | 325                                            | +218          | "                                | 436                                            | +315          | "                                | 265                                            | +318          | "                                |
| 228 | 331                                            | +245          | "                                | 425                                            | +316          | "                                | 265                                            | +318          | "                                |
| 229 | 319                                            | +250          | "                                | 411                                            | +317          | "                                | 265                                            | +318          | "                                |
| 230 | 824                                            | -120          | "                                | 1.32 × 10 <sup>3</sup>                         | -216          | "                                | 645                                            | +107          | "                                |
| 231 | 536                                            | +31           | "                                | 824                                            | +103          | "                                | 415                                            | +209          | "                                |
| 232 | 743                                            | -21           | "                                | 1.28 × 10 <sup>3</sup>                         | +183          | "                                | 645                                            | +106          | "                                |
| 233 | 526                                            | +40           | "                                | 832                                            | +149          | "                                | 410                                            | +211          | "                                |
| 234 | 721                                            | -23           | "                                | 1.42 × 10 <sup>3</sup>                         | +156          | "                                | 528                                            | +158          | "                                |
| 235 | 605                                            | +12           | "                                | 868                                            | +360          | "                                | 239                                            | +362          | "                                |
| 236 | 433                                            | +183          | "                                | 1.02 × 10 <sup>3</sup>                         | +212          | "                                | 410                                            | +211          | "                                |
| 237 | 380                                            | +209          | "                                | 675                                            | +500          | "                                | 203                                            | +502          | "                                |
| 238 | 350                                            | +221          | "                                | 623                                            | +701          | "                                | 191                                            | +702          | "                                |
| 239 | 211                                            | +266          | "                                | 543                                            | +974          | "                                | 182                                            | +982          | "                                |
| 240 | 505                                            | +50           | "                                | 1.32 × 10 <sup>3</sup>                         | +208          | "                                | 410                                            | +211          | "                                |
| 241 | 450                                            | +61           | "                                | 1.14 × 10 <sup>3</sup>                         | +210          | "                                | 410                                            | +211          | "                                |
| 242 | 475                                            | +63           | "                                | 1.06 × 10 <sup>3</sup>                         | +211          | "                                | 410                                            | +211          | "                                |
| 243 | 405                                            | +179          | "                                | 652                                            | +698          | "                                | 191                                            | +702          | "                                |
| 244 | 386                                            | +205          | "                                | 620                                            | +701          | "                                | 191                                            | +702          | "                                |
| 245 | 421                                            | +185          | "                                | 640                                            | +699          | "                                | 191                                            | +702          | "                                |
| 246 | 383                                            | +207          | "                                | 682                                            | +484          | "                                | 208                                            | +486          | "                                |
| 247 | 422                                            | +199          | "                                | 924                                            | +302          | "                                | 396                                            | +304          | "                                |
| 248 | 639                                            | -161          | "                                | 583                                            | +105          | "                                | 354                                            | +294          | "                                |
| 249 | 17.5 × 10 <sup>3</sup>                         | -124          | "                                | 25.8 × 10 <sup>3</sup>                         | -321          | "                                | 18.6 × 10 <sup>3</sup>                         | -448          | "                                |
| 250 | 10.5 × 10 <sup>3</sup>                         | -79           | "                                | 16.7 × 10 <sup>3</sup>                         | -212          | "                                | 11.9 × 10 <sup>3</sup>                         | -507          | "                                |
| 251 | 5.29 × 10 <sup>3</sup>                         | -36           | "                                | 9.24 × 10 <sup>3</sup>                         | -143          | "                                | 4.88 × 10 <sup>3</sup>                         | -487          | "                                |
| 252 | 21.6 × 10 <sup>3</sup>                         | -144          | "                                | 32.3 × 10 <sup>3</sup>                         | -365          | "                                | 20.6 × 10 <sup>3</sup>                         | -449          | "                                |
| 253 | 1.98 × 10 <sup>3</sup>                         | +28           | "                                | 7.62 × 10 <sup>3</sup>                         | -62           | "                                | 2.30 × 10 <sup>3</sup>                         | -87           | "                                |
| 254 | 12.4 × 10 <sup>3</sup>                         | -106          | "                                | 15.6 × 10 <sup>3</sup>                         | -203          | "                                | 7.08 × 10 <sup>3</sup>                         | -328          | "                                |
| 255 | 17.9 × 10 <sup>3</sup>                         | -131          | "                                | 24.8 × 10 <sup>3</sup>                         | -272          | "                                | 16.6 × 10 <sup>3</sup>                         | -308          | "                                |
| 256 | 16.8 × 10 <sup>3</sup>                         | -129          | "                                | 22.9 × 10 <sup>3</sup>                         | -264          | "                                | 14.5 × 10 <sup>3</sup>                         | -381          | "                                |
| 257 | 6.88 × 10 <sup>3</sup>                         | -54           | "                                | 13.9 × 10 <sup>3</sup>                         | -179          | "                                | 6.21 × 10 <sup>3</sup>                         | -422          | "                                |
| 258 | 6.02 × 10 <sup>3</sup>                         | -42           | "                                | 11.2 × 10 <sup>3</sup>                         | -158          | "                                | 5.49 × 10 <sup>3</sup>                         | -456          | "                                |
| 259 | 13.2 × 10 <sup>3</sup>                         | -109          | "                                | 22.4 × 10 <sup>3</sup>                         | -252          | "                                | 12.2 × 10 <sup>3</sup>                         | -470          | "                                |
| 260 | 16.4 × 10 <sup>3</sup>                         | -120          | "                                | 23.8 × 10 <sup>3</sup>                         | -270          | "                                | 14.6 × 10 <sup>3</sup>                         | -485          | "                                |
| 261 | 18.6 × 10 <sup>3</sup>                         | -128          | "                                | 42.6 × 10 <sup>3</sup>                         | -391          | "                                | 27.4 × 10 <sup>3</sup>                         | -641          | "                                |
| 262 | 9.64 × 10 <sup>3</sup>                         | -94           | "                                | 17.9 × 10 <sup>3</sup>                         | -224          | "                                | 8.61 × 10 <sup>3</sup>                         | -588          | "                                |
| 263 | 2.39 × 10 <sup>3</sup>                         | +15           | "                                | 6.93 × 10 <sup>3</sup>                         | -891          | "                                | 2.19 × 10 <sup>3</sup>                         | -501          | "                                |
| 264 | 1.68 × 10 <sup>3</sup>                         | +32           | "                                | 4.83 × 10 <sup>3</sup>                         | -521          | "                                | 1.55 × 10 <sup>3</sup>                         | +57           | "                                |
| 265 | -18.7 × 10 <sup>3</sup>                        | -222          | "                                | 24.5 × 10 <sup>3</sup>                         | -342          | "                                | 16.3 × 10 <sup>3</sup>                         | -342          | "                                |
| 266 | 8.38 × 10 <sup>3</sup>                         | -124          | "                                | 10.6 × 10 <sup>3</sup>                         | -296          | "                                | 7.35 × 10 <sup>3</sup>                         | -296          | "                                |
| 267 | 624                                            | +10           | "                                | 928                                            | -42           | "                                | 483                                            | -42           | "                                |
| 268 | 921                                            | +35           | "                                | 1.03 × 10 <sup>3</sup>                         | -28           | "                                | 826                                            | -28           | "                                |
| 269 | 3.21 × 10 <sup>3</sup>                         | -89           | "                                | 4.28 × 10 <sup>3</sup>                         | -251          | "                                | 2.38 × 10 <sup>3</sup>                         | -251          | "                                |
| 270 | 3.3 × 10 <sup>3</sup>                          | -98           | "                                | 4.93 × 10 <sup>3</sup>                         | -124          | "                                | 2.88 × 10 <sup>3</sup>                         | -256          | "                                |
| 271 | 7.46 × 10 <sup>3</sup>                         | -169          | "                                | 18.3 × 10 <sup>3</sup>                         | -405          | "                                | 16.6 × 10 <sup>3</sup>                         | -546          | "                                |
| 272 | 1.39 × 10 <sup>3</sup>                         | -132          | "                                | 8.11 × 10 <sup>3</sup>                         | -216          | "                                | 14.5 × 10 <sup>3</sup>                         | -367          | "                                |
| 273 | 342                                            | +23           | "                                | 560                                            | -51           | "                                | 6.21 × 10 <sup>3</sup>                         | -44           | "                                |
| 274 | 694                                            | -41           | "                                | 925                                            | -88           | "                                | 5.49 × 10 <sup>3</sup>                         | -109          | "                                |
| 275 | 1.54 × 10 <sup>3</sup>                         | -142          | "                                | 3.00 × 10 <sup>3</sup>                         | -295          | "                                | 12.2 × 10 <sup>3</sup>                         | -381          | "                                |
| 276 | 1.03 × 10 <sup>3</sup>                         | -95           | "                                | 3.49 × 10 <sup>3</sup>                         | -186          | "                                | 14.6 × 10 <sup>3</sup>                         | -242          | "                                |

TABLE 11

| Nos | Example 1                                      |               | Carbonate-Free                   |                                                |               |                                  | Carbonate & Fluoride-Free                      |               |                                  |
|-----|------------------------------------------------|---------------|----------------------------------|------------------------------------------------|---------------|----------------------------------|------------------------------------------------|---------------|----------------------------------|
|     | Resistance value at 25° C. R <sub>25</sub> (Ω) | TCR (ppm/°C.) | Rate of Change in Resistance (%) | Resistance value at 25° C. R <sub>25</sub> (Ω) | TCR (ppm/°C.) | Rate of Change in Resistance (%) | Resistance value at 25° C. R <sub>25</sub> (Ω) | TCR (ppm/°C.) | Rate of Change in Resistance (%) |
| 1   | 9.23 × 10 <sup>3</sup>                         | -48           | <±2                              | 15.2 × 10 <sup>3</sup>                         | -268          | <±2                              | 8.78 × 10 <sup>3</sup>                         | -916          | <±2                              |
| 2   | 5.69 × 10 <sup>3</sup>                         | +21           | "                                | 7.94 × 10 <sup>3</sup>                         | -196          | "                                | 5.10 × 10 <sup>3</sup>                         | -522          | "                                |
| 3   | 3.48 × 10 <sup>3</sup>                         | +163          | "                                | 4.22 × 10 <sup>3</sup>                         | -154          | "                                | 3.16 × 10 <sup>3</sup>                         | -398          | "                                |
| 4   | 3.16 × 10 <sup>3</sup>                         | +125          | "                                | 4.09 × 10 <sup>3</sup>                         | -150          | "                                | 3.05 × 10 <sup>3</sup>                         | -216          | "                                |
| 5   | 5.74 × 10 <sup>3</sup>                         | +12           | "                                | 8.26 × 10 <sup>3</sup>                         | -214          | "                                | 5.17 × 10 <sup>3</sup>                         | -529          | "                                |
| 6   | 3.52 × 10 <sup>3</sup>                         | +174          | "                                | 6.13 × 10 <sup>3</sup>                         | -189          | "                                | 3.22 × 10 <sup>3</sup>                         | -402          | "                                |
| 7   | 5.48 × 10 <sup>3</sup>                         | +36           | "                                | 5.63 × 10 <sup>3</sup>                         | -171          | "                                | 5.01 × 10 <sup>3</sup>                         | -516          | "                                |
| 8   | 5.16 × 10 <sup>3</sup>                         | +38           | "                                | 5.49 × 10 <sup>3</sup>                         | -170          | "                                | 2.82 × 10 <sup>3</sup>                         | -201          | "                                |
| 9   | 3.15 × 10 <sup>3</sup>                         | +126          | "                                | 4.98 × 10 <sup>3</sup>                         | -166          | "                                | 2.73 × 10 <sup>3</sup>                         | -185          | "                                |
| 10  | 3.23 × 10 <sup>3</sup>                         | +150          | "                                | 5.16 × 10 <sup>3</sup>                         | -167          | "                                | 3.04 × 10 <sup>3</sup>                         | -215          | "                                |
| 11  | 2.84 × 10 <sup>3</sup>                         | +195          | "                                | 4.62 × 10 <sup>3</sup>                         | -162          | "                                | 2.65 × 10 <sup>3</sup>                         | -177          | "                                |
| 12  | 2.46 × 10 <sup>3</sup>                         | +242          | "                                | 4.41 × 10 <sup>3</sup>                         | -161          | "                                | 2.62 × 10 <sup>3</sup>                         | -175          | "                                |
| 13  | 5.88 × 10 <sup>3</sup>                         | +7            | "                                | 6.02 × 10 <sup>3</sup>                         | -191          | "                                | 2.82 × 10 <sup>3</sup>                         | -201          | "                                |

TABLE 11-continued

| (Characteristic values corresponding to the sample in Table 3) |                            |                              |                            |                              |                            |                              |
|----------------------------------------------------------------|----------------------------|------------------------------|----------------------------|------------------------------|----------------------------|------------------------------|
| Nos                                                            | Example 1                  |                              | Carbonate-Free             |                              | Carbonate & Fluoride-Free  |                              |
|                                                                | Resistance value at 25° C. | Rate of Change in Resistance | Resistance value at 25° C. | Rate of Change in Resistance | Resistance value at 25° C. | Rate of Change in Resistance |
|                                                                | R <sub>25</sub> (Ω)        | TCR (ppm/°C.)                | R <sub>25</sub> (Ω)        | TCR (ppm/°C.)                | R <sub>25</sub> (Ω)        | TCR (ppm/°C.)                |
| 14                                                             | $4.21 \times 10^3$         | +108                         | "                          | $5.81 \times 10^3$           | -172                       | "                            |
| 15                                                             | $4.92 \times 10^3$         | +43                          | "                          | $6.11 \times 10^3$           | -198                       | "                            |
| 16                                                             | $3.00 \times 10^3$         | +161                         | "                          | $5.99 \times 10^3$           | -182                       | "                            |
| 17                                                             | $5.38 \times 10^3$         | +34                          | "                          | $6.15 \times 10^3$           | -199                       | "                            |
| 18                                                             | $3.81 \times 10^3$         | +136                         | "                          | $6.01 \times 10^3$           | -188                       | "                            |
| 19                                                             | $2.84 \times 10^3$         | +167                         | "                          | $5.85 \times 10^3$           | -180                       | "                            |
| 20                                                             | $2.40 \times 10^3$         | +193                         | "                          | $5.65 \times 10^3$           | -173                       | "                            |
| 21                                                             | $2.69 \times 10^3$         | +181                         | "                          | $5.84 \times 10^3$           | -178                       | "                            |
| 22                                                             | $2.18 \times 10^3$         | +180                         | "                          | $5.62 \times 10^3$           | -171                       | "                            |
| 23                                                             | $3.08 \times 10^3$         | +130                         | "                          | $5.88 \times 10^3$           | -181                       | "                            |
| 24                                                             | $2.61 \times 10^3$         | +185                         | "                          | $5.67 \times 10^3$           | -174                       | "                            |
| 25                                                             | $3.40 \times 10^3$         | +151                         | "                          | $6.19 \times 10^3$           | -209                       | "                            |
| 26                                                             | $2.99 \times 10^3$         | +203                         | "                          | $6.22 \times 10^3$           | -211                       | "                            |
| 27                                                             | $3.08 \times 10^3$         | +176                         | "                          | $6.25 \times 10^3$           | -214                       | "                            |
| 28                                                             | $8.72 \times 10^3$         | -62                          | "                          | $14.3 \times 10^3$           | -278                       | "                            |
| 29                                                             | $5.11 \times 10^3$         | +119                         | "                          | $11.2 \times 10^3$           | -257                       | "                            |
| 30                                                             | $2.92 \times 10^3$         | +267                         | "                          | $8.92 \times 10^3$           | -148                       | "                            |
| 31                                                             | $2.89 \times 10^3$         | +246                         | "                          | $5.71 \times 10^3$           | -92                        | "                            |
| 32                                                             | $4.94 \times 10^3$         | +205                         | "                          | $9.96 \times 10^3$           | -246                       | "                            |
| 33                                                             | $3.09 \times 10^3$         | +167                         | "                          | $7.23 \times 10^3$           | -104                       | "                            |
| 34                                                             | $4.89 \times 10^3$         | +103                         | "                          | $6.21 \times 10^3$           | -490                       | "                            |
| 35                                                             | $4.57 \times 10^3$         | +96                          | "                          | $5.31 \times 10^3$           | -243                       | "                            |
| 36                                                             | $2.66 \times 10^3$         | +145                         | "                          | $3.68 \times 10^3$           | -216                       | "                            |
| 37                                                             | $2.74 \times 10^3$         | +149                         | "                          | $5.52 \times 10^3$           | -258                       | "                            |
| 38                                                             | $2.33 \times 10^3$         | +189                         | "                          | $4.86 \times 10^3$           | -234                       | "                            |
| 39                                                             | $1.97 \times 10^3$         | +240                         | "                          | $3.32 \times 10^3$           | -207                       | "                            |
| 40                                                             | $5.03 \times 10^3$         | +65                          | "                          | $5.21 \times 10^3$           | -239                       | "                            |
| 41                                                             | $3.23 \times 10^3$         | +128                         | "                          | $5.83 \times 10^3$           | -264                       | "                            |
| 42                                                             | $4.71 \times 10^3$         | +95                          | "                          | $5.25 \times 10^3$           | -240                       | "                            |
| 43                                                             | $2.89 \times 10^3$         | +139                         | "                          | $5.75 \times 10^3$           | -261                       | "                            |
| 44                                                             | $4.88 \times 10^3$         | +81                          | "                          | $4.98 \times 10^3$           | -238                       | "                            |
| 45                                                             | $3.05 \times 10^3$         | +129                         | "                          | $5.67 \times 10^3$           | -259                       | "                            |
| 46                                                             | $3.20 \times 10^3$         | +103                         | "                          | $4.65 \times 10^3$           | -225                       | "                            |
| 47                                                             | $2.87 \times 10^3$         | +151                         | "                          | $4.61 \times 10^3$           | -235                       | "                            |
| 48                                                             | $2.44 \times 10^3$         | +140                         | "                          | $3.81 \times 10^3$           | -220                       | "                            |
| 49                                                             | $2.08 \times 10^3$         | +183                         | "                          | $4.77 \times 10^3$           | -233                       | "                            |
| 50                                                             | $2.85 \times 10^3$         | +160                         | "                          | $4.68 \times 10^3$           | -227                       | "                            |
| 51                                                             | $2.54 \times 10^3$         | +179                         | "                          | $4.87 \times 10^3$           | -234                       | "                            |
| 52                                                             | $4.68 \times 10^3$         | +89                          | "                          | $5.30 \times 10^3$           | -243                       | "                            |
| 53                                                             | $4.70 \times 10^3$         | +95                          | "                          | $5.32 \times 10^3$           | -245                       | "                            |
| 54                                                             | $4.77 \times 10^3$         | +78                          | "                          | $5.46 \times 10^3$           | -261                       | "                            |
| 55                                                             | $7.16 \times 10^3$         | -163                         | "                          | $9.33 \times 10^3$           | -462                       | "                            |
| 56                                                             | $4.81 \times 10^3$         | -82                          | "                          | $6.42 \times 10^3$           | -419                       | "                            |
| 57                                                             | $7.22 \times 10^3$         | -184                         | "                          | $10.2 \times 10^3$           | -497                       | "                            |
| 58                                                             | $4.93 \times 10^3$         | -93                          | "                          | $7.21 \times 10^3$           | -444                       | "                            |
| 59                                                             | $6.13 \times 10^3$         | -121                         | "                          | $8.25 \times 10^3$           | -498                       | "                            |
| 60                                                             | $6.01 \times 10^3$         | -105                         | "                          | $8.43 \times 10^3$           | -499                       | "                            |
| 61                                                             | $3.87 \times 10^3$         | +53                          | "                          | $7.91 \times 10^3$           | -497                       | "                            |
| 62                                                             | $3.62 \times 10^3$         | +77                          | "                          | $7.62 \times 10^3$           | -496                       | "                            |
| 63                                                             | $3.14 \times 10^3$         | +68                          | "                          | $6.41 \times 10^3$           | -490                       | "                            |
| 64                                                             | $3.00 \times 10^3$         | +85                          | "                          | $6.15 \times 10^3$           | -489                       | "                            |
| 65                                                             | $6.24 \times 10^3$         | -135                         | "                          | $7.32 \times 10^3$           | -495                       | "                            |
| 66                                                             | $4.07 \times 10^3$         | +5                           | "                          | $7.04 \times 10^3$           | -494                       | "                            |
| 67                                                             | $5.85 \times 10^3$         | -85                          | "                          | $6.02 \times 10^3$           | -488                       | "                            |
| 68                                                             | $3.41 \times 10^3$         | +58                          | "                          | $6.52 \times 10^3$           | -491                       | "                            |
| 69                                                             | $5.67 \times 10^3$         | -18                          | "                          | $5.88 \times 10^3$           | -487                       | "                            |
| 70                                                             | $3.29 \times 10^3$         | +60                          | "                          | $5.06 \times 10^3$           | -472                       | "                            |
| 71                                                             | $4.33 \times 10^3$         | -52                          | "                          | $6.83 \times 10^3$           | -493                       | "                            |
| 72                                                             | $3.68 \times 10^3$         | +21                          | "                          | $6.39 \times 10^3$           | -490                       | "                            |
| 73                                                             | $3.99 \times 10^3$         | +18                          | "                          | $4.86 \times 10^3$           | -468                       | "                            |
| 74                                                             | $3.31 \times 10^3$         | +28                          | "                          | $5.25 \times 10^3$           | -478                       | "                            |
| 75                                                             | $4.18 \times 10^3$         | -20                          | "                          | $5.06 \times 10^3$           | -472                       | "                            |
| 76                                                             | $3.54 \times 10^3$         | +40                          | "                          | $4.72 \times 10^3$           | -479                       | "                            |
| 77                                                             | $3.08 \times 10^3$         | +72                          | "                          | $5.61 \times 10^3$           | -481                       | "                            |
| 78                                                             | $3.20 \times 10^3$         | +70                          | "                          | $5.24 \times 10^3$           | -478                       | "                            |
| 79                                                             | $3.49 \times 10^3$         | +20                          | "                          | $5.16 \times 10^3$           | -476                       | "                            |
| 80                                                             | $3.10 \times 10^3$         | +166                         | "                          | $4.74 \times 10^3$           | -467                       | "                            |
| 81                                                             | $4.02 \times 10^3$         | +172                         | "                          | $6.14 \times 10^3$           | -492                       | "                            |
| 82                                                             | $3.48 \times 10^3$         | +159                         | "                          | $3.98 \times 10^3$           | -398                       | "                            |
| 83                                                             | $3.84 \times 10^3$         | +144                         | "                          | $4.52 \times 10^3$           | -456                       | "                            |

TABLE 12

(Characteristic values corresponding to the sample in Table 4)

| Nos | Example 1                  |                              |                            | Carbonate-Free             |                              |                            | Carbonate & Fluoride-Free  |                              |                            |
|-----|----------------------------|------------------------------|----------------------------|----------------------------|------------------------------|----------------------------|----------------------------|------------------------------|----------------------------|
|     | Resistance value at 25° C. | Rate of Change in Resistance | Resistance value at 25° C. | Resistance value at 25° C. | Rate of Change in Resistance | Resistance value at 25° C. | Resistance value at 25° C. | Rate of Change in Resistance | Resistance value at 25° C. |
|     | R <sub>25</sub> (Ω)        | TCR (ppm/°C.)                | (%)                        | R <sub>25</sub> (Ω)        | TCR (ppm/°C.)                | (%)                        | R <sub>25</sub> (Ω)        | TCR (ppm/°C.)                | (%)                        |
| 1   | $20.3 \times 10^3$         | -289                         | < $\pm 2$                  | $26.3 \times 10^3$         | -986                         | < $\pm 2$                  | $25.4 \times 10^3$         | -986                         | < $\pm 2$                  |
| 2   | $17.5 \times 10^3$         | -278                         | "                          | $22.5 \times 10^3$         | -877                         | "                          | $21.7 \times 10^3$         | -877                         | "                          |
| 3   | $13.2 \times 10^3$         | -252                         | "                          | $19.3 \times 10^3$         | -805                         | "                          | $18.4 \times 10^3$         | -805                         | "                          |
| 4   | $5.34 \times 10^3$         | -190                         | "                          | $10.3 \times 10^3$         | -681                         | "                          | $9.26 \times 10^3$         | -681                         | "                          |
| 5   | $21.5 \times 10^3$         | -285                         | "                          | $27.5 \times 10^3$         | -995                         | "                          | $26.4 \times 10^3$         | -995                         | "                          |
| 6   | $18.4 \times 10^3$         | -275                         | "                          | $23.1 \times 10^3$         | -880                         | "                          | $22.3 \times 10^3$         | -880                         | "                          |
| 7   | $14.9 \times 10^3$         | -250                         | "                          | $19.8 \times 10^3$         | -803                         | "                          | $19.0 \times 10^3$         | -803                         | "                          |
| 8   | $4.25 \times 10^3$         | -187                         | "                          | $10.1 \times 10^3$         | -684                         | "                          | $9.77 \times 10^3$         | -684                         | "                          |
| 9   | $15.3 \times 10^3$         | -265                         | "                          | $19.2 \times 10^3$         | -804                         | "                          | $18.8 \times 10^3$         | -804                         | "                          |
| 10  | $15.1 \times 10^3$         | -285                         | "                          | $23.6 \times 10^3$         | -418                         | "                          | $21.4 \times 10^3$         | -842                         | "                          |
| 11  | $13.9 \times 10^3$         | -249                         | "                          | $16.4 \times 10^3$         | -376                         | "                          | $17.3 \times 10^3$         | -794                         | "                          |
| 12  | $11.5 \times 10^3$         | -218                         | "                          | $15.2 \times 10^3$         | -351                         | "                          | $14.6 \times 10^3$         | -693                         | "                          |
| 13  | $9.84 \times 10^3$         | -205                         | "                          | $17.6 \times 10^3$         | -402                         | "                          | $16.9 \times 10^3$         | -761                         | "                          |
| 14  | $8.07 \times 10^3$         | -188                         | "                          | $9.31 \times 10^3$         | -598                         | "                          | $9.48 \times 10^3$         | -652                         | "                          |
| 15  | $16.3 \times 10^3$         | -297                         | "                          | $20.3 \times 10^3$         | -783                         | "                          | $21.4 \times 10^3$         | -842                         | "                          |
| 16  | $14.7 \times 10^3$         | -259                         | "                          | $16.8 \times 10^3$         | -428                         | "                          | $17.3 \times 10^3$         | -794                         | "                          |
| 17  | $12.7 \times 10^3$         | -231                         | "                          | $15.4 \times 10^3$         | -398                         | "                          | $14.6 \times 10^3$         | -693                         | "                          |
| 18  | $10.4 \times 10^3$         | -227                         | "                          | $14.9 \times 10^3$         | -372                         | "                          | $16.9 \times 10^3$         | -761                         | "                          |
| 19  | $8.65 \times 10^3$         | -205                         | "                          | $9.72 \times 10^3$         | -481                         | "                          | $9.48 \times 10^3$         | -652                         | "                          |
| 20  | $13.9 \times 10^3$         | -261                         | "                          | $15.2 \times 10^3$         | -384                         | "                          | $14.6 \times 10^3$         | -693                         | "                          |
| 21  | $13.4 \times 10^3$         | -268                         | "                          | $15.8 \times 10^3$         | -402                         | "                          | $16.9 \times 10^3$         | -761                         | "                          |
| 22  | $12.3 \times 10^3$         | -242                         | "                          | $14.4 \times 10^3$         | -369                         | "                          | $14.6 \times 10^3$         | -693                         | "                          |
| 23  | $10.7 \times 10^3$         | -225                         | "                          | $15.5 \times 10^3$         | -401                         | "                          | $16.9 \times 10^3$         | -761                         | "                          |
| 24  | $12.9 \times 10^3$         | -243                         | "                          | $13.9 \times 10^3$         | -340                         | "                          | $14.6 \times 10^3$         | -693                         | "                          |
| 25  | $11.8 \times 10^3$         | -236                         | "                          | $15.1 \times 10^3$         | -377                         | "                          | $16.9 \times 10^3$         | -761                         | "                          |
| 26  | $12.7 \times 10^3$         | -240                         | "                          | $14.2 \times 10^3$         | -358                         | "                          | $14.6 \times 10^3$         | -693                         | "                          |
| 27  | $10.7 \times 10^3$         | -235                         | "                          | $14.9 \times 10^3$         | -373                         | "                          | $16.9 \times 10^3$         | -761                         | "                          |
| 28  | $10.4 \times 10^3$         | -205                         | "                          | $14.3 \times 10^3$         | -364                         | "                          | $14.6 \times 10^3$         | -693                         | "                          |
| 29  | $9.12 \times 10^3$         | -207                         | "                          | $15.9 \times 10^3$         | -418                         | "                          | $16.9 \times 10^3$         | -761                         | "                          |
| 30  | $9.03 \times 10^3$         | -198                         | "                          | $14.5 \times 10^3$         | -370                         | "                          | $14.6 \times 10^3$         | -693                         | "                          |
| 31  | $8.88 \times 10^3$         | -191                         | "                          | $13.4 \times 10^3$         | -314                         | "                          | $16.9 \times 10^3$         | -761                         | "                          |
| 32  | $12.6 \times 10^3$         | -243                         | "                          | $15.8 \times 10^3$         | -404                         | "                          | $14.6 \times 10^3$         | -693                         | "                          |
| 33  | $11.4 \times 10^3$         | -222                         | "                          | $13.6 \times 10^3$         | -318                         | "                          | $14.6 \times 10^3$         | -693                         | "                          |
| 34  | $13.8 \times 10^3$         | -261                         | "                          | $14.9 \times 10^3$         | -382                         | "                          | $14.6 \times 10^3$         | -693                         | "                          |
| 35  | $9.73 \times 10^3$         | -209                         | "                          | $15.2 \times 10^3$         | -383                         | "                          | $16.9 \times 10^3$         | -761                         | "                          |

TABLE 13

(Characteristic values corresponding to the sample in Table 5)

| Nos | Example 1                  |                              |                            | Carbonate-Free             |                              |                            | Carbonate & Fluoride-Free  |                              |                            |
|-----|----------------------------|------------------------------|----------------------------|----------------------------|------------------------------|----------------------------|----------------------------|------------------------------|----------------------------|
|     | Resistance value at 25° C. | Rate of Change in Resistance | Resistance value at 25° C. | Resistance value at 25° C. | Rate of Change in Resistance | Resistance value at 25° C. | Resistance value at 25° C. | Rate of Change in Resistance | Resistance value at 25° C. |
|     | R <sub>25</sub> (Ω)        | TCR (ppm/°C.)                | (%)                        | R <sub>25</sub> (Ω)        | TCR (ppm/°C.)                | (%)                        | R <sub>25</sub> (Ω)        | TCR (ppm/°C.)                | (%)                        |
| 1   | $48.3 \times 10^3$         | -298                         | < $\pm 2$                  | $53.8 \times 10^3$         | -483                         | < $\pm 2$                  | $52.5 \times 10^3$         | -877                         | < $\pm 2$                  |
| 2   | $14.8 \times 10^3$         | -273                         | "                          | $19.5 \times 10^3$         | -395                         | "                          | $18.9 \times 10^3$         | -580                         | "                          |
| 3   | $2.54 \times 10^3$         | -93                          | "                          | $6.23 \times 10^3$         | -315                         | "                          | $5.81 \times 10^3$         | -416                         | "                          |
| 4   | $2.19 \times 10^3$         | -90                          | "                          | $3.15 \times 10^3$         | -310                         | "                          | $2.30 \times 10^3$         | -304                         | "                          |
| 5   | $16.2 \times 10^3$         | -279                         | "                          | $20.5 \times 10^3$         | -403                         | "                          | $19.3 \times 10^3$         | -576                         | "                          |
| 6   | $2.80 \times 10^3$         | -95                          | "                          | $6.34 \times 10^3$         | -392                         | "                          | $5.79 \times 10^3$         | -415                         | "                          |
| 7   | $20.1 \times 10^3$         | -292                         | "                          | $26.3 \times 10^3$         | -425                         | "                          | $25.3 \times 10^3$         | -685                         | "                          |
| 8   | $18.5 \times 10^3$         | -281                         | "                          | $22.1 \times 10^3$         | -410                         | "                          | $21.6 \times 10^3$         | -675                         | "                          |
| 9   | $8.78 \times 10^3$         | -195                         | "                          | $9.56 \times 10^3$         | -380                         | "                          | $9.26 \times 10^3$         | -525                         | "                          |
| 10  | $7.96 \times 10^3$         | -197                         | "                          | $9.02 \times 10^3$         | -378                         | "                          | $8.92 \times 10^3$         | -518                         | "                          |
| 11  | $2.01 \times 10^3$         | -105                         | "                          | $3.25 \times 10^3$         | -309                         | "                          | $3.03 \times 10^3$         | -403                         | "                          |
| 12  | $2.00 \times 10^3$         | -98                          | "                          | $2.89 \times 10^3$         | -305                         | "                          | $2.84 \times 10^3$         | -398                         | "                          |
| 13  | $1.12 \times 10^3$         | -45                          | "                          | $2.18 \times 10^3$         | -303                         | "                          | $2.13 \times 10^3$         | -387                         | "                          |
| 14  | $24.3 \times 10^3$         | -298                         | "                          | $26.9 \times 10^3$         | -432                         | "                          | $25.3 \times 10^3$         | -685                         | "                          |
| 15  | $21.8 \times 10^3$         | -290                         | "                          | $23.0 \times 10^3$         | -415                         | "                          | $21.6 \times 10^3$         | -675                         | "                          |
| 16  | $9.95 \times 10^3$         | -225                         | "                          | $9.82 \times 10^3$         | -392                         | "                          | $9.26 \times 10^3$         | -525                         | "                          |
| 17  | $9.03 \times 10^3$         | -221                         | "                          | $9.03 \times 10^3$         | -381                         | "                          | $8.92 \times 10^3$         | -518                         | "                          |
| 18  | $4.68 \times 10^3$         | -185                         | "                          | $3.25 \times 10^3$         | -363                         | "                          | $3.03 \times 10^3$         | -403                         | "                          |
| 19  | $4.41 \times 10^3$         | -168                         | "                          | $3.01 \times 10^3$         | -314                         | "                          | $2.84 \times 10^3$         | -398                         | "                          |
| 20  | $1.85 \times 10^3$         | -62                          | "                          | $2.21 \times 10^3$         | -309                         | "                          | $2.13 \times 10^3$         | -387                         | "                          |
| 21  | $10.08 \times 10^3$        | -223                         | "                          | $9.83 \times 10^3$         | -392                         | "                          | $9.26 \times 10^3$         | -525                         | "                          |
| 22  | $2.38 \times 10^3$         | -114                         | "                          | $3.21 \times 10^3$         | -365                         | "                          | $3.03 \times 10^3$         | -403                         | "                          |
| 23  | $8.14 \times 10^3$         | -186                         | "                          | $9.56 \times 10^3$         | -353                         | "                          | $9.26 \times 10^3$         | -525                         | "                          |
| 24  | $1.95 \times 10^3$         | -106                         | "                          | $3.14 \times 10^3$         | -358                         | "                          | $3.03 \times 10^3$         | -403                         | "                          |
| 25  | $7.68 \times 10^3$         | -181                         | "                          | $9.54 \times 10^3$         | -393                         | "                          | $9.26 \times 10^3$         | -525                         | "                          |
| 26  | $1.88 \times 10^3$         | -99                          | "                          | $3.17 \times 10^3$         | -374                         | "                          | $3.03 \times 10^3$         | -403                         | "                          |
| 27  | $9.84 \times 10^3$         | -200                         | "                          | $9.02 \times 10^3$         | -362                         | "                          | $8.92 \times 10^3$         | -518                         | "                          |

TABLE 13-continued

| Nos | Example 1                  |                              | Carbonate-Free             |                              |                            |                              | Carbonate & Fluoride-Free  |                              |                            |                              |
|-----|----------------------------|------------------------------|----------------------------|------------------------------|----------------------------|------------------------------|----------------------------|------------------------------|----------------------------|------------------------------|
|     | Resistance value at 25° C. | Rate of Change in Resistance | Resistance value at 25° C. | Rate of Change in Resistance | Resistance value at 25° C. | Rate of Change in Resistance | Resistance value at 25° C. | Rate of Change in Resistance | Resistance value at 25° C. | Rate of Change in Resistance |
|     | R <sub>25</sub> (Ω)        | TCR (ppm/°C.)                | R <sub>25</sub> (Ω)        | TCR (ppm/°C.)                | R <sub>25</sub> (Ω)        | TCR (ppm/°C.)                | R <sub>25</sub> (Ω)        | TCR (ppm/°C.)                | R <sub>25</sub> (Ω)        | TCR (ppm/°C.)                |
| 28  | $3.01 \times 10^3$         | -141                         | "                          | $2.92 \times 10^3$           | -316                       | "                            | $2.84 \times 10^3$         | -398                         | "                          | "                            |
| 29  | $8.16 \times 10^3$         | -184                         | "                          | $9.21 \times 10^3$           | -321                       | "                            | $8.92 \times 10^3$         | -518                         | "                          | "                            |
| 30  | $2.18 \times 10^3$         | -120                         | "                          | $2.90 \times 10^3$           | -316                       | "                            | $2.84 \times 10^3$         | -398                         | "                          | "                            |
| 31  | $8.78 \times 10^3$         | -188                         | "                          | $8.98 \times 10^3$           | -321                       | "                            | $8.92 \times 10^3$         | -518                         | "                          | "                            |
| 32  | $2.54 \times 10^3$         | -121                         | "                          | $2.96 \times 10^3$           | -319                       | "                            | $2.84 \times 10^3$         | -398                         | "                          | "                            |
| 33  | $17.4 \times 10^3$         | -277                         | "                          | $21.9 \times 10^3$           | -403                       | "                            | $21.6 \times 10^3$         | -675                         | "                          | "                            |
| 34  | $18.9 \times 10^3$         | -289                         | "                          | $22.0 \times 10^3$           | -410                       | "                            | $21.6 \times 10^3$         | -675                         | "                          | "                            |
| 35  | $43.9 \times 10^3$         | -297                         | "                          | $45.6 \times 10^3$           | -463                       | "                            | $44.8 \times 10^3$         | -857                         | "                          | "                            |
| 36  | $14.8 \times 10^3$         | -261                         | "                          | $16.3 \times 10^3$           | -405                       | "                            | $15.0 \times 10^3$         | -521                         | "                          | "                            |
| 37  | $4.13 \times 10^3$         | -180                         | "                          | $5.34 \times 10^3$           | -362                       | "                            | $4.77 \times 10^3$         | -408                         | "                          | "                            |
| 38  | $1.93 \times 10^3$         | -120                         | "                          | $3.51 \times 10^3$           | -354                       | "                            | $2.07 \times 10^3$         | -311                         | "                          | "                            |
| 39  | $14.8 \times 10^3$         | -273                         | "                          | $17.5 \times 10^3$           | -413                       | "                            | $15.3 \times 10^3$         | -527                         | "                          | "                            |
| 40  | $4.24 \times 10^3$         | -186                         | "                          | $5.83 \times 10^3$           | -372                       | "                            | $4.80 \times 10^3$         | -411                         | "                          | "                            |
| 41  | $18.2 \times 10^3$         | -271                         | "                          | $19.8 \times 10^3$           | -412                       | "                            | $19.4 \times 10^3$         | -621                         | "                          | "                            |
| 42  | $16.4 \times 10^3$         | -254                         | "                          | $18.6 \times 10^3$           | -408                       | "                            | $18.2 \times 10^3$         | -613                         | "                          | "                            |
| 43  | $6.85 \times 10^3$         | -186                         | "                          | $7.82 \times 10^3$           | -395                       | "                            | $7.32 \times 10^3$         | -480                         | "                          | "                            |
| 44  | $6.18 \times 10^3$         | -184                         | "                          | $7.53 \times 10^3$           | -389                       | "                            | $7.01 \times 10^3$         | -478                         | "                          | "                            |
| 45  | $2.81 \times 10^3$         | -125                         | "                          | $3.43 \times 10^3$           | -325                       | "                            | $3.24 \times 10^3$         | -411                         | "                          | "                            |
| 46  | $2.16 \times 10^3$         | -118                         | "                          | $3.21 \times 10^3$           | -320                       | "                            | $3.02 \times 10^3$         | -408                         | "                          | "                            |
| 47  | 985                        | -15                          | "                          | $1.53 \times 10^3$           | -302                       | "                            | $1.21 \times 10^3$         | -398                         | "                          | "                            |
| 48  | $7.90 \times 10^3$         | -197                         | "                          | $7.42 \times 10^3$           | -380                       | "                            | $7.32 \times 10^3$         | -480                         | "                          | "                            |
| 49  | $4.11 \times 10^3$         | -174                         | "                          | $3.28 \times 10^3$           | -328                       | "                            | $3.24 \times 10^3$         | -411                         | "                          | "                            |
| 50  | $6.99 \times 10^3$         | -181                         | "                          | $7.38 \times 10^3$           | -375                       | "                            | $7.32 \times 10^3$         | -480                         | "                          | "                            |
| 51  | $3.05 \times 10^3$         | -155                         | "                          | $3.80 \times 10^3$           | -331                       | "                            | $3.24 \times 10^3$         | -411                         | "                          | "                            |
| 52  | $7.41 \times 10^3$         | -192                         | "                          | $7.36 \times 10^3$           | -375                       | "                            | $7.32 \times 10^3$         | -480                         | "                          | "                            |
| 53  | $3.40 \times 10^3$         | -148                         | "                          | $3.92 \times 10^3$           | -380                       | "                            | $3.24 \times 10^3$         | -411                         | "                          | "                            |
| 54  | $7.10 \times 10^3$         | -189                         | "                          | $7.21 \times 10^3$           | -369                       | "                            | $7.01 \times 10^3$         | -478                         | "                          | "                            |
| 55  | $2.99 \times 10^3$         | -133                         | "                          | $3.56 \times 10^3$           | -345                       | "                            | $3.02 \times 10^3$         | -408                         | "                          | "                            |
| 56  | $5.84 \times 10^3$         | -170                         | "                          | $7.26 \times 10^3$           | -361                       | "                            | $7.01 \times 10^3$         | -478                         | "                          | "                            |
| 57  | $1.95 \times 10^3$         | -119                         | "                          | $3.21 \times 10^3$           | -353                       | "                            | $3.02 \times 10^3$         | -408                         | "                          | "                            |
| 58  | $6.65 \times 10^3$         | -179                         | "                          | $7.36 \times 10^3$           | -372                       | "                            | $7.01 \times 10^3$         | -478                         | "                          | "                            |
| 59  | $2.45 \times 10^3$         | -130                         | "                          | $3.25 \times 10^3$           | -350                       | "                            | $3.02 \times 10^3$         | -408                         | "                          | "                            |
| 60  | $18.6 \times 10^3$         | -283                         | "                          | $19.3 \times 10^3$           | -403                       | "                            | $18.2 \times 10^3$         | -613                         | "                          | "                            |
| 61  | $19.1 \times 10^3$         | -290                         | "                          | $18.6 \times 10^3$           | -410                       | "                            | $18.2 \times 10^3$         | -613                         | "                          | "                            |
| 62  | $1.66 \times 10^3$         | -105                         | "                          | $2.10 \times 10^3$           | -380                       | "                            | $2.06 \times 10^3$         | -487                         | "                          | "                            |
| 63  | $1.59 \times 10^3$         | -100                         | "                          | $2.24 \times 10^3$           | -383                       | "                            | $2.15 \times 10^3$         | -498                         | "                          | "                            |
| 64  | $1.76 \times 10^3$         | -109                         | "                          | $1.98 \times 10^3$           | -375                       | "                            | $1.92 \times 10^3$         | -478                         | "                          | "                            |

TABLE 14

| Nos | Example 1                  |                              | Carbonate-Free             |                              |                            |                              | Carbonate & Fluoride-Free  |                              |                            |                              |
|-----|----------------------------|------------------------------|----------------------------|------------------------------|----------------------------|------------------------------|----------------------------|------------------------------|----------------------------|------------------------------|
|     | Resistance value at 25° C. | Rate of Change in Resistance | Resistance value at 25° C. | Rate of Change in Resistance | Resistance value at 25° C. | Rate of Change in Resistance | Resistance value at 25° C. | Rate of Change in Resistance | Resistance value at 25° C. | Rate of Change in Resistance |
|     | R <sub>25</sub> (Ω)        | TCR (ppm/°C.)                | R <sub>25</sub> (Ω)        | TCR (ppm/°C.)                | R <sub>25</sub> (Ω)        | TCR (ppm/°C.)                | R <sub>25</sub> (Ω)        | TCR (ppm/°C.)                | R <sub>25</sub> (Ω)        | TCR (ppm/°C.)                |
| 1   | $83.6 \times 10^3$         | -300                         | $<\pm 2$                   | $87.5 \times 10^3$           | -493                       | $<\pm 2$                     | $84.3 \times 10^3$         | -989                         | $<\pm 2$                   | $<\pm 2$                     |
| 2   | $38.5 \times 10^3$         | -285                         | "                          | $41.5 \times 10^3$           | -423                       | "                            | $39.4 \times 10^3$         | -720                         | "                          | "                            |
| 3   | $19.8 \times 10^3$         | -120                         | "                          | $21.6 \times 10^3$           | -401                       | "                            | $20.4 \times 10^3$         | -378                         | "                          | "                            |
| 4   | $4.83 \times 10^3$         | +12                          | "                          | $4.92 \times 10^3$           | -263                       | "                            | $4.05 \times 10^3$         | -185                         | "                          | "                            |
| 5   | $38.7 \times 10^3$         | -214                         | "                          | $40.5 \times 10^3$           | -418                       | "                            | $39.2 \times 10^3$         | -723                         | "                          | "                            |
| 6   | $19.6 \times 10^3$         | -118                         | "                          | $21.4 \times 10^3$           | -409                       | "                            | $20.6 \times 10^3$         | -380                         | "                          | "                            |
| 7   | $52.5 \times 10^3$         | -298                         | "                          | $53.8 \times 10^3$           | -454                       | "                            | $53.2 \times 10^3$         | -830                         | "                          | "                            |
| 8   | $45.3 \times 10^3$         | -295                         | "                          | $46.5 \times 10^3$           | -438                       | "                            | $46.3 \times 10^3$         | -810                         | "                          | "                            |
| 9   | $48.7 \times 10^3$         | -267                         | "                          | $49.3 \times 10^3$           | -437                       | "                            | $49.1 \times 10^3$         | -812                         | "                          | "                            |
| 10  | $27.4 \times 10^3$         | -205                         | "                          | $28.9 \times 10^3$           | -407                       | "                            | $28.5 \times 10^3$         | -750                         | "                          | "                            |
| 11  | $33.0 \times 10^3$         | -198                         | "                          | $34.0 \times 10^3$           | -198                       | "                            | $33.8 \times 10^3$         | -780                         | "                          | "                            |
| 12  | $8.31 \times 10^3$         | +23                          | "                          | $9.60 \times 10^3$           | -283                       | "                            | $9.25 \times 10^3$         | -520                         | "                          | "                            |
| 13  | $7.20 \times 10^3$         | +31                          | "                          | $8.03 \times 10^3$           | -265                       | "                            | $7.80 \times 10^3$         | -490                         | "                          | "                            |
| 14  | $2.38 \times 10^3$         | +89                          | "                          | $3.08 \times 10^3$           | -250                       | "                            | $3.04 \times 10^3$         | -353                         | "                          | "                            |
| 15  | $59.6 \times 10^3$         | -289                         | "                          | $53.6 \times 10^3$           | -449                       | "                            | $53.2 \times 10^3$         | -830                         | "                          | "                            |
| 16  | $51.2 \times 10^3$         | -274                         | "                          | $46.8 \times 10^3$           | -424                       | "                            | $46.3 \times 10^3$         | -810                         | "                          | "                            |
| 17  | $57.7 \times 10^3$         | -283                         | "                          | $49.0 \times 10^3$           | -430                       | "                            | $49.1 \times 10^3$         | -812                         | "                          | "                            |
| 18  | $30.1 \times 10^3$         | -245                         | "                          | $29.1 \times 10^3$           | -380                       | "                            | $28.5 \times 10^3$         | -750                         | "                          | "                            |
| 19  | $35.2 \times 10^3$         | -201                         | "                          | $34.1 \times 10^3$           | -415                       | "                            | $33.8 \times 10^3$         | -780                         | "                          | "                            |
| 20  | $10.1 \times 10^3$         | -15                          | "                          | $9.34 \times 10^3$           | -350                       | "                            | $9.25 \times 10^3$         | -520                         | "                          | "                            |
| 21  | $9.08 \times 10^3$         | -50                          | "                          | $7.89 \times 10^3$           | -314                       | "                            | $7.80 \times 10^3$         | -490                         | "                          | "                            |
| 22  | $4.01 \times 10^3$         | +3                           | "                          | $3.21 \times 10^3$           | -289                       | "                            | $3.04 \times 10^3$         | -353                         | "                          | "                            |
| 23  | $54.9 \times 10^3$         | -283                         | "                          | $46.8 \times 10^3$           | -438                       | "                            | $46.3 \times 10^3$         | -830                         | "                          | "                            |
| 24  | $15.6 \times 10^3$         | -95                          | "                          | $9.36 \times 10^3$           | -352                       | "                            | $9.25 \times 10^3$         | -520                         | "                          | "                            |
| 25  | $32.7 \times 10^3$         | -254                         | "                          | $46.5 \times 10^3$           | -423                       | "                            | $46.3 \times 10^3$         | -810                         | "                          | "                            |

TABLE 14-continued

| Nos | Example 1                  |                              | Carbonate-Free             |                              |                            | Carbonate & Fluoride-Free    |                        |      |
|-----|----------------------------|------------------------------|----------------------------|------------------------------|----------------------------|------------------------------|------------------------|------|
|     | Resistance value at 25° C. | Rate of Change in Resistance | Resistance value at 25° C. | Rate of Change in Resistance | Resistance value at 25° C. | Rate of Change in Resistance |                        |      |
|     | R <sub>25</sub> (Ω)        | TCR (ppm/°C.)                | R <sub>25</sub> (Ω)        | TCR (ppm/°C.)                | R <sub>25</sub> (Ω)        | TCR (ppm/°C.)                |                        |      |
| 26  | 5.23 × 10 <sup>3</sup>     | -18                          | "                          | 9.30 × 10 <sup>3</sup>       | -273                       | "                            | 9.25 × 10 <sup>3</sup> | -520 |
| 27  | 47.4 × 10 <sup>3</sup>     | -270                         | "                          | 46.5 × 10 <sup>3</sup>       | -430                       | "                            | 46.3 × 10 <sup>3</sup> | -830 |
| 28  | 9.98 × 10 <sup>3</sup>     | -78                          | "                          | 9.31 × 10 <sup>3</sup>       | -360                       | "                            | 9.25 × 10 <sup>3</sup> | -520 |
| 29  | 47.3 × 10 <sup>3</sup>     | -272                         | "                          | 33.9 × 10 <sup>3</sup>       | -416                       | "                            | 33.8 × 10 <sup>3</sup> | -780 |
| 30  | 18.0 × 10 <sup>3</sup>     | -105                         | "                          | 9.35 × 10 <sup>3</sup>       | -370                       | "                            | 9.25 × 10 <sup>3</sup> | -520 |
| 31  | 35.2 × 10 <sup>3</sup>     | -187                         | "                          | 33.2 × 10 <sup>3</sup>       | -421                       | "                            | 33.8 × 10 <sup>3</sup> | -780 |
| 32  | 9.51 × 10 <sup>3</sup>     | -5                           | "                          | 8.93 × 10 <sup>3</sup>       | -320                       | "                            | 9.25 × 10 <sup>3</sup> | -520 |
| 33  | 37.0 × 10 <sup>3</sup>     | -201                         | "                          | 34.1 × 10 <sup>3</sup>       | -431                       | "                            | 33.8 × 10 <sup>3</sup> | -780 |
| 34  | 11.3 × 10 <sup>3</sup>     | -11                          | "                          | 9.25 × 10 <sup>3</sup>       | -368                       | "                            | 9.25 × 10 <sup>3</sup> | -520 |
| 35  | 46.8 × 10 <sup>3</sup>     | -300                         | "                          | 45.9 × 10 <sup>3</sup>       | -433                       | "                            | 46.3 × 10 <sup>3</sup> | -810 |
| 36  | 48.5 × 10 <sup>3</sup>     | -295                         | "                          | 46.4 × 10 <sup>3</sup>       | -430                       | "                            | 46.3 × 10 <sup>3</sup> | -810 |
| 37  | 43.3 × 10 <sup>3</sup>     | -280                         | "                          | 46.8 × 10 <sup>3</sup>       | -435                       | "                            | 46.3 × 10 <sup>3</sup> | -810 |
| 38  | 42.9 × 10 <sup>3</sup>     | -283                         | "                          | 45.8 × 10 <sup>3</sup>       | -429                       | "                            | 46.3 × 10 <sup>3</sup> | -810 |
| 39  | 67.1 × 10 <sup>3</sup>     | -299                         | "                          | 71.2 × 10 <sup>3</sup>       | -498                       | "                            | 70.1 × 10 <sup>3</sup> | -995 |
| 40  | 25.6 × 10 <sup>3</sup>     | -154                         | "                          | 29.3 × 10 <sup>3</sup>       | -408                       | "                            | 28.4 × 10 <sup>3</sup> | -788 |
| 41  | 16.8 × 10 <sup>3</sup>     | -121                         | "                          | 18.1 × 10 <sup>3</sup>       | -374                       | "                            | 17.7 × 10 <sup>3</sup> | -385 |
| 42  | 2.13 × 10 <sup>3</sup>     | -62                          | "                          | 3.21 × 10 <sup>3</sup>       | -270                       | "                            | 2.95 × 10 <sup>3</sup> | -207 |
| 43  | 27.1 × 10 <sup>3</sup>     | -156                         | "                          | 29.5 × 10 <sup>3</sup>       | -412                       | "                            | 28.2 × 10 <sup>3</sup> | -790 |
| 44  | 16.4 × 10 <sup>3</sup>     | -128                         | "                          | 18.4 × 10 <sup>3</sup>       | -368                       | "                            | 17.6 × 10 <sup>3</sup> | -381 |
| 45  | 45.5 × 10 <sup>3</sup>     | -284                         | "                          | 48.9 × 10 <sup>3</sup>       | -425                       | "                            | 48.6 × 10 <sup>3</sup> | -825 |
| 46  | 37.9 × 10 <sup>3</sup>     | -217                         | "                          | 39.0 × 10 <sup>3</sup>       | -416                       | "                            | 38.2 × 10 <sup>3</sup> | -810 |
| 47  | 41.5 × 10 <sup>3</sup>     | -254                         | "                          | 42.8 × 10 <sup>3</sup>       | -421                       | "                            | 42.1 × 10 <sup>3</sup> | -819 |
| 48  | 19.8 × 10 <sup>3</sup>     | -101                         | "                          | 20.8 × 10 <sup>3</sup>       | -382                       | "                            | 20.3 × 10 <sup>3</sup> | -780 |
| 49  | 25.5 × 10 <sup>3</sup>     | -137                         | "                          | 26.5 × 10 <sup>3</sup>       | -393                       | "                            | 26.3 × 10 <sup>3</sup> | -789 |
| 50  | 5.11 × 10 <sup>3</sup>     | -95                          | "                          | 6.23 × 10 <sup>3</sup>       | -283                       | "                            | 6.03 × 10 <sup>3</sup> | -310 |
| 51  | 4.78 × 10 <sup>3</sup>     | -73                          | "                          | 5.34 × 10 <sup>3</sup>       | -279                       | "                            | 5.05 × 10 <sup>3</sup> | -308 |
| 52  | 1.09 × 10 <sup>3</sup>     | -25                          | "                          | 2.10 × 10 <sup>3</sup>       | -268                       | "                            | 2.09 × 10 <sup>3</sup> | -280 |
| 53  | 6.95 × 10 <sup>3</sup>     | -105                         | "                          | 5.21 × 10 <sup>3</sup>       | -280                       | "                            | 5.05 × 10 <sup>3</sup> | -310 |
| 54  | 39.4 × 10 <sup>3</sup>     | -219                         | "                          | 38.4 × 10 <sup>3</sup>       | -420                       | "                            | 38.2 × 10 <sup>3</sup> | -815 |
| 55  | 38.1 × 10 <sup>3</sup>     | -183                         | "                          | 38.6 × 10 <sup>3</sup>       | -425                       | "                            | 38.2 × 10 <sup>3</sup> | -804 |
| 56  | 36.8 × 10 <sup>3</sup>     | -195                         | "                          | 37.9 × 10 <sup>3</sup>       | -418                       | "                            | 38.2 × 10 <sup>3</sup> | -809 |
| 57  | 26.5 × 10 <sup>3</sup>     | -295                         | "                          | 28.8 × 10 <sup>3</sup>       | -489                       | "                            | 27.1 × 10 <sup>3</sup> | -849 |
| 58  | 16.2 × 10 <sup>3</sup>     | -286                         | "                          | 18.2 × 10 <sup>3</sup>       | -465                       | "                            | 17.1 × 10 <sup>3</sup> | -452 |
| 59  | 6.81 × 10 <sup>3</sup>     | -267                         | "                          | 7.43 × 10 <sup>3</sup>       | -378                       | "                            | 7.34 × 10 <sup>3</sup> | -424 |
| 60  | 22.4 × 10 <sup>3</sup>     | -284                         | "                          | 24.8 × 10 <sup>3</sup>       | -412                       | "                            | 23.7 × 10 <sup>3</sup> | -784 |
| 61  | 13.8 × 10 <sup>3</sup>     | -253                         | "                          | 15.4 × 10 <sup>3</sup>       | -324                       | "                            | 14.6 × 10 <sup>3</sup> | -382 |
| 62  | 5.32 × 10 <sup>3</sup>     | -218                         | "                          | 5.92 × 10 <sup>3</sup>       | -295                       | "                            | 5.82 × 10 <sup>3</sup> | -316 |
| 63  | 41.6 × 10 <sup>3</sup>     | -254                         | "                          | 43.8 × 10 <sup>3</sup>       | -454                       | "                            | 42.5 × 10 <sup>3</sup> | -573 |
| 64  | 27.2 × 10 <sup>3</sup>     | -180                         | "                          | 29.6 × 10 <sup>3</sup>       | -398                       | "                            | 28.8 × 10 <sup>3</sup> | -375 |
| 65  | 9.53 × 10 <sup>3</sup>     | +88                          | "                          | 8.95 × 10 <sup>3</sup>       | -314                       | "                            | 9.82 × 10 <sup>3</sup> | -306 |
| 66  | 23.4 × 10 <sup>3</sup>     | -263                         | "                          | 25.3 × 10 <sup>3</sup>       | -263                       | "                            | 24.0 × 10 <sup>3</sup> | -501 |
| 67  | 14.1 × 10 <sup>3</sup>     | -201                         | "                          | 15.9 × 10 <sup>3</sup>       | -201                       | "                            | 15.4 × 10 <sup>3</sup> | -328 |
| 68  | 5.73 × 10 <sup>3</sup>     | -83                          | "                          | 6.25 × 10 <sup>3</sup>       | -254                       | "                            | 6.15 × 10 <sup>3</sup> | -287 |
| 69  | 24.1 × 10 <sup>3</sup>     | -526                         | "                          | 26.4 × 10 <sup>3</sup>       | -526                       | "                            | 25.7 × 10 <sup>3</sup> | -526 |
| 70  | 15.2 × 10 <sup>3</sup>     | -349                         | "                          | 15.2 × 10 <sup>3</sup>       | -349                       | "                            | 16.6 × 10 <sup>3</sup> | -349 |
| 71  | 6.69 × 10 <sup>3</sup>     | -104                         | "                          | 7.41 × 10 <sup>3</sup>       | -295                       | "                            | 7.32 × 10 <sup>3</sup> | -324 |
| 72  | 38.6 × 10 <sup>3</sup>     | -253                         | "                          | 40.3 × 10 <sup>3</sup>       | -418                       | "                            | 39.4 × 10 <sup>3</sup> | -485 |
| 73  | 27.5 × 10 <sup>3</sup>     | -180                         | "                          | 29.5 × 10 <sup>3</sup>       | -384                       | "                            | 28.4 × 10 <sup>3</sup> | -366 |
| 74  | 8.32 × 10 <sup>3</sup>     | +91                          | "                          | 9.14 × 10 <sup>3</sup>       | -214                       | "                            | 9.03 × 10 <sup>3</sup> | -343 |
| 75  | 30.4 × 10 <sup>3</sup>     | -284                         | "                          | 32.4 × 10 <sup>3</sup>       | -462                       | "                            | 31.0 × 10 <sup>3</sup> | -796 |
| 76  | 18.6 × 10 <sup>3</sup>     | -235                         | "                          | 20.5 × 10 <sup>3</sup>       | -390                       | "                            | 19.5 × 10 <sup>3</sup> | -391 |
| 77  | 7.71 × 10 <sup>3</sup>     | -203                         | "                          | 8.21 × 10 <sup>3</sup>       | -283                       | "                            | 8.64 × 10 <sup>3</sup> | -312 |
| 78  | 39.6 × 10 <sup>3</sup>     | -180                         | "                          | 41.6 × 10 <sup>3</sup>       | -254                       | "                            | 40.8 × 10 <sup>3</sup> | -299 |
| 79  | 31.5 × 10 <sup>3</sup>     | -174                         | "                          | 33.5 × 10 <sup>3</sup>       | -209                       | "                            | 32.2 × 10 <sup>3</sup> | -284 |
| 80  | 8.54 × 10 <sup>3</sup>     | +95                          | "                          | 9.15 × 10 <sup>3</sup>       | -196                       | "                            | 9.03 × 10 <sup>3</sup> | -254 |
| 81  | 33.4 × 10 <sup>3</sup>     | -263                         | "                          | 35.3 × 10 <sup>3</sup>       | -435                       | "                            | 34.3 × 10 <sup>3</sup> | -511 |
| 82  | 19.6 × 10 <sup>3</sup>     | -242                         | "                          | 21.9 × 10 <sup>3</sup>       | -353                       | "                            | 20.8 × 10 <sup>3</sup> | -360 |
| 83  | 7.51 × 10 <sup>3</sup>     | -195                         | "                          | 8.24 × 10 <sup>3</sup>       | -286                       | "                            | 8.20 × 10 <sup>3</sup> | -313 |
| 84  | 44.8 × 10 <sup>3</sup>     | -294                         | "                          | 46.8 × 10 <sup>3</sup>       | -463                       | "                            | 45.5 × 10 <sup>3</sup> | -775 |
| 85  | 32.8 × 10 <sup>3</sup>     | -281                         | "                          | 34.3 × 10 <sup>3</sup>       | -401                       | "                            | 33.1 × 10 <sup>3</sup> | -381 |
| 86  | 9.11 × 10 <sup>3</sup>     | -240                         | "                          | 9.8 × 10 <sup>3</sup>        | -2931                      | "                            | 10.3 × 10 <sup>3</sup> | -329 |
| 87  | 34.3 × 10 <sup>3</sup>     | -285                         | "                          | 36.5 × 10 <sup>3</sup>       | -459                       | "                            | 35.1 × 10 <sup>3</sup> | -769 |
| 88  | 24.5 × 10 <sup>3</sup>     | -239                         | "                          | 26.8 × 10 <sup>3</sup>       | -375                       | "                            | 25.4 × 10 <sup>3</sup> | -375 |
| 89  | 7.87 × 10 <sup>3</sup>     | -176                         | "                          | 8.14 × 10 <sup>3</sup>       | -275                       | "                            | 8.03 × 10 <sup>3</sup> | -352 |
| 90  | 28.4 × 10 <sup>3</sup>     | -287                         | "                          | 30.5 × 10 <sup>3</sup>       | -469                       | "                            | 29.6 × 10 <sup>3</sup> | -789 |
| 91  | 18.5 × 10 <sup>3</sup>     | -453                         | "                          | 20.9 × 10 <sup>3</sup>       | -353                       | "                            | 19.8 × 10 <sup>3</sup> | -384 |
| 92  | 5.43 × 10 <sup>3</sup>     | -224                         | "                          | 6.12 × 10 <sup>3</sup>       | -302                       | "                            | 6.25 × 10 <sup>3</sup> | -363 |
| 93  | 26.3 × 10 <sup>3</sup>     | -282                         | "                          | 28.6 × 10 <sup>3</sup>       | -434                       | "                            | 27.0 × 10 <sup>3</sup> | -600 |
| 94  | 15.2 × 10 <sup>3</sup>     | -253                         | "                          | 17.8 × 10 <sup>3</sup>       | -319                       | "                            | 16.4 × 10 <sup>3</sup> | -321 |
| 95  | 5.43 × 10 <sup>3</sup>     | -224                         | "                          | 5.58 × 10 <sup>3</sup>       | -264                       | "                            | 5.63 × 10 <sup>3</sup> | -302 |
| 96  | 28.3 × 10 <sup>3</sup>     | -186                         | "                          | 31.5 × 10 <sup>3</sup>       | -353                       | "                            | 18.4 × 10 <sup>3</sup> | -441 |
| 97  | 26.5 × 10 <sup>3</sup>     | -215                         | "                          | 24.6 × 10 <sup>3</sup>       | -321                       | "                            | 15.3 × 10 <sup>3</sup> | -425 |
| 98  | 32.8 × 10 <sup>3</sup>     | -255                         | "                          | 33.1 × 10 <sup>3</sup>       | -189                       | "                            | 29.5 × 10 <sup>3</sup> | -295 |
| 99  | 31.1 × 10 <sup>3</sup>     | -281                         | "                          | 30.5 × 10 <sup>3</sup>       | -340                       | "                            | 30.0 × 10 <sup>3</sup> | -518 |

TABLE 14-continued

| Nos | Example 1                  |                              |                            | Carbonate-Free      |               |                            | Carbonate & Fluoride-Free |               |                              |
|-----|----------------------------|------------------------------|----------------------------|---------------------|---------------|----------------------------|---------------------------|---------------|------------------------------|
|     | Resistance value at 25° C. | Rate of Change in Resistance | Resistance value at 25° C. | R <sub>25</sub> (Ω) | TCR (ppm/°C.) | Resistance value at 25° C. | R <sub>25</sub> (Ω)       | TCR (ppm/°C.) | Rate of Change in Resistance |
| 100 | $32.5 \times 10^3$         | -296                         | "                          | $31.1 \times 10^3$  | -290          | "                          | $23.4 \times 10^3$        | -399          | "                            |
| 101 | $7.35 \times 10^3$         | -58                          | "                          | $8.44 \times 10^3$  | -159          | "                          | $4.90 \times 10^3$        | -365          | "                            |
| 102 | $8.03 \times 10^3$         | -103                         | "                          | $8.33 \times 10^3$  | -353          | "                          | $4.62 \times 10^3$        | -521          | "                            |
| 103 | $9.46 \times 10^3$         | -59                          | "                          | $11.5 \times 10^3$  | -197          | "                          | $5.51 \times 10^3$        | -403          | "                            |
| 104 | $11.5 \times 10^3$         | -206                         | "                          | $13.0 \times 10^3$  | -395          | "                          | $7.70 \times 10^3$        | -530          | "                            |
| 105 | $7.48 \times 10^3$         | -251                         | "                          | $8.15 \times 10^3$  | -420          | "                          | $4.80 \times 10^3$        | -565          | "                            |

TABLE 15

| Nos | Example 1                  |                              |                            | Carbonate-Free      |               |                            | Carbonate & Fluoride-Free |               |                              |
|-----|----------------------------|------------------------------|----------------------------|---------------------|---------------|----------------------------|---------------------------|---------------|------------------------------|
|     | Resistance value at 25° C. | Rate of Change in Resistance | Resistance value at 25° C. | R <sub>25</sub> (Ω) | TCR (ppm/°C.) | Resistance value at 25° C. | R <sub>25</sub> (Ω)       | TCR (ppm/°C.) | Rate of Change in Resistance |
| 1   | $2.03 \times 10^3$         | +193                         | <±2                        | $3.01 \times 10^3$  | +304          | <±2                        | $2.87 \times 10^3$        | +307          | <±2                          |
| 2   | 923                        | +210                         | "                          | $1.53 \times 10^3$  | +318          | "                          | $1.09 \times 10^3$        | +395          | "                            |
| 3   | 710                        | +235                         | "                          | 811                 | +412          | "                          | 781                       | +480          | "                            |
| 4   | 493                        | +280                         | "                          | 583                 | +431          | "                          | 527                       | +545          | "                            |
| 5   | 963                        | +205                         | "                          | $1.23 \times 10^3$  | +320          | "                          | $1.05 \times 10^3$        | +400          | "                            |
| 6   | 720                        | +215                         | "                          | 803                 | +390          | "                          | 780                       | +475          | "                            |
| 7   | 893                        | +203                         | "                          | $1.99 \times 10^3$  | +315          | "                          | $1.96 \times 10^3$        | +348          | "                            |
| 8   | 818                        | +218                         | "                          | 556                 | +426          | "                          | 545                       | +529          | "                            |
| 9   | 625                        | +244                         | "                          | 701                 | +405          | "                          | 703                       | +503          | "                            |
| 10  | 631                        | +241                         | "                          | 707                 | +401          | "                          | 703                       | +503          | "                            |
| 11  | 321                        | +285                         | "                          | 572                 | +4161         | "                          | 566                       | +5141         | "                            |
| 12  | 218                        | +299                         | "                          | 503                 | +386          | "                          | 524                       | +541          | "                            |
| 13  | 595                        | +275                         | "                          | 701                 | +405          | "                          | 703                       | +503          | "                            |
| 14  | 308                        | +281                         | "                          | 572                 | +416          | "                          | 566                       | +514          | "                            |
| 15  | 583                        | +276                         | "                          | 701                 | +405          | "                          | 703                       | +503          | "                            |
| 16  | 300                        | +280                         | "                          | 572                 | +416          | "                          | 566                       | +514          | "                            |
| 17  | 610                        | +279                         | "                          | 701                 | +405          | "                          | 703                       | +503          | "                            |
| 18  | 318                        | +286                         | "                          | 572                 | +416          | "                          | 566                       | +514          | "                            |
| 19  | 925                        | +203                         | "                          | 580                 | +422          | "                          | 545                       | +529          | "                            |
| 20  | 781                        | +218                         | "                          | 699                 | +403          | "                          | 703                       | +503          | "                            |
| 21  | 785                        | +228                         | "                          | 571                 | +425          | "                          | 545                       | +529          | "                            |
| 22  | 523                        | +248                         | "                          | 678                 | +409          | "                          | 703                       | +503          | "                            |
| 23  | 712                        | +251                         | "                          | 559                 | +414          | "                          | 545                       | +529          | "                            |
| 24  | 455                        | +263                         | "                          | 650                 | +400          | "                          | 703                       | +503          | "                            |
| 25  | 585                        | +269                         | "                          | 685                 | +410          | "                          | 703                       | +503          | "                            |
| 26  | 564                        | +268                         | "                          | 671                 | +405          | "                          | 703                       | +503          | "                            |
| 27  | $5.85 \times 10^3$         | -298                         | "                          | $7.25 \times 10^3$  | -483          | "                          | $6.14 \times 10^3$        | -705          | "                            |
| 28  | $3.23 \times 10^3$         | -284                         | "                          | $4.26 \times 10^3$  | -448          | "                          | $3.88 \times 10^3$        | -509          | "                            |
| 29  | $1.84 \times 10^3$         | -283                         | "                          | $2.62 \times 10^3$  | -431          | "                          | $2.17 \times 10^3$        | -417          | "                            |
| 30  | 814                        | -163                         | "                          | 893                 | -285          | "                          | 866                       | -284          | "                            |
| 31  | $3.10 \times 10^3$         | -276                         | "                          | $4.21 \times 10^3$  | -451          | "                          | $3.90 \times 10^3$        | -515          | "                            |
| 32  | $1.94 \times 10^3$         | -284                         | "                          | $2.85 \times 10^3$  | -436          | "                          | $2.18 \times 10^3$        | -421          | "                            |
| 33  | $2.03 \times 10^3$         | -299                         | "                          | $5.07 \times 10^3$  | -452          | "                          | $5.14 \times 10^3$        | -618          | "                            |
| 34  | $1.86 \times 10^3$         | -286                         | "                          | $1.48 \times 10^3$  | -303          | "                          | $1.02 \times 10^3$        | -326          | "                            |
| 35  | $1.03 \times 10^3$         | -251                         | "                          | $1.52 \times 10^3$  | -301          | "                          | $1.50 \times 10^3$        | -347          | "                            |
| 36  | $1.02 \times 10^3$         | -233                         | "                          | $1.47 \times 10^3$  | -316          | "                          | $1.50 \times 10^3$        | -347          | "                            |
| 37  | 985                        | -185                         | "                          | $1.14 \times 10^3$  | -281          | "                          | $1.07 \times 10^3$        | -334          | "                            |
| 38  | 818                        | -135                         | "                          | 886                 | -251          | "                          | 9.02                      | -295          | "                            |
| 39  | $1.48 \times 10^3$         | -281                         | "                          | $1.52 \times 10^3$  | -301          | "                          | $1.50 \times 10^3$        | -347          | "                            |
| 40  | $1.25 \times 10^3$         | -220                         | "                          | $1.14 \times 10^3$  | -281          | "                          | $1.07 \times 10^3$        | -334          | "                            |
| 41  | $1.11 \times 10^3$         | -256                         | "                          | $1.52 \times 10^3$  | -301          | "                          | $1.50 \times 10^3$        | -347          | "                            |
| 42  | $1.03 \times 10^3$         | -188                         | "                          | $1.14 \times 10^3$  | -281          | "                          | $1.07 \times 10^3$        | -334          | "                            |
| 43  | $1.23 \times 10^3$         | -248                         | "                          | $1.52 \times 10^3$  | -301          | "                          | $1.50 \times 10^3$        | -347          | "                            |
| 44  | $1.09 \times 10^3$         | -195                         | "                          | $1.14 \times 10^3$  | -281          | "                          | $1.07 \times 10^3$        | -334          | "                            |
| 45  | $1.90 \times 10^3$         | -299                         | "                          | $1.55 \times 10^3$  | -314          | "                          | $1.02 \times 10^3$        | -326          | "                            |
| 46  | $2.54 \times 10^3$         | -273                         | "                          | $1.86 \times 10^3$  | -295          | "                          | $1.50 \times 10^3$        | -314          | "                            |
| 47  | $1.28 \times 10^3$         | -249                         | "                          | $1.35 \times 10^3$  | -288          | "                          | $1.02 \times 10^3$        | -326          | "                            |
| 48  | 980                        | -203                         | "                          | $1.38 \times 10^3$  | -256          | "                          | $1.50 \times 10^3$        | -341          | "                            |
| 49  | $2.05 \times 10^3$         | -285                         | "                          | $1.56 \times 10^3$  | -311          | "                          | $1.02 \times 10^3$        | -326          | "                            |
| 50  | $1.76 \times 10^3$         | -251                         | "                          | $1.67 \times 10^3$  | -285          | "                          | $1.50 \times 10^3$        | -341          | "                            |
| 51  | $1.24 \times 10^3$         | -240                         | "                          | $1.58 \times 10^3$  | -295          | "                          | $1.50 \times 10^3$        | -341          | "                            |
| 52  | $1.48 \times 10^3$         | -259                         | "                          | $1.55 \times 10^3$  | -336          | "                          | $1.50 \times 10^3$        | -341          | "                            |
| 53  | 703                        | +112                         | "                          | 884                 | +162          | "                          | 830                       | +261          | "                            |
| 54  | 625                        | +101                         | "                          | 878                 | +156          | "                          | 816                       | +258          | "                            |

TABLE 16

| NO | (Characteristic value corresponding to the sample in Table 8) |                              |                            |                              |                            |                              |
|----|---------------------------------------------------------------|------------------------------|----------------------------|------------------------------|----------------------------|------------------------------|
|    | Example 1                                                     |                              | Carbonate-Free             |                              | Carbonate & Fluoride-Free  |                              |
|    | Resistance value at 25° C.                                    | Rate of Change in Resistance | Resistance value at 25° C. | Rate of Change in Resistance | Resistance value at 25° C. | Rate of Change in Resistance |
|    | R <sub>25</sub> (Ω)                                           | TCR (ppm/°C.)                | R <sub>25</sub> (Ω)        | TCR (ppm/°C.)                | R <sub>25</sub> (Ω)        | TCR (ppm/°C.)                |
| 1  | $2.92 \times 10^3$                                            | +118                         | $<\pm 2$                   | $3.46 \times 10^3$           | +321                       | $<\pm 2$                     |
| 2  | $1.16 \times 10^3$                                            | +124                         | "                          | $2.03 \times 10^3$           | +403                       | "                            |
| 3  | 983                                                           | +159                         | "                          | $1.65 \times 10^3$           | +463                       | "                            |
| 4  | 786                                                           | +214                         | "                          | 892                          | +494                       | "                            |
| 5  | $2.98 \times 10^3$                                            | +120                         | "                          | $3.84 \times 10^3$           | +360                       | "                            |
| 6  | $1.26 \times 10^3$                                            | +123                         | "                          | $2.35 \times 10^3$           | +420                       | "                            |
| 7  | 965                                                           | +160                         | "                          | $2.14 \times 10^3$           | +430                       | "                            |
| 8  | 789                                                           | +223                         | "                          | 874                          | +490                       | "                            |
| 9  | 963                                                           | +163                         | "                          | $1.92 \times 10^3$           | +453                       | "                            |
| 10 | $1.03 \times 10^3$                                            | +123                         | "                          | $1.86 \times 10^3$           | +314                       | "                            |
| 11 | 925                                                           | +155                         | "                          | $1.02 \times 10^3$           | +368                       | "                            |
| 12 | 833                                                           | +202                         | "                          | 983                          | +480                       | "                            |
| 13 | 805                                                           | +248                         | "                          | 854                          | +475                       | "                            |
| 14 | 744                                                           | +249                         | "                          | 821                          | +485                       | "                            |
| 15 | 635                                                           | +255                         | "                          | 735                          | +492                       | "                            |
| 16 | $2.00 \times 10^3$                                            | +89                          | "                          | $1.96 \times 10^3$           | +303                       | "                            |
| 17 | $1.51 \times 10^3$                                            | +115                         | "                          | $1.82 \times 10^3$           | +343                       | "                            |
| 18 | $1.14 \times 10^3$                                            | +126                         | "                          | $1.72 \times 10^3$           | +392                       | "                            |
| 19 | $1.02 \times 10^3$                                            | +180                         | "                          | $1.68 \times 10^3$           | +403                       | "                            |
| 20 | 921                                                           | +205                         | "                          | 956                          | +424                       | "                            |
| 21 | 829                                                           | +238                         | "                          | 912                          | +490                       | "                            |
| 22 | $1.05 \times 10^3$                                            | +105                         | "                          | $1.12 \times 10^3$           | +390                       | "                            |
| 23 | 921                                                           | +150                         | "                          | 985                          | +436                       | "                            |
| 24 | 884                                                           | +136                         | "                          | 925                          | +453                       | "                            |
| 25 | 795                                                           | +181                         | "                          | 894                          | +483                       | "                            |
| 26 | 935                                                           | +161                         | "                          | 913                          | +409                       | "                            |
| 27 | 880                                                           | +180                         | "                          | 862                          | +490                       | "                            |
| 28 | 706                                                           | +223                         | "                          | 752                          | +493                       | "                            |
| 29 | 641                                                           | +244                         | "                          | 680                          | +496                       | "                            |
| 30 | 654                                                           | +249                         | "                          | 672                          | +495                       | "                            |
| 31 | 606                                                           | +250                         | "                          | 632                          | +480                       | "                            |
| 32 | 753                                                           | +195                         | "                          | 690                          | +476                       | "                            |
| 33 | 706                                                           | +203                         | "                          | 683                          | +481                       | "                            |
| 34 | $1.08 \times 10^3$                                            | +123                         | "                          | $1.12 \times 10^3$           | +373                       | "                            |
| 35 | $1.14 \times 10^3$                                            | +106                         | "                          | $1.14 \times 10^3$           | +359                       | "                            |
| 36 | 929                                                           | +192                         | "                          | 953                          | +393                       | "                            |
|    |                                                               |                              |                            |                              | 956                        | +634                         |

TABLE 17

| Nos | (Characteristic value corresponding to the sample in Table 9) |                              |                            |                              |                            |                              |
|-----|---------------------------------------------------------------|------------------------------|----------------------------|------------------------------|----------------------------|------------------------------|
|     | Example 1                                                     |                              | Carbonate-Free             |                              | Carbonate & Fluoride-Free  |                              |
|     | Resistance value at 25° C.                                    | Rate of Change in Resistance | Resistance value at 25° C. | Rate of Change in Resistance | Resistance value at 25° C. | Rate of Change in Resistance |
|     | R <sub>25</sub> (Ω)                                           | TCR (ppm/°C.)                | R <sub>25</sub> (Ω)        | TCR (ppm/°C.)                | R <sub>25</sub> (Ω)        | TCR (ppm/°C.)                |
| 1   | $9.07 \times 10^3$                                            | -276                         | $<\pm 2$                   | $9.56 \times 10^3$           | -483                       | $<\pm 2$                     |
| 2   | $20.2 \times 10^3$                                            | -278                         | "                          | $23.1 \times 10^3$           | -495                       | "                            |
| 3   | $16.5 \times 10^3$                                            | -289                         | "                          | $19.4 \times 10^3$           | -496                       | "                            |
| 4   | $2.45 \times 10^3$                                            | -216                         | "                          | $3.77 \times 10^3$           | -350                       | "                            |
| 5   | 825                                                           | +222                         | "                          | $1.01 \times 10^3$           | +362                       | "                            |
| 6   | $4.01 \times 10^3$                                            | -152                         | "                          | $4.22 \times 10^3$           | -249                       | "                            |
| 7   | $31.6 \times 10^3$                                            | -292                         | "                          | $34.0 \times 10^3$           | -486                       | "                            |
| 8   | $18.5 \times 10^3$                                            | -296                         | "                          | $24.1 \times 10^3$           | -493                       | "                            |
| 9   | $6.88 \times 10^3$                                            | -277                         | "                          | $8.03 \times 10^3$           | -446                       | "                            |
| 10  | $2.55 \times 10^3$                                            | -242                         | "                          | $3.96 \times 10^3$           | -387                       | "                            |
| 11  | $4.29 \times 10^3$                                            | -269                         | "                          | $4.93 \times 10^3$           | -477                       | "                            |
| 12  | $7.68 \times 10^3$                                            | -275                         | "                          | $8.95 \times 10^3$           | -467                       | "                            |
| 13  | $25.4 \times 10^3$                                            | -293                         | "                          | $29.4 \times 10^3$           | -480                       | "                            |
| 14  | $27.9 \times 10^3$                                            | -261                         | "                          | $34.9 \times 10^3$           | -417                       | "                            |
| 15  | $10.6 \times 10^3$                                            | -116                         | "                          | $16.9 \times 10^3$           | -290                       | "                            |
| 16  | $13.9 \times 10^3$                                            | -288                         | "                          | $14.7 \times 10^3$           | -491                       | "                            |
| 17  | $9.21 \times 10^3$                                            | -287                         | "                          | $11.9 \times 10^3$           | -465                       | "                            |
| 18  | $3.85 \times 10^3$                                            | -249                         | "                          | $4.95 \times 10^3$           | -425                       | "                            |
| 19  | $12.6 \times 10^3$                                            | -234                         | "                          | $16.6 \times 10^3$           | -392                       | "                            |
| 20  | $9.44 \times 10^3$                                            | -216                         | "                          | $14.3 \times 10^3$           | -401                       | "                            |
| 21  | 924                                                           | -169                         | "                          | $1.18 \times 10^3$           | -373                       | "                            |
| 22  | $8.05 \times 10^3$                                            | -264                         | "                          | $9.02 \times 10^3$           | -495                       | "                            |
| 23  | $4.02 \times 10^3$                                            | -250                         | "                          | $5.13 \times 10^3$           | -388                       | "                            |
| 24  | $1.21 \times 10^3$                                            | -234                         | "                          | $2.07 \times 10^3$           | -379                       | "                            |
| 25  | $5.09 \times 10^3$                                            | -262                         | "                          | $7.09 \times 10^3$           | -416                       | "                            |
| 26  | $5.49 \times 10^3$                                            | -270                         | "                          | $5.92 \times 10^3$           | -433                       | "                            |
|     |                                                               |                              |                            |                              | 5.84 $\times 10^3$         | -574                         |

TABLE 17-continued

| (Characteristic value corresponding to the sample in Table 9) |                                                |                                                       |                                                |                                                       |                                                |                                                |                    |      |   |
|---------------------------------------------------------------|------------------------------------------------|-------------------------------------------------------|------------------------------------------------|-------------------------------------------------------|------------------------------------------------|------------------------------------------------|--------------------|------|---|
| Example 1                                                     |                                                | Carbonate-Free                                        |                                                | Carbonate & Fluoride-Free                             |                                                |                                                |                    |      |   |
| Resis-<br>tance value<br>at 25° C.<br>R <sub>25</sub>         | Rate of<br>Change<br>in Resis-<br>tance<br>(%) | Resis-<br>tance value<br>at 25° C.<br>R <sub>25</sub> | Rate of<br>Change<br>in Resis-<br>tance<br>(%) | Resis-<br>tance value<br>at 25° C.<br>R <sub>25</sub> | Rate of<br>Change<br>in Resis-<br>tance<br>(%) | Rate of<br>Change<br>in Resis-<br>tance<br>(%) |                    |      |   |
| Nos (Ω)                                                       | (ppm/°C.)                                      |                                                       |                                                |                                                       |                                                |                                                |                    |      |   |
| 27                                                            | $18.4 \times 10^3$                             | -298                                                  | "                                              | $22.2 \times 10^3$                                    | -482                                           | "                                              | $20.5 \times 10^3$ | -865 | " |
| 28                                                            | $12.6 \times 10^3$                             | -186                                                  | "                                              | $15.6 \times 10^3$                                    | -316                                           | "                                              | $13.3 \times 10^3$ | -414 | " |
| 29                                                            | $4.11 \times 10^3$                             | -107                                                  | "                                              | $5.20 \times 10^3$                                    | -222                                           | "                                              | $4.46 \times 10^3$ | -295 | " |
| 30                                                            | $28.4 \times 10^3$                             | -284                                                  | "                                              | $36.3 \times 10^3$                                    | -492                                           | "                                              | $31.1 \times 10^3$ | -639 | " |
| 31                                                            | $16.0 \times 10^3$                             | -292                                                  | "                                              | $16.9 \times 10^3$                                    | -499                                           | "                                              | $16.5 \times 10^3$ | -821 | " |
| 32                                                            | 925                                            | -106                                                  | "                                              | 995                                                   | -232                                           | "                                              | 990                | -259 | " |
| 33                                                            | $7.96 \times 10^3$                             | -295                                                  | "                                              | $10.3 \times 10^3$                                    | -486                                           | "                                              | $8.24 \times 10^3$ | -795 | " |
| 34                                                            | $3.82 \times 10^3$                             | -264                                                  | "                                              | $5.28 \times 10^3$                                    | -378                                           | "                                              | $4.33 \times 10^3$ | -496 | " |
| 35                                                            | $1.02 \times 10^3$                             | +96                                                   | "                                              | $2.05 \times 10^3$                                    | +89                                            | "                                              | $1.14 \times 10^3$ | +125 | " |
| 36                                                            | 524                                            | +250                                                  | "                                              | 647                                                   | +370                                           | "                                              | 628                | +482 | " |
| 37                                                            | $36.0 \times 10^3$                             | -289                                                  | "                                              | $37.7 \times 10^3$                                    | -485                                           | "                                              | $36.3 \times 10^3$ | -992 | " |
| 38                                                            | $15.5 \times 10^3$                             | -275                                                  | "                                              | $19.0 \times 10^3$                                    | -466                                           | "                                              | $16.4 \times 10^3$ | -584 | " |
| 39                                                            | $8.00 \times 10^3$                             | -270                                                  | "                                              | $9.93 \times 10^3$                                    | -447                                           | "                                              | $8.14 \times 10^3$ | -534 | " |
| 40                                                            | $4.05 \times 10^3$                             | -206                                                  | "                                              | $6.01 \times 10^3$                                    | -250                                           | "                                              | $4.27 \times 10^3$ | -317 | " |
| 41                                                            | $5.09 \times 10^3$                             | -219                                                  | "                                              | $5.70 \times 10^3$                                    | -365                                           | "                                              | $5.45 \times 10^3$ | -487 | " |
| 42                                                            | $2.26 \times 10^3$                             | -244                                                  | "                                              | $3.07 \times 10^3$                                    | -430                                           | "                                              | $2.87 \times 10^3$ | -521 | " |
| 43                                                            | $12.0 \times 10^3$                             | -289                                                  | "                                              | $14.9 \times 10^3$                                    | -477                                           | "                                              | $12.4 \times 10^3$ | -855 | " |
| 44                                                            | $7.03 \times 10^3$                             | -294                                                  | "                                              | $10.2 \times 10^3$                                    | -411                                           | "                                              | $7.14 \times 10^3$ | -505 | " |
| 45                                                            | $5.49 \times 10^3$                             | -233                                                  | "                                              | $9.05 \times 10^3$                                    | -395                                           | "                                              | $6.23 \times 10^3$ | -480 | " |
| 46                                                            | 980                                            | +204                                                  | "                                              | $1.30 \times 10^3$                                    | +285                                           | "                                              | $1.19 \times 10^3$ | +329 | " |
| 47                                                            | $6.97 \times 10^3$                             | -288                                                  | "                                              | $9.66 \times 10^3$                                    | -483                                           | "                                              | $8.11 \times 10^3$ | -683 | " |
| 48                                                            | $2.79 \times 10^3$                             | -195                                                  | "                                              | $5.11 \times 10^3$                                    | -303                                           | "                                              | $3.18 \times 10^3$ | -359 | " |
| 49                                                            | $20.6 \times 10^3$                             | -289                                                  | "                                              | $24.7 \times 10^3$                                    | -480                                           | "                                              | $22.4 \times 10^3$ | -805 | " |
| 50                                                            | $15.4 \times 10^3$                             | -221                                                  | "                                              | $21.3 \times 10^3$                                    | -419                                           | "                                              | $17.7 \times 10^3$ | -551 | " |
| 51                                                            | $5.82 \times 10^3$                             | -125                                                  | "                                              | $7.10 \times 10^3$                                    | -344                                           | "                                              | $7.01 \times 10^3$ | -384 | " |
| 52                                                            | $4.02 \times 10^3$                             | -128                                                  | "                                              | $6.09 \times 10^3$                                    | -285                                           | "                                              | $4.98 \times 10^3$ | -399 | " |
| 53                                                            | $2.77 \times 10^3$                             | -105                                                  | "                                              | $4.95 \times 10^3$                                    | -216                                           | "                                              | $3.03 \times 10^3$ | -304 | " |
| 54                                                            | $5.29 \times 10^3$                             | -212                                                  | "                                              | $9.22 \times 10^3$                                    | -382                                           | "                                              | $6.18 \times 10^3$ | -454 | " |
| 55                                                            | $10.5 \times 10^3$                             | -277                                                  | "                                              | $15.6 \times 10^3$                                    | -495                                           | "                                              | $11.4 \times 10^3$ | -882 | " |
| 56                                                            | $3.00 \times 10^3$                             | -212                                                  | "                                              | $3.18 \times 10^3$                                    | -212                                           | "                                              | $3.05 \times 10^3$ | -309 | " |
| 57                                                            | $13.6 \times 10^3$                             | -266                                                  | "                                              | $16.2 \times 10^3$                                    | -423                                           | "                                              | $14.9 \times 10^3$ | -529 | " |
| 58                                                            | $11.2 \times 10^3$                             | -221                                                  | "                                              | $14.5 \times 10^3$                                    | -326                                           | "                                              | $13.4 \times 10^3$ | -418 | " |
| 59                                                            | $2.01 \times 10^3$                             | -106                                                  | "                                              | $4.22 \times 10^3$                                    | -210                                           | "                                              | $2.16 \times 10^3$ | -293 | " |
| 60                                                            | $3.12 \times 10^3$                             | -121                                                  | "                                              | $5.67 \times 10^3$                                    | -199                                           | "                                              | $3.39 \times 10^3$ | -305 | " |
| 61                                                            | $15.7 \times 10^3$                             | -296                                                  | "                                              | $16.9 \times 10^3$                                    | -491                                           | "                                              | $16.3 \times 10^3$ | -867 | " |
| 62                                                            | $10.7 \times 10^3$                             | -291                                                  | "                                              | $12.6 \times 10^3$                                    | -482                                           | "                                              | $11.0 \times 10^3$ | -797 | " |
| 63                                                            | $1.04 \times 10^3$                             | -200                                                  | "                                              | $2.09 \times 10^3$                                    | -275                                           | "                                              | $1.19 \times 10^3$ | -312 | " |
| 64                                                            | $2.55 \times 10^3$                             | -212                                                  | "                                              | $4.11 \times 10^3$                                    | -346                                           | "                                              | $2.76 \times 10^3$ | -425 | " |
| 65                                                            | $2.84 \times 10^3$                             | -209                                                  | "                                              | $5.71 \times 10^3$                                    | -315                                           | "                                              | $3.19 \times 10^3$ | -404 | " |
| 66                                                            | $21.9 \times 10^3$                             | -225                                                  | "                                              | $2.18 \times 10^3$                                    | -303                                           | "                                              | $2.05 \times 10^3$ | -377 | " |
| 67                                                            | $6.05 \times 10^3$                             | -234                                                  | "                                              | $24.9 \times 10^3$                                    | -473                                           | "                                              | $22.8 \times 10^3$ | -676 | " |
| 68                                                            | $5.79 \times 10^3$                             | -277                                                  | "                                              | $8.07 \times 10^3$                                    | -493                                           | "                                              | $6.39 \times 10^3$ | -820 | " |
| 69                                                            | $13.5 \times 10^3$                             | -280                                                  | "                                              | $18.8 \times 10^3$                                    | -469                                           | "                                              | $15.7 \times 10^3$ | -796 | " |
| 70                                                            | $10.1 \times 10^3$                             | -225                                                  | "                                              | $14.7 \times 10^3$                                    | -407                                           | "                                              | $11.6 \times 10^3$ | -491 | " |
| 71                                                            | $1.85 \times 10^3$                             | -174                                                  | "                                              | $2.41 \times 10^3$                                    | -312                                           | "                                              | $2.35 \times 10^3$ | -353 | " |
| 72                                                            | $94.8 \times 10^3$                             | -88                                                   | "                                              | $1.80 \times 10^3$                                    | -243                                           | "                                              | $1.07 \times 10^3$ | -307 | " |
| 73                                                            | $15.2 \times 10^3$                             | -285                                                  | "                                              | $20.3 \times 10^3$                                    | -469                                           | "                                              | $16.2 \times 10^3$ | -751 | " |
| 74                                                            | $17.9 \times 10^3$                             | -290                                                  | "                                              | $24.9 \times 10^3$                                    | -473                                           | "                                              | $20.5 \times 10^3$ | -787 | " |
| 75                                                            | $1.85 \times 10^3$                             | -192                                                  | "                                              | $4.85 \times 10^3$                                    | -315                                           | "                                              | $2.16 \times 10^3$ | -356 | " |
| 76                                                            | $1.44 \times 10^3$                             | +221                                                  | "                                              | $2.03 \times 10^3$                                    | +357                                           | "                                              | $1.99 \times 10^3$ | +420 | " |
| 77                                                            | $3.79 \times 10^3$                             | -236                                                  | "                                              | $5.96 \times 10^3$                                    | -405                                           | "                                              | $4.24 \times 10^3$ | -485 | " |
| 78                                                            | $7.00 \times 10^3$                             | -250                                                  | "                                              | $9.53 \times 10^3$                                    | -436                                           | "                                              | $7.14 \times 10^3$ | -652 | " |
| 79                                                            | $7.89 \times 10^3$                             | -262                                                  | "                                              | $10.2 \times 10^3$                                    | -449                                           | "                                              | $8.53 \times 10^3$ | -645 | " |
| 80                                                            | $13.4 \times 10^3$                             | -249                                                  | "                                              | $17.9 \times 10^3$                                    | -415                                           | "                                              | $15.3 \times 10^3$ | -577 | " |
| 81                                                            | $6.03 \times 10^3$                             | -260                                                  | "                                              | $6.33 \times 10^3$                                    | -382                                           | "                                              | $6.21 \times 10^3$ | -514 | " |
| 82                                                            | $3.09 \times 10^3$                             | -263                                                  | "                                              | $5.11 \times 10^3$                                    | -425                                           | "                                              | $4.02 \times 10^3$ | -520 | " |
| 83                                                            | $1.72 \times 10^3$                             | -187                                                  | "                                              | $4.07 \times 10^3$                                    | -249                                           | "                                              | $2.00 \times 10^3$ | -348 | " |
| 84                                                            | $3.85 \times 10^3$                             | -179                                                  | "                                              | $7.35 \times 10^3$                                    | -235                                           | "                                              | $4.11 \times 10^3$ | -380 | " |
| 85                                                            | $9.11 \times 10^3$                             | -296                                                  | "                                              | $14.5 \times 10^3$                                    | -489                                           | "                                              | $10.6 \times 10^3$ | -925 | " |
| 86                                                            | $6.04 \times 10^3$                             | -236                                                  | "                                              | $6.41 \times 10^3$                                    | -415                                           | "                                              | $6.22 \times 10^3$ | -545 | " |
| 87                                                            | $10.5 \times 10^3$                             | -277                                                  | "                                              | $14.2 \times 10^3$                                    | -495                                           | "                                              | $12.9 \times 10^3$ | -889 | " |
| 88                                                            | $17.7 \times 10^3$                             | -281                                                  | "                                              | $23.4 \times 10^3$                                    | -479                                           | "                                              | $19.5 \times 10^3$ | -826 | " |
| 89                                                            | $6.75 \times 10^3$                             | -267                                                  | "                                              | $10.7 \times 10^3$                                    | -452                                           | "                                              | $8.19 \times 10^3$ | -695 | " |
| 90                                                            | $2.29 \times 10^3$                             | -216                                                  | "                                              | $5.33 \times 10^3$                                    | -326                                           | "                                              | $3.14 \times 10^3$ | -459 | " |
| 91                                                            | $16.5 \times 10^3$                             | -241                                                  | "                                              | $17.9 \times 10^3$                                    | -473                                           | "                                              | $17.4 \times 10^3$ | -626 | " |
| 92                                                            | $15.6 \times 10^3$                             | -270                                                  | "                                              | $21.4 \times 10^3$                                    | -470                                           | "                                              | $18.6 \times 10^3$ | -893 | " |
| 93                                                            | $18.3 \times 10^3$                             | -281                                                  | "                                              | $24.0 \times 10^3$                                    | -475                                           | "                                              | $21.5 \times 10^3$ | -884 | " |
| 94                                                            | $15.4 \times 10^3$                             | -290                                                  | "                                              | $23.6 \times 10^3$                                    | -468                                           | "                                              | $19.9 \times 10^3$ | -834 | " |
| 95                                                            | $4.02 \times 10^3$                             | -287                                                  | "                                              | $7.12 \times 10^3$                                    | -356                                           | "                                              | $4.15 \times 10^3$ | -477 | " |
| 96                                                            | $1.89 \times 10^3$                             | -162                                                  | "                                              | $3.01 \times 10^3$                                    | -250                                           | "                                              | $2.90 \times 10^3$ | -299 | " |
| 97                                                            | $20.3 \times 10^3$                             | -273                                                  | "                                              | $24.7 \times 10^3$                                    | -493                                           | "                                              | $22.4 \times 10^3$ | -805 | " |
| 98                                                            | $10.1 \times 10^3$                             | -269                                                  | "                                              | $13.3 \times 10^3$                                    | -452                                           | "                                              | $11.5 \times 10^3$ | -603 | " |
| 99                                                            | $6.25 \times 10^3$                             | -216                                                  | "                                              | $9.69 \times 10^3$                                    | -395                                           | "                                              | $7.18 \times 10^3$ | -525 | " |
| 100                                                           | $3.80 \times 10^3$                             | -207                                                  | "                                              | $6.18 \times 10^3$                                    | -376                                           | "                                              | $3.87 \times 10^3$ | -489 | " |

TABLE 17-continued

| (Characteristic value corresponding to the sample in Table 9) |                              |                            |                              |                            |                              |
|---------------------------------------------------------------|------------------------------|----------------------------|------------------------------|----------------------------|------------------------------|
| Example 1                                                     |                              | Carbonate-Free             |                              | Carbonate & Fluoride-Free  |                              |
| Resistance value at 25° C.                                    | Rate of Change in Resistance | Resistance value at 25° C. | Rate of Change in Resistance | Resistance value at 25° C. | Rate of Change in Resistance |
| R <sub>25</sub><br>Nos (Ω)                                    | TCR<br>(ppm/°C.)             | R <sub>25</sub><br>(Ω)     | TCR<br>(ppm/°C.)             | R <sub>25</sub><br>(Ω)     | TCR<br>(ppm/°C.)             |
| 101 $1.15 \times 10^3$                                        | -149                         | "                          | $1.82 \times 10^3$           | -288                       | "                            |
| 102 $12.8 \times 10^3$                                        | -280                         | "                          | $16.7 \times 10^3$           | -481                       | "                            |
| 103 $18.3 \times 10^3$                                        | -226                         | "                          | $23.0 \times 10^3$           | -432                       | "                            |
| 104 $21.4 \times 10^3$                                        | -280                         | "                          | $29.2 \times 10^3$           | -476                       | "                            |
| 105 $7.03 \times 10^3$                                        | -216                         | "                          | $12.6 \times 10^3$           | -358                       | "                            |
| 106 969                                                       | +70                          | "                          | 992                          | +148                       | "                            |
| 107 $3.00 \times 10^3$                                        | -201                         | "                          | $3.56 \times 10^3$           | -388                       | "                            |
| 108 $4.17 \times 10^3$                                        | -212                         | "                          | $7.23 \times 10^3$           | -365                       | "                            |
| 109 $5.84 \times 10^3$                                        | -182                         | "                          | $9.44 \times 10^3$           | -250                       | "                            |
| 110 $5.99 \times 10^3$                                        | -209                         | "                          | $10.1 \times 10^3$           | -371                       | "                            |
| 111 $7.03 \times 10^3$                                        | -220                         | "                          | $7.51 \times 10^3$           | -428                       | "                            |
| 112 $9.76 \times 10^3$                                        | -254                         | "                          | $13.4 \times 10^3$           | -452                       | "                            |
| 113 $4.01 \times 10^3$                                        | -172                         | "                          | $6.33 \times 10^3$           | -333                       | "                            |
| 114 $4.70 \times 10^3$                                        | -225                         | "                          | $6.49 \times 10^3$           | -329                       | "                            |
| 115 $9.54 \times 10^3$                                        | -185                         | "                          | $15.4 \times 10^3$           | -376                       | "                            |
| 116 $9.09 \times 10^3$                                        | -196                         | "                          | $9.29 \times 10^3$           | -395                       | "                            |
| 117 $6.19 \times 10^3$                                        | -200                         | "                          | $8.81 \times 10^3$           | -400                       | "                            |
| 118 $6.25 \times 10^3$                                        | -225                         | "                          | $9.24 \times 10^3$           | -416                       | "                            |
| 119 $5.87 \times 10^3$                                        | -230                         | "                          | $10.1 \times 10^3$           | -420                       | "                            |
| 120 $5.14 \times 10^3$                                        | -209                         | "                          | $9.91 \times 10^3$           | -405                       | "                            |
|                                                               |                              |                            |                              | $5.89 \times 10^3$         | -509                         |

## EXAMPLE 2

In accordance with Example 1, multilayered ceramic substrates were prepared, except that the molybdates, fluorides and glass powders having the compositions 30 specified in Table 18 were used without any heat treatment, and their R<sub>25</sub>, TCR and rate of changes in resistance were measured. The results are indicated in Table 19 with the corresponding sample numbers.

TABLE 18

| NOs | Molybdate<br>(wt. %)                                   | Composition |         |                      |                  |                  |                       |                   |                   |
|-----|--------------------------------------------------------|-------------|---------|----------------------|------------------|------------------|-----------------------|-------------------|-------------------|
|     |                                                        | Glass<br>B  |         | Fluorides<br>(wt. %) |                  |                  | Carbonates<br>(wt. %) |                   |                   |
|     |                                                        | (wt. %)     | (wt. %) | SrF <sub>2</sub>     | BaF <sub>2</sub> | MgF <sub>2</sub> | CaF <sub>2</sub>      | SrCO <sub>3</sub> | BaCO <sub>3</sub> |
| 1   | MgMoO <sub>4</sub>                                     | 40          | 59      |                      |                  |                  | 0.5                   |                   | 0.5               |
| 2   | CaMoO <sub>4</sub>                                     | 40          | 59      | 0.5                  |                  |                  |                       |                   | 0.5               |
| 3   | SrMoO <sub>4</sub>                                     | 40          | 59      |                      |                  |                  | 0.5                   | 0.5               |                   |
| 4   | BaMoO <sub>4</sub>                                     | 40          | 59      |                      | 0.5              |                  |                       |                   | 0.5               |
| 5   | (Mg <sub>0.3</sub> Ca <sub>0.7</sub> )MoO <sub>4</sub> | 60          | 20      | 10                   |                  |                  |                       |                   | 10                |
| 6   | MgMoO <sub>4</sub>                                     | 30          | 20      |                      |                  | 10               | 10                    |                   |                   |
|     | Ca <sub>3</sub> MoO <sub>6</sub>                       | 30          |         |                      |                  |                  |                       |                   |                   |
| 7   | ZnMoO <sub>4</sub>                                     | 65          | 34      |                      |                  | 0.5              |                       |                   | 0.5               |
| 8   | Al <sub>2</sub> Mo <sub>3</sub> O <sub>12</sub>        | 60          | 39      |                      | 0.5              |                  | 0.5                   |                   |                   |
| 9   | ZrMo <sub>2</sub> O <sub>8</sub>                       | 45          | 54      | 0.5                  |                  |                  |                       | 0.5               |                   |
| 10  | HfMo <sub>2</sub> O <sub>8</sub>                       | 45          | 54      |                      |                  | 0.5              | 0.5                   |                   |                   |
| 11  | Y <sub>6</sub> MoO <sub>12</sub>                       | 80          | 5       | 7.5                  |                  |                  |                       |                   | 7.5               |
| 12  | La <sub>6</sub> MoO <sub>12</sub>                      | 80          | 5       | 7.5                  |                  |                  |                       |                   | 7.5               |
| 13  | Ce <sub>6</sub> MoO <sub>12</sub>                      | 80          | 5       | 7.5                  |                  |                  |                       |                   | 7.5               |
| 14  | Pr <sub>6</sub> MoO <sub>12</sub>                      | 80          | 5       | 7.5                  |                  |                  |                       |                   | 7.5               |
| 15  | Nd <sub>6</sub> MoO <sub>12</sub>                      | 80          | 5       | 7.5                  |                  |                  |                       |                   | 7.5               |
| 16  | Sm <sub>6</sub> MoO <sub>12</sub>                      | 80          | 5       | 7.5                  |                  |                  |                       |                   | 7.5               |
| 17  | Eu <sub>6</sub> MoO <sub>12</sub>                      | 80          | 5       | 7.5                  |                  |                  |                       |                   | 7.5               |
| 18  | Gd <sub>6</sub> MoO <sub>12</sub>                      | 80          | 5       | 7.5                  |                  |                  |                       |                   | 7.5               |
| 19  | Tb <sub>6</sub> MoO <sub>12</sub>                      | 80          | 5       | 7.5                  |                  |                  |                       |                   | 7.5               |
| 20  | Dy <sub>6</sub> MoO <sub>12</sub>                      | 80          | 5       | 7.5                  |                  |                  |                       |                   | 7.5               |
| 21  | Ho <sub>6</sub> MoO <sub>12</sub>                      | 80          | 5       | 7.5                  |                  |                  |                       |                   | 7.5               |
| 22  | Erg <sub>6</sub> MoO <sub>12</sub>                     | 80          | 5       | 7.5                  |                  |                  |                       |                   | 7.5               |
| 23  | Tm <sub>6</sub> MoO <sub>12</sub>                      | 80          | 5       | 7.5                  |                  |                  |                       |                   | 7.5               |
| 24  | Yb <sub>6</sub> MoO <sub>12</sub>                      | 80          | 5       | 7.5                  |                  |                  |                       |                   | 7.5               |
| 25  | Lu <sub>6</sub> MoO <sub>12</sub>                      | 80          | 5       | 7.5                  |                  |                  |                       |                   | 7.5               |
| 26  | Nb <sub>6</sub> Mo <sub>3</sub> O <sub>14</sub>        | 55          | 44      |                      | 0.5              |                  |                       | 0.5               |                   |
| 27  | Ta <sub>2</sub> Mo <sub>3</sub> O <sub>14</sub>        | 55          | 44      |                      |                  | 0.5              | 0.5                   |                   |                   |
| 28  | MnMoO <sub>4</sub>                                     | 65          | 34      |                      |                  | 0.5              | 0.5                   |                   |                   |

TABLE 19

| Nos | Example 2                  |                                  |                            | Fluoride Free              |               |                                  |
|-----|----------------------------|----------------------------------|----------------------------|----------------------------|---------------|----------------------------------|
|     | Resistance value at 25° C. | Rate of Change in Resistance (%) | Resistance value at 25° C. | Resistance value at 25° C. | TCR (ppm/°C.) | Rate of Change in Resistance (%) |
|     | R <sub>25</sub> (Ω)        | TCR (ppm/°C.)                    | R <sub>25</sub> (Ω)        | R <sub>25</sub> (Ω)        | (ppm/°C.)     | (%)                              |
| 1   | $3.04 \times 10^3$         | -1316                            | $<\pm 2$                   | $4.35 \times 10^3$         | -1356         | $<\pm 2$                         |
| 2   | $29.8 \times 10^3$         | -1435                            | "                          | $35.2 \times 10^3$         | -1483         | "                                |
| 3   | 674                        | -1385                            | "                          | 823                        | -1411         | "                                |
| 4   | 388                        | +1156                            | "                          | 524                        | +1192         | "                                |
| 5   | $8.44 \times 10^3$         | -1384                            | "                          | $9.83 \times 10^3$         | -1401         | "                                |
| 6   | $6.24 \times 10^3$         | -1309                            | "                          | $7.29 \times 10^3$         | -1328         | "                                |
| 7   | $4.80 \times 10^3$         | -1370                            | "                          | $5.63 \times 10^3$         | -1412         | "                                |
| 8   | $11.6 \times 10^3$         | -1462                            | "                          | $12.5 \times 10^3$         | -1489         | "                                |
| 9   | $17.4 \times 10^3$         | -1615                            | "                          | $18.9 \times 10^3$         | -1676         | "                                |
| 10  | $15.4 \times 10^3$         | -1468                            | "                          | $16.2 \times 10^3$         | +1498         | "                                |
| 11  | $5.95 \times 10^3$         | -1216                            | "                          | $6.82 \times 10^3$         | -1273         | "                                |
| 12  | $5.03 \times 10^3$         | -1206                            | "                          | $6.23 \times 10^3$         | -1256         | "                                |
| 13  | $3.95 \times 10^3$         | -1195                            | "                          | $4.36 \times 10^3$         | +1232         | "                                |
| 14  | $3.88 \times 10^3$         | -1192                            | "                          | $4.21 \times 10^3$         | -1213         | "                                |
| 15  | $4.99 \times 10^3$         | -1312                            | "                          | $5.36 \times 10^3$         | -1363         | "                                |
| 19  | $7.18 \times 10^3$         | -1269                            | "                          | $8.05 \times 10^3$         | -1272         | "                                |
| 20  | $7.33 \times 10^3$         | -1050                            | "                          | $8.65 \times 10^3$         | -1080         | "                                |
| 21  | $7.18 \times 10^3$         | -1182                            | "                          | $8.23 \times 10^3$         | -1210         | "                                |
| 22  | $7.85 \times 10^3$         | -1324                            | "                          | $8.41 \times 10^3$         | -1363         | "                                |
| 23  | $6.94 \times 10^3$         | -1306                            | "                          | $7.81 \times 10^3$         | +1353         | "                                |
| 24  | $6.03 \times 10^3$         | -1244                            | "                          | $7.03 \times 10^3$         | -1286         | "                                |
| 25  | $4.67 \times 10^3$         | -1195                            | "                          | $5.63 \times 10^3$         | -1215         | "                                |
| 26  | 625                        | +1059                            | "                          | 725                        | +1080         | "                                |
| 27  | $1.45 \times 10^3$         | -1345                            | "                          | $2.03 \times 10^3$         | -1376         | "                                |
| 28  | 905                        | +1230                            | "                          | $1.06 \times 10^3$         | -1271         | "                                |

## COMPARISON EXAMPLE 1

MoSi<sub>2</sub>-TaSi<sub>2</sub> Glass Base Resistor Material

A mixture of 16 parts by weight of MoSi<sub>2</sub> with 9 parts by weight of TaSi<sub>2</sub> was heated at 1400° C. in vacuum. The resulting product was pulverized together with ethanol by alumina balls in a pot mill for 24 hours, and was dried to obtain fine powders having a particle size of 10  $\mu\text{m}$  or lower. Seventy five (75) parts by weight of glass frit consisting of BaO, B<sub>2</sub>O<sub>3</sub>, MgO, CaO and SiO<sub>2</sub> and 25 parts by weight of the organic vehicle (20 parts by weight of butyl carbitol plus 5 parts by weight of ethyl cellulose) were added to 25 parts by weight of the thus obtained fine powders, and were roll-milled to obtain a resistive paste.

Except that this resistive paste was used, a multilayered ceramic board was obtained in the same manner as in the foregoing examples.

As a result, the product obtained by forming the resistive film produced from said paste on a ceramic green sheet, heat-treating them for the decomposition of the organics and, thereafter, simultaneously sintering them could not be put to practical use, since it warped due to differences in the coefficients of expansion and shrinkage between both the sintered bodies, as illustrated in FIG. 4, and swelled due to the evolution of a gas by the decomposing reaction of MoSi<sub>2</sub> and TaSi<sub>2</sub>, as illustrated in FIG. 5. It is to be noted that 11a, 14a and 13a are a layer corresponding to the aforesaid layer 1a, a layer corresponding to the aforesaid layer 4a and a thick-film resistor corresponding to the aforesaid thick-film resistor 3a, respectively.

## COMPARISON EXAMPLE 2

MoSi<sub>2</sub>-BaF<sub>2</sub> Glass Base Resistor Material

Seventy (70) parts by weight of MoSi<sub>2</sub> and 20 parts by weight of BaF<sub>2</sub> were mixed with 10 parts by weight of glass frit comprising SiO<sub>2</sub>, ZnO, ZrO<sub>2</sub>, CaO and Al<sub>2</sub>O<sub>3</sub>

35 by ball-milling, and the resulting powders were heat-treated at 1200° C. in an argon (Ar) gas atmosphere. Thereafter, the product was pulverized together with ethanol for 24 hours by alumina balls in a pot mill, and was dried to obtain fine powders having a particle size of 10  $\mu\text{m}$  or lower.

40 Except that this resistive paste was used, a multilayered ceramic board was obtained in the same manner as in Example 1. Shown in Table 20 are the results of the R<sub>25</sub>, TCR and rate of change in resistance value of the thick-film resistor of the multilayered ceramic substrate, 45 which were measured in the same manner as in Example 1.

TABLE 20

| 50 | Resistance Value R <sub>25</sub> at 25° C., Ohms | TCR ppm/°C. | Rate of Change in Resistance Value, % |
|----|--------------------------------------------------|-------------|---------------------------------------|
|    | Comp. Ex. 2                                      | 124.5       | +1120                                 |
|    |                                                  |             | 9.7% increase                         |

55 From the above results, it has been found that the multilayered ceramic boards according to the examples all undergo neither warping nor swelling, and their rate of change in resistance value is within  $\pm 2\%$ , and that, in particular, the TCR of those having the resistor material heat-treated does not exceed  $\pm 500$  ppm/°C. in the 60 case where the fluorides of alkaline earth metals are used and  $\pm 300$  ppm/°C. in the case where the carbonates of alkaline earth metals are used. It has been noted, on the other hand, that the multilayered ceramic board of Comp. Ex. 1 undergoes warping, whereas the multilayered ceramic board of Comp. Ex. 2 has its resistor showing a rate of change in resistance value that is four times higher and a TCR that is one order of magnitude higher.

## EFFECTS OF THE INVENTION

According to the present invention, there can be provided a sintered body containing at least one molybdate selected from at least one molybdate group selected from the groups (A) to (G) defined in the foregoing, with or without the fluoride of an alkaline earth metal, and an electrical resistor paste containing a resistive material for said sintered body and the carbonate of an alkaline earth metal. Accordingly, if the resistor material or paste for this sintered body is used and sintered along with a conductor material based on, e.g., a base metal and a ceramic green sheet in a nonoxidizing atmosphere to form a resistor, it is very unlikely that the sintered body may either warp or swell due to sintering. It is further possible not only to decrease a change-with-time of the resistance value esp. at a high humidity but also to reduce the temperature dependence coefficient of the resistance value of the resistor not to exceed  $\pm 300$  ppm/ $^{\circ}\text{C}$ ., for instance.

Hence, it is possible to meet both the demands for reductions in the size and cost of circuit boards having resistors incorporated thereinto and to provide excellent electronic parts to electronic equipment needing precise work.

Further, if the molybdate belonging to the aforesaid groups (A) to (G), preferably with the fluoride of an alkaline earth metal are heat-treated with glass, it is then possible to decrease the absolute value of the temperature dependent coefficient of the resistor and add excellent capabilities to electronic circuits needing precise performance, compared with the case where such any heat-treatment is not carried out.

What is claimed is:

1. An electrical resistor comprising a sintered body containing 30 to 96% by weight of at least one molybdate selected from the group consisting of (A) to (G) and 4 to 70% by weight of glass;

(A) Molybdates of alkaline earth metals,

(B) Molybdates of zinc,

(C) Molybdates of elements Y, La, Ce, Pr, Nd, Sm, Eu, Gd, Tb, Dy, Ho, Er, Tm, Yb and Lu, and complex molybdates of two or more of said elements,

(D) Molybdates of aluminum

(E) Molybdates of elements zirconium and hafnium, and complex molybdates thereof,

(F) Molybdates of elements niobium and tantalum, and complex molybdates thereof, and

(G) Molybdates of manganese.

2. An electrical resistor as defined in claim 1, wherein said at least one molybdate group selected from said groups (A) to (G) is two or more groups.

3. An electrical resistor as defined in claim 1 or 2, wherein said sintered body is obtained by the step of sintering at 800° to 1100° C. a resistor material containing 30 to 96% by weight, calculated as molybdate, of at least one of the corresponding molybdates selected from the group consisting of the aforesaid groups (A) to (G) and their precursors and 4 to 70% by weight of glass;

wherein said precursors comprise a molybdenum compound that is converted to a molybdate by heat treatment and compounds of the elements of said groups (A) to (G).

4. An electrical resistor comprising a sintered body containing 30 to 95% by weight of at least one molybdate selected from the following groups (A) to (G), 4.5

to 69.5% by weight of glass and 0.5 to 40% by weight of a fluoride of an alkaline earth metal;

(A) Molybdates of alkaline earth metals,

(B) Molybdates of zinc,

(C) Molybdates of elements Y, La, Ce, Pr, Nd, Sm, Eu, Gd, Tb, Dy, Ho, Er, Tm, Yb and Lu, and complex molybdates of two or more of said elements,

(D) Molybdates of aluminum

(E) Molybdates of elements zirconium and hafnium, and complex molybdates thereof,

(F) Molybdates of elements niobium and tantalum, and complex molybdates thereof, and

(G) Molybdates of manganese.

5. An electrical resistor as defined in claim 4, wherein said at least one molybdate group selected from said groups (A) to (G) is two or more groups.

6. An electrical resistor as defined in claim 4 or 5, wherein said sintered body is obtained by the step of sintering at 800° to 1100° C. a resistor material containing 30 to 95% by weight, calculated as molybdate, of at least one of the corresponding molybdates selected from the group consisting of the aforesaid groups (A) to (G) and their precursors, 4.5 to 69.5% by weight of glass and 0.5 to 40% by weight of a fluoride of an alkaline earth metal;

wherein said precursors comprise a molybdenum compound that is converted to a molybdate by heat treatment and compounds of the elements of said groups (A) to (G).

7. An electrical resistor paste comprising 40 to 95% by weight of at least one molybdate group selected from the group consisting of (A) to (G), 4 to 59% by weight of glass, 0.5 to 25% by weight of a fluoride of an alkaline earth metal and 0.5 to 50% by weight of a carbonate of an alkaline earth metal;

(A) Molybdates of alkaline earth metals and precursors thereof,

(B) Molybdates of zinc and precursors thereof,

(C) Molybdates of elements Y, La, Ce, Pr, Nd, Sm, Eu, Gd, Tb, Dy, Ho, Er, Tm, Yb and Lu, and complex molybdates of two or more of said elements and precursors thereof,

(D) Molybdates of aluminum and precursors thereof

(E) Molybdates of elements zirconium and hafnium, and complex molybdates thereof and precursors thereof,

(F) Molybdates of elements niobium and tantalum, and complex molybdates thereof and precursors thereof, and

(G) Molybdates of manganese and precursors thereof;

wherein said precursors comprise a molybdenum compound that is converted to a molybdate by heat treatment and compounds of the elements of said groups (A) to (G), respectively.

8. An electrical resistor paste as defined in claim 7, wherein said at least one molybdate group selected from said groups (A) to (G) is two or more groups.

9. An electrical resistor paste comprising 34.8 to 95% by weight of at least one molybdate selected from the group consisting of (A) to (G) and their precursors, 0.3 to 29.9% by weight of a fluoride of an alkaline earth metal, 0.3 to 33.3% by weight of a carbonate of an alkaline earth metal and 2.1 to 49.5% by weight of glass

(A) Molybdates of alkaline earth metals,

(B) Molybdates of zinc,

(C) Molybdates of elements Y, La, Ce, Pr, Nd, Sm, Eu, Gd, Tb, Dy, Ho, Er, Tm, Yb and Lu, and complex molybdates of two or more of said elements,

(D) Molybdates of aluminum

(E) Molybdates of elements zirconium and hafnium, and complex molybdates thereof,

(F) Molybdates of elements niobium and tantalum, and complex molybdates thereof, and

(G) Molybdates of manganese;

wherein said precursors comprise a molybdenum compound that is converted to a molybdate by heat treatment and compounds of the elements of said groups (A) to (G).

10. An electrical resistor which is a sintered body comprising bulk particles, acicular particles deposited onto said bulk particles and a glass layer, said bulk particles comprising at least one molybdate selected from the group consisting of (A) to (G), and said acicular particles comprising a reduction product of said molybdate;

(A) Molybdates of alkaline earth metals,

(B) Molybdates of zinc,

(C) Molybdates of elements Y, La, Ce, Pr, Nd, Sm, Eu, Gd, Tb, Dy, Ho, Er, Tm, Yb and Lu, and complex molybdates of two or more of said elements,

(D) Molybdates of aluminum

(E) Molybdates of elements zirconium and hafnium, and complex molybdates thereof,

(F) Molybdates of elements niobium and tantalum, and complex molybdates thereof, and

(G) Molybdates of manganese.

11. An electrical resistor as defined in claim 10, wherein said bulk and acicular particles are obtained by the step of sintering at 800° to 1100° C. a resistor material comprising at least one of the molybdates selected from the group consisting of (A) to (G) and their precursors;

wherein said precursors comprise a molybdenum compound that is converted to a molybdate by heat treatment and compounds of the elements of said groups (A) to (G).

12. An electrical resistor as defined in claim 10 or 11, wherein said acicular particles are a product obtained by the reduction of the surfaces of said bulk particles.

13. An electrical resistor paste comprising bulk particles containing 40 to 95% by weight of at least one molybdate group selected from the group consisting of (A) to (G), 0.5 to 25% by weight of a fluoride of an alkaline earth metal, 0.5 to 50% by weight of a carbonate of an alkaline earth metal and 4 to 59% by weight of a glass, and in which the surfaces of said bulk particles are reduced to form acicular particles by sintering at 800° to 1100° C. at least the non-combustible portion of the non-volatile matter thereof in a non-oxidizing atmosphere, thereby obtaining a sintered body in which said acicular particles are deposited onto said bulk particles,

(A) Molybdates of alkaline earth metals and precursors thereof,

(B) Molybdates of zinc and precursors thereof,

(C) Molybdates of elements Y, La, Ce, Pr, Nd, Sm, Eu, Gd, Tb, Dy, Ho, Er, Tm, Yb and Lu, and

complex molybdates of two or more of said elements and precursors thereof,

(D) Molybdates of aluminum and precursors thereof

(E) Molybdates of elements zirconium and hafnium, and complex molybdates thereof and precursors thereof,

(F) Molybdates of elements niobium and tantalum, and complex molybdates thereof and precursors thereof, and

10 (G) Molybdates of manganese and precursors thereof;

wherein said precursors comprise a molybdenum compound that is converted to a molybdate by heat treatment and compounds of the elements of said groups (A) to (G).

15 14. An electrical resistor paste which comprising bulk particles containing 34.8 to 95% by weight of one or more molybdates selected from the group consisting of (A) to (G) and their precursors, 0.3 to 29.9% by weight

20 of a fluoride of an alkaline earth metal, 0.3 to 33.3% by weight of a carbonate of an alkaline earth metal and 2.1 to 49.5% by weight of glass, and in which the surfaces of said bulk particles are reduced to form acicular particles by sintering at 800° to 1100° C. at least the non-combustible portion of the non-volatile matter thereof in a non-oxidizing atmosphere, thereby obtaining a sintered body in which said acicular particles are deposited onto said bulk particles,

(A) Molybdates of alkaline earth metals,

(B) Molybdates of zinc,

(C) Molybdates of elements Y, La, Ce, Pr, Nd, Sm, Eu, Gd, Tb, Dy, Ho, Er, Tm, Yb and Lu, and complex molybdates of two or more of said elements,

(D) Molybdates of aluminum

(E) Molybdates of elements zirconium and hafnium, and complex molybdates thereof,

(F) Molybdates of elements niobium and tantalum, and complex molybdates thereof, and

40 (G) Molybdates of manganese;

wherein said precursors comprise a molybdenum compound that is converted to a molybdate by heat treatment and compounds of the elements of said groups (A) to (G).

45 15. An electrical resistor paste as defined in claim 9, wherein said at least one molybdate selected from the group consisting of (A) to (G) and their precursors, comprises at least 2 molybdates.

16. An electrical resistor as defined in claim 1 or 10, 50 wherein said molybdate is selected from the group consisting of 30-96 weight % (A), 55-95 weight % (B), 50-96 weight % (C), 35-96 weight % (D), 40-96 weight % (E), 45-96 weight % (F), and 50-96 weight % (G).

17. An electrical resistor as defined in claim 4, 55 wherein said molybdate is selected from the group consisting of 30-95 weight % (A), 60-95 weight % (B), 55-95 weight % (C), 40-95 weight % (D), 40-95 weight % (E), 50-95 weight % (F), and 55-95 weight % (G).

18. An electrical paste as defined in claim 7 or 14, 60 wherein said molybdate is selected from the group consisting of 40-95 weight % (A), 65-95 weight % (B), 60-95 weight % (C), 45-95 weight % (D), 50-95 weight % (E), 55-95 weight % (F), and 65-95 weight % (G).

\* \* \* \* \*